# EUROPEAN PATENT SPECIFICATION

(11) **EP 0 337 490 B1**
(45) Date of publication and mention of the grant of the patent: **20.12.1995**
(21) Application number: 89106744.9
(22) Date of filing: 14.04.1989
(51) Int. Cl.: G03C 1/76, G03C 1/825, G03C 1/95

(54) **Silver halide light-sensitive photographic material**
Lichtempfindliches photographisches Silberhalogenidmaterial
Matériau photographique à l'halogénure d'argent sensible à la lumière

(30) Priority: 15.04.1988 JP 92804/88; 13.06.1988 JP 145492/88; 20.06.1988 JP 151791/88; 11.10.1988 JP 255425/88; 07.02.1989 JP 27894/89; 09.02.1989 JP 30405/89
(43) Date of publication of application: 18.10.1989
(73) Proprietor: Fuji Photo Film Co., Ltd., Kanagawa-ken (JP)
(72) Inventor: Shiba, Keisuke c/o Fuji Photo Film Co., Ltd., Minami Ashigara-shi Kanagawa (JP); Yamanouchi, Junichi c/o Fuji Photo Film Co., Ltd., Minami Ashigara-shi Kanagawa (JP); Hasebe, Kazunori c/o Fuji Photo Film Co., Ltd., Minami Ashigara-shi Kanagawa (JP); Taguchi, Seiichi c/o Fuji Photo Film Co., Ltd., Minami Ashigara-shi Kanagawa (JP); Shioda, Kazuo c/o Fuji Photo Film Co., Ltd., Minami Ashigara-shi Kanagawa (JP); Nishikawa, Toshihiro c/o Fuji Foto Film Co., Ltd., Minami Ashigara-shi Kanagawa (JP); Ohno, Shigeru c/o Fuji Foto Film Co., Ltd., Minami Ashigara-shi Kanagawa (JP); Fuchizawa, Tetsuro c/o Fuji Foto Film Co., Ltd., Fujinomiya-shi Shizuoka (JP)
(74) Representative: Grünecker, Kinkeldey, Stockmair & Schwanhäusser Anwaltssozietät

(56) References cited:
- EP-A- 0 154 920
- EP-A- 0 258 903
- DE-A- 1 909 463
- DE-A- 2 163 904
- FR-A- 2 338 513
- GB-A- 2 023 299
- GB-A- 2 078 235
- GB-A- 2 108 865
- US-A- 2 527 583
- US-A- 3 486 897
- PATENT ABSTRACTS OF JAPAN vol. 11, no. 32 (P-541)(2479) 30 January 1987, & JP-A- 61 201242
- PATENT ABSTRACTS OF JAPAN vol. 12, no. 284 (P-740)(3131) 4 August 1988, & JP-A- 63 63040
- PATENT ABSTRACTS OF JAPAN vol. 11, no. 35 (P-542)(2482) 3 February 1987, & JP-A-61 205934
- PATENT ABSTRACTS OF JAPAN vol. 11, no. 68 (P-553)(2515) 28 February 1987, & JP-A- 61 231550
- PATENT ABSTRACTS OF JAPAN vol. 11, no. 170 (P-581)(2617) 2 June 1987, & JP-A- 62 2270

## Description

The present invention relates to a silver halide light-sensitive color photographic material having a reflective support, which exhibits excellent sharpness and edge contrast in images and excellent whiteness in non-image areas. In particular, the present invention relates to a color photographic paper especially suitable for rapid development processing.

The present invention also relates to a method of forming a color image to form excellent line images or character images along with photographic or CG (computer graphic) images.

With the recent popularization of silver halide photographic materials, the demand for silver halide photographic materials which can be rapidly and simply processed to produce a product of excellent quality, as compared with other image-forming systems, is increasing. Picture-taking photographic materials have heretofore been improved for gradation reproducibility, image graininess and image sharpness. Various means may be used to attain the improved material including, for example, use of silver halide emulsions of high sensitivity comprising fine grains, formation of plural light-sensitive layers, formation of thin light-sensitive layers, economization of the amount of silver halides to be used, use of less light-scattering silver halide emulsions, incorporation of anti-halation or anti-irradiation dyes and use of mordant layers for anti-halation or anti-irradiation dyes. For color photographic materials, DIR couplers or color mixing preventing agents may be used to improve the sharpness by interimage effect. Picture-taking photographic materials have, in many cases, a transparent plate or film support. The support itself may be dyed for anti-halation, or an anti-halation black backing layer (AHB) or an anti-halation layer (AHU) may be provided therefor.

Various dyes used in color printing photographic materials for the purpose of color reproduction, tone reproduction, rapid processing and anti-irradiation have been improved. For instance, the improvement of these dyes is referred to in JP-A-50-145125, JP-A-52-20830, JP-A-50-147712, JP-A-59-111641, JP-A-61-148448, JP-A-61-161538, JP-A-61-151649, JP-A-61-151650, JP A-61-151651, JP-A-61-170742, JP-A-61-175638, JP-A-61-235837, JP-A-61-248044, JP-A-62-164043, JP-A-62-253145, JP-A-62-253146, JP-A-62-253142, JP-A-62-275262 and JP-A-62-283336 and Research Disclosure RD-17643 (December 1978, page 22) and RD-18716 (November 1979, page 647), (the term "JP-A" as used herein means an "unexamined published Japanese patent application"). Methods of providing AHU in color photographic materials are also known. These methods are described in, for example, US-A-2,882,156, US-A-2,326,057, US-A-2,839,401 and US-A-3,706,563 and JP-A-55-33172, JP-A-59-193447 and JP-A-62-32448.

Also, methods of using water-insoluble dyes as dispersions of the fine crystals thereof are disclosed in JP-A-55-155350, 55-155351, 56-12639, and 63-197943, and EP-B-15,601.

Furthermore, methods of using dyes adsorbed on fine metal salt grains are disclosed in US-A-2,719,088, US-A-2,496,841, and US-A-2,496,843, and JP-A-60-45237. JP-A-61231550 discloses an image forming method wherein the gamma value of the silver halide photographic sensitive material after development is regulated to 0.8 to 1.7 by mixing silver halide emulsions having higher and lower sensitivities and applying them to a support. This method permits a higher quality image to be obtained with reduced unevenness in image density.

Color printing photographic materials naturally utilize baryta paper as the support. Recently, however, a waterproof support formed by coating polyethylene on the both surfaces of a raw paper is often used in place of the baryta paper for the purpose of rapid processing. In order to improve the whiteness of the polyethylene-laminated paper support to achieve that of the baryta paper, titanium oxide grains or titanium oxide grains which have been surface-treated with aluminium oxide or silicon oxide may be incorporated into the polyethylene layer. However, the image sharpness of the titanium oxide-containing polyethylene-laminated paper support is still inferior to that of baryta paper. The improvement of titanium oxide-containing polyethylene layers is described in, for example, JP-B-58-43734 and JP-A-58-17433, JP-A-58-14830 and JP-A-61-259246 (the term "JP-B" as used herein means an "examined Japanese patent publication").

A method of forming a waterproof resin layer on a raw paper by coating a composition containing an unsaturated organic compound having one or more double bonds in one molecule and polymerizable by electron rays and a white pigment on a raw paper and hardening the composition on the paper by irradiation of electron rays thereto under heat is described in, for example, JP-A-57-27257, JP-A-57-49946, JP-A-61-262738 and JP-A-62-61049.

Silver halide photographic materials having a mirror-reflective or secondary diffusive reflective support are also known. For example, they are described in JP-A-63-24251, JP-A-63-24253 and JP-A-63-24255.

JP-A-63-63036 mentions the provision of a colloidal silver-containing antihalation layer in a direct positive color photographic paper or in a high-sensitivity reflective color photographic paper having a thinner reflective support than a conventional one so as to inhibit the deterioration of the sharpness due to the transmission density of the support being less than 0.8. JP-A-63-63040 mentions the provision of an auxiliary layer in a direct positive photographic material or in a negative photographic material containing a silver chloride-containing emulsion layer and a colloidal silver layer so as to prevent the occurrance of contact fog caused by the colloidal silver in rapid processing.

A particular technical means is required to attain improvement, which can be apparently recognized, with respect to the image sharpness and the tone reproducibility of the highlight details in the silver halide photographic material having the reflective support, especially in the color photographic paper having a primary diffusive reflective white support, without lowering the whiteness thereof.

The use of conventional anti-irradiation dyes or colloidal silver for anti-irradiation causes various problems including, fogging, an increase in the occurrence of staining, the remains of unnecessary colors and lowering of sensitivity. Additionally, it is limitative for improvement of sharpness.

In general, a photographic original of, for example, a color negative film or color positive slide obtained by photographing using a picture-taking photographic material is printed on a color photographic paper by imagewise exposure to obtain a color print. Recently, the demand for photographs having both a photographic image and a character image in combination is greatly increasing. In order to combine characters of excellent image quality and a picture in one photographic print, in general, a method of printing a film block copy, which has separately been prepared by printing the necessary characters on a lith film, and printing them in combination is employed. However, such a method is complicated and requires a long time to be completed.

In place of a film block copy, a printed sheet formed by printing characters on a semi-transparent raw paper with a word processor may by used, but the color print obtainable therewith has a poor image quality. The method of printing CG, line images or character images on a color photographic paper from a memory means previously inputted as a digital information with a printer having a CRT exposure system, is also known. For instance, printers having a CRT exposure system are disclosed in JP-A-62-43281, JP-A-62-184446, JP-A-62-295037, JP-A-62-295038 and JP-A-62-295039. JP-A-62-89965 discloses a printer having an FOT (fiber optics tube).

The image quality of the photographic picture image obtained by conventional exposure printing systems is extremely high. However, the image quality of the line image or character image to be combined with the picture image is not as good as that of the picture image.

On the other hand, prints obtained from color photographic papers are widely used for various kinds of cards including an ID card, license card, credit card, bank card, etc. Methods for preparing the cards are described, for example, in JP-A-62-50755, JP-A-62-58247, JP-A-62-58248 and JP-A-62-58249. Prints obtained from thin color photographic papers are also used for seal prints or post cards which are directly stuck to other supports. These are described in, for example, JP-A-60-41949 and JP-A-60-41950.

A method of directly photographing and recording a photographic image as displayed on a CRT with an instant photographic material has already been put to practical use, for example, as VIDEOFIX-85 (trade name). This method is also described in, for example, JP-A-60-176385.

Scanning exposure systems are advantageous in that characters, figures and photographic images (continuous tone images) are easily digitalized for direct image synthesis or image processing or they are outputted with ease. However, on the contrary, such systems are disadvantageous in that the image quality of the line images or character images formed is much poorer than the image quality of the photographic images formed.

If a silver halide emulsion having a high silver chloride content (for example, 80 mol% or more of the total silver halide) is used in at least one layer of a color photographic material so as to accelerate and simplify the color development procedure of the material, the sensitivity is hardly elevated and the sensitivity as well as the stability of latent images formed is rather inferior to that of a material having a conventional silver chlorobromide emulsion (for example, silver halide emulsion having a silver chloride content of less than 20 mol%). If a large amount of dyes is used for the purpose of anti-irradiation or anti-halation, the effective sensitivity would be further lowered, and especially, the spectral sensitivity would often be lower because of the anti-color sensitizing action or because of desorption of the sensitizing dyes used. Silver chloride-rich silver halide emulsios have almost no light absorption in the visible range (400 to 700 nm) and the sensitivity is essentially obtained from spectral sensitization, thus the problem of lowering the spectral sensitivity is a big problem.

Scanning exposure systems use laser rays having light intensity in at least three different wavelength ranges, fluorescent emission, LED (luminescence emitting diode) emission or liquid crystal emission and, if desired, it is combined with color separation filters. Especially in a scanning exposure system with fluorescent emission, for example, a CRT or FOT exposure system, selection of proper fluorescent bodies with pertinent light emission intensity and efficiency for the spectral sensitivity of the respective light-sensitive layers of color photographic papers to be exposed therewith is necessary so as to accelerate, simplify and stabilize the exposure step. In general, stable tungsten light, halogen lamp light or xenon lamp light is used in the photographic exposure system, and the sensitivity of the respective light-sensitive layers of color photographic papers to be exposed therewith is determined in accordance with the light source. However, the ratio of the sensitivity of the respective light-sensitive layers of conventional color photographic papers does not match with CRT or FOT exposure systems at all. In most color photographic papers, the sensitivity to light with a longer wavelength, especially red-sensitivity is relatively insufficient.

It is the object of the present invention to overcome said problems in the prior art and to provide a white reflective support-having photographic material which has improved whiteness in the non-image part and excellent image sharpness, which has excellent tone reproducibility in the highlight details, which is suited for rapid development (for a color development time of 90 s or less) and which has been improved so that the processing solution does not penetrate into the paper from the cut edge thereof to stain the finished photograph. Further, the present invention wants to provide a method of forming color images simply, rapidly and at a low production cost, for obtaining prints composed of line images and/or character images having excellent image quality, especially having high edge contrast, and CG images and/or photographic images.

According to the present invention this object is attained with a color photographic material comprising: at least one silver halide light-sensitive layer provided on a reflective support containing white pigment grains in a waterproof resin layer, wherein said pigment grains are present in said waterproof resin layer in a density of from 10% by weight or more, and a colored layer which can be decolored by photographic processing located between said support and said silver halide light-sensitive layer, characterized in that the degree of dispersion of the white pigment grains in the layer is from 0.20 or less as the fluctuation coefficient (s/R̅) of the possessory area ratio (%) per unit area of 6 »m x 6 »m, where R̅ means the mean possessory area ratio per unit area and s means the standard deviation of the possessory area ratio per the unit area.

According to the present invention there is also provided a method of forming a color image characterized in that the color photographic material of the present invention is printed by a scanning exposure system and then subjected to color development processing.

In a particularly preferred embodiment of the present invention the color photographic material is a reflection color photographic material, the at least one silver halide light-sensitive layer contains a colour coupler, the waterproof resin layer is located on the side of the support coated with said silver halide light-sensitive layer, and said silver halide light-sensitive layer contains an emulsion of silver chlorobromide having a mean silver chloride content of 90 mol% or more and having a silver bromide-localized phase in the inside and/or surface of the emulsion grain.

Further preferred embodiments are set forth in the dependent claims.

Fig. 1 shows a flow sheet of one embodiment of a process of forming prints by a CRT exposure system.

Fig. 2 shows the scanning exposure direction for a Japanese character and the position for determination of the density of the parts of the character.

Fig. 3 is a spectral graph showing the relationship between the visual density and the position of the scanning direction in determination of the density of the Japanese character by means of a scanning exposure system with a microdensitometer. The axis of the ordinate indicates the visual density of fine lines constituting the character and that of the abscissa indicates the position of the scanning direction.

Fig. 4-a and Fig. 4-b show spectral sensitivity curves of samples (F) and (E) of Examples B-5 and B-6, respectively, where B (... ... ...), G (------) and R (_____) mean the relative spectral sensitivity of blue-sensitive layer, green-sensitive layer and red-sensitive layer, respectively. The value for R is a 12-magnified one. The axis of the ordinate indicates the relative spectral sensitivity, and that of the abscissa indicates the wavelength (nm).

Fig. 5 shows relative emission strength distribution of the mixture of fluorescent substances of P-22R and P-45. The axis of the ordinate indicates the relative emission strength, and that of the abscissa indicates the wavelength (nm).

Fig. 6 shows spectral transmittance curves of B, G, R and Y filters. The axis of the ordinate indicates the transmittance, and that of the abscissa indicates the wavelength (nm).

Fig. 7 is a graph to explain the evaluation method of edge sharpness, where the axis of the ordinate indicates the density and that of the abscissa indicates the distance. Ds means the density difference, and L means the transition width of the stepwise image with Ds.

The present invention will be explained in detail hereunder.

The white support for use in the silver halide photographic material of the present invention can be prepared by coating a waterproof resin layer on the substrate. Suitable substrates include raw papers made from natural pulp or synthetic pulp or a mixture thereof as well as plastic films such as polyester films of polyethylene terephthalate or polybutylene terephthalate or cellulose triacetate film, polystyrene film, polypropylene film or other polyolefin films.

The raw paper for use in the present invention is made from materials which are generally used for photographic papers. Specifically, natural pulp derived from soft wood or hard wood is used as a main raw material for the paper, which may optionally contain filler such as fine grains of clay, talc, calcium carbonate or urea resin, a sizing agent such as resin, alkylketene dimer, higher fatty acid, paraffin wax or alkenylsuccinic acid, a paper reinforcing agent such as polyacrylamide and a fixing agent such as papermaker's alum earth or cationic polymer. In particular, a natural paper containing a reactive sizing agent such as alkylketene dimer or alkenylsuccinic acid and having a pH of from 5 to 7 (determined by conventional manner, that is, water is dropped on the paper, placing a plane electrode, for example, a pH-meter having a plane-electrode type GST-5313F manufactured by Toa Electrowave Industries (Japan), and the pH at the portion where water is dropped is measured after pH becomes constant) is preferred. The natural pulp may be substituted by synthetic pulp, or a mixture comprising natural pulp and synthetic pulp in a proper ratio can also be used.

The surface of the pulp may be sized with a film-forming polymer such as gelatin, starch, carboxymethyl cellulose, polyacrylamide, polyvinyl alcohol or modified polyvinyl alcohol. The modified polyvinyl alcohol includes carboxyl-modified or a silanol-modified one or a copolymer with acrylamide. For surface-sizing with such a film-forming polymer, the amount of the polymer to be coated may be from 0.1 to 5.0 g/m², preferably from 0.5 to 2.0 g/m². The film-forming polymer may contain, if desired, an antistatic agent, a fluorescent brightening agent, pigment and a defoaming agent.

The raw paper for use in the present invention can be prepared by processing a pulp slurry comprising the pulp mentioned above and, if desired, other additives such as a filler, a sizing agent, a paper reinforcing agent and a fixing agent, with a papermaking machine such as Fourdrinier machine, followed by drying and rolling the paper strip thus formed. Either before or after the drying step, the paper strip is sized on the surface thereof, and it is subjected to calender treatment between the drying step and the rolling step. When the surface-sizing treatment is carried out after drying, the calender treatment may be effected either before or after the surface-sizing treatment.

The determination of whether the raw paper to be used as the substrate of the support for the photographic materials of the present invention is a neutral paper or not can be performed by measuring the pH value thereof using a plane-electrode type GST-5313F (manufactured by Toa Electrowave Industries, Japan) as an electrode. In the determination, a neutral paper preferably has a pH of 5 or more, and preferably up to 9, and more preferably up to 7.

The waterproof resin layer may also be provided in the preferred reflection color photographic material according to the invention.

The waterproof resin layer, such as a vinyl chloride resin, may constitute the support by itself.

The waterproof resin for use in the present invention is one preferably having a water absorption (% by weight) of 0.5 or less, more preferably 0.1 or less, including, for example, polyalkylenes (e.g., a polymer of ethylene, or propylene or copolymer thereof), vinyl polymers or copolymers of vinyl compounds (e.g., a polymer of styrene and acrylate or copolymer thereof) and polyesters and copolyesters. Preferred are polyalkylene resins, and low density polyethylene, high density polyethylene, polypropylene and blends thereof are especially used among them. If desired, the resins may contain additives including fluorescent brightening agents, antioxidants, antistatic agents and releasing agents. The thickness of the resin layer may be from 5 to 200 »m, especially from 10 to 40 »m. The formation of the resin layer, in general, is carried out by kneading a white pigment together with the resin by a melt blending method and extruding through a melt extruder to laminate the blend on a support substrate.

Unsaturated organic compounds having one or more polymerizable carbon-carbon double bonds on one molecule (e.g., methacrylate compounds) as described in JP-A-57-27257, JP-A-57-49946 and JP-A-61-262738, and di-, tri- or tetra-acrylates as represented by the general formula described in JP-A-61-262738 can also be used. In this case, the polymer may be coated on a support substrate and then hardened by irradiation with electron rays to form a waterproof resin layer thereon. A white pigment and other additives may be dispersed in the unsaturated organic compound. Any other resins may also be dispersed into the compound.

For formation of the waterproof resin layer on the support substrate for use in the present invention, various lamination methods as described in, for example, New Handbook for Lamination Coating (edited by Kako Kijutsu Kenkyu-kai, Japan) may be used. For instance, the dry lamination method, and the non-solvent dry lamination method can be used. For coating the resin blend on the surface of the substrate, any means selected from the gravure roll coating method, the wire bar coating method, the doctor blade coating method, the reverse roll coating method, the dip coating method, the air knife coating method, the callendar coating method, the kiss coating method, the squeeze coating method and the Fountain type coating method can be employed.

In accordance with the present invention, the waterproof resin contains a white pigment. For instance, suitable white pigments include rutile-type titanium oxide, anatase-type titanium oxide, barium sulfate, calcium sulfate, silicon oxide, zinc oxide, titanium phosphate and aluminium oxide. The surface of the fine grains of the titanium oxide pigment is preferably surface-treated with an inorganic oxide such as silica or aluminium oxide and a dihydric or tetrahydric alcohol such as 2,4-dihydroxy-2-methylpentane or trimethylolethane as described in JP-A-58-17151, separately or in combination. Generally, the fine grains have a mean grain size of from 0.05 to 0.4 »m, and preferably from 0.1 to 0.3 »m.

The surface of the support is preferably treated by corona discharge, glow discharge or flame treatment and a protective layer group for silver halide photographic materials is provided on the thus surface-treated support.

The total thickness of the support is preferably from 30 to 350 g/m² (from about 30 to 400 »m), more preferably from 50 to 200 g/m². Of the total thickness, the waterproof resin layer is preferably from 5 to 200 »m, more preferably from 10 to 40 »m.

One characteristic feature of the support for use in the present invention is that it contains fine grains of a white pigment (especially preferably titanium oxide) in a density of 10% by weight or more, preferably 12% by weight or more, more preferably from 15% by weight to 60% by weight, as dispersed in the waterproof resin layer. In particular, the fine grains of white pigment are preferably dispersed densely and uniformly (that is, in order that there is no part sparsely containing the fine grains) in the surface of the waterproof resin layer or in a thickness of e.g 10 »m from the surface of the layer.

To evaluate the dispersion of the fine white pigment grains in the resin layer, the surface of the resin layer or the thickness of the layer from the surface to about 0.1 »m, preferably about 50 nm (500 Å) is subjected to glow discharge for ion-sputtering so as to sputter the surface resin, and the fine grains thus exposed are observed with an electronic microscope. The photographed possessory area of the fine grains on the surface of the thus treated resin layer is obtained from the electromicroscopic photograph and the fluctuation coefficient of the possessory area ratio (%) is calculated for evaluation of the intended dispersibility. The ion-sputtering method employable for this purpose is described in detail in Y. Murayama and K. Kashiwagi, Technique for Surface Treatment with Plasma (Kikai-no Kenkyu), Vol. 33, No. 6 (1981).

In order to control the fluctuation coefficient of the fine white pigment grains to be 0.20 or less, in accordance with the present invention, it is preferred that the white pigment is fully kneaded with the resin component in the presence of a surfactant. It is also preferred that the surface of the pigment grains be pre-treated with the above-mentioned di- to tetra-hydric alcohol.

The possessory area ratio (%) of the fine white pigment grains per a determined unit area is obtained by dividing the observed area into the adjacent unit areas having a size of 6 »m x 6 »m and determining the possessory area ratio (%) (Ri) of the fine grains as projected in the unit area. The fluctuation coefficient of the possessory area ratio (%) is obtained as the ratio of (s/R̅) of the standard deviation (s) of (Ri) to the mean value (R̅) of (Ri). The number (n) of the unit areas as intended for the purpose is preferably 6 or more. Accordingly, the fluctuation coefficient (s/R̅) can be obtained from the following formula:

In accordance with the present invention, the fluctuation coefficient of the possessory area ratio(%) of the fine pigment grains is 0.20 or less, preferably 0.15 or less, and more preferably 0.08 or less. When the fluctuation coefficient is 0.08 or less, the dispersion of the grains is substantially "uniform".

It is particularly preferred that in the preferred reflection color photographic material the pigment density is 12% by weight or more and S/R̅ is 0.15 or less.

In general, when the above-mentioned white pigment is incorporated into the support of a silver halide photographic material, the photograph formed on the material would visually have a whitened background and have a worsened sharpness of the image formed. As opposed to this, when the density of the white pigment and the degree of the dispersion thereof satisfy the conditions as defined in accordance with the present invention, the strength of the primary diffusive reflected light (see Hand Book of Science of Color (new edit.), edited by Japan Color Society: published by Tokyo Univ. Publication Association; Sept. 1985, Chap. 18) to the incident light may be elevated and the extension of the diffusive light can be reduced. The improved effect of the present support is displayed not only for the incident light for exposure of the photographic material but also for the incident light for visually seeing the photograph, which is one characteristic advantage attainable by the present invention.

The colored layer used in the present invention can be decolored after photographic processing, e.g., development, bleach-fixation, rinsing or stabilization, and is provided between the support and the silver halide photographic light-sensitive layer.

Fixation of a light absorbent (a dye and/or colloidal silver) in the colored layer may effectively impart an anti-halation effect to the silver halide light-sensitive layer without a reduction of the spectral sensitivity nor an increase of fog. Suitable light absorbents included colloidal silver (black to yellow) and/or dyes. Colloidal silver and a dye are preferably used in amounts such that the colloidal silver provides reflect density of from 0.1 to 1.5, and the dye provides transmission density of from 0.1 to 1.2. Provision of the colored layer is effective for more satisfactorily inhibiting the deterioration of the sharpness of the image which would be caused by the extension of the diffused light from the support.

As the colored layer used in the present invention, a colloidal silver emulsion is preferably used as the light absorbent. Any and every colloidal silver emulsion which is generally used for picture-taking color photographic materials can be used for this purpose. Black or yellow colloidal silver can be used.

The colloidal silver can be prepared in accordance with the methods described in, for example, US-A-2,688,601 and US-A-3,459,563 and BE-B-622,695. The colloidal silver for use in the present invention is preferably fully desalted to have an electroconductivity of not higher than 1800 »scm⁻¹, after preparation. The content of the colloidal silver in the colloidal silver-containing layer is from 0.01 to 0.5 g/m², and preferably from 0.05 to 0.2 g/m², as silver.

Dyes may also be incorporated into the colored layer, together with the colloidal silver, to inhibit irradiation, stabilize the sensitivity, improve the safelight stability and improve the spectral sensitivity distribution.

Another preferred embodiment of the present invention, is that the colored layer may contain a dye and a cationic polymer for mordanting the same, in combination. The polymer preferably has a molecular weight of at least 5,000.

The cationic polymer which is preferably used in the present invention is a non-coloring polymer having at least one hydrogen-containing ammonium base in the cation site which functions as an anion exchange polymer.

Typically, cationic polymers represented by the following general formula (I) are preferred for use in the present invention.

In the formula (I), A represents a monomer unit derived from a copolymerizable monomer having at least two copolymerizable ethylenic unsaturated groups, one of which is in the side chain of the monomer. B represents a monomer unit derived from a copolymerizable ethylenic unsaturated monomer. R₁ represents a hydrogen atom, a lower alkyl group or an aralkyl group. Q represents a single bond or an alkylene group, an arylene group, an aralkylene group,
or
L represents an alkylene group, an arylene group or an aralkylene group. R represents an alkyl group. G represents
R₂, R₃, R₄, R₅, R₆, R₇, R₈ and R₉ each represents a hydrogen atom, an alkyl group, an aryl group or an aralkyl group. These may be same as or different from each other. The above-mentioned groups may optionally be substituted. X^{⊖} represents an anion.

Any two or more of Q, R₂, R₃, and R₄ or Q, R₅, R₆, R₇, R₈ and R₉ may be bonded to each other to form a ring structure together with the adjacent nitrogen atom.

In the group of formula
at least one of R₂, R₃, and R₄ must be a hydrogen atom.

x, y and z each represent a molar percentage, and x is from 0 to 60, y is from 0 to 60 and z is from 30 to 100.

The compounds of the formula (I) will be explained in more detail hereunder.

Examples of the monomers A include divinylbenzene, ethylene glycol dimethacrylate, diethylene glycol dimethacrylate, triethylene glycol dimethacrylate, ethylene glycol diacrylate, diethylene glycol diacrylate, 1,6-hexanediol diacrylate, neopentylglycol dimethacrylate and tetramethylene dimethacrylate. Among the foregoing, divinylbenzene and ethylene glycol dimethacrylate are especially preferred.

Examples of the ethylenic unsaturated monomers represented by B include ethylene, propylene, 1-butene, isobutene, styrene, α-methylstyrene, vinylketone, monoethylenic unsaturated esters of aliphatic acids (e.g., vinyl acetate, allyl acetate), ethylenic unsaturated monocarboxylic acid or dicarboxylic acid esters (e.g., methyl methacrylate, ethyl methacrylate, n-butyl methacrylate, n-hexyl methacrylate, cyclohexyl methacrylate, benzyl methacrylate, n-butyl acrylate, n-hexyl acrylate, 2-ethylhexyl acrylate), monoethylenic unsaturated compounds (e.g., acrylonitrile) and dienes (e.g., butadiene, isoprene). Among them, styrene, n-butyl methacrylate and cyclohexyl methacrylate are especially preferred. B may contain two or more of the monomer units.

R₁ is preferably a hydrogen atom or a lower alkyl group having from 1 to 6 carbon atoms (e.g., methyl, ethyl, n-propyl, n-butyl, n-amyl, n-hexyl) or an aralkyl group (e.g., benzyl). In particular, R₁ is especially preferably a hydrogen atom or a methyl group.

Q is preferably an optionally substituted divalent alkylene group having from 1 to 12 carbon atoms (e.g., methylene or -(CH₂)₆-), an optionally substituted phenylene or an optionally substituted aralkylene having from 7 to 12 carbon atoms (e.g.,
or
In addition, the following groups are also preferred for Q.

In the formulae, L represents an optionally substituted alkylene group having from 1 to 6 carbon atoms, or an optionally substituted arylene group, or an optionally substituted aralkylene group having from 7 to 12 carbon atoms. Especially preferably, it is an optionally substituted alkylene group having from 1 to 6 carbon atoms. R represents an alkyl group having from 1 to 6 carbon atoms.

G represents
or

In the formulae, R₂, R₃, R₄, R₅, R₆, R₇, R₈ and R₉ are the same or different and each is preferably a hydrogen atom, an alkyl group having from 1 to 20 carbon atoms, an aryl group having from 6 to 20 carbon atoms, or an aralkyl group having from 7 to 20 carbon atoms. The alkyl group, aryl group and aralkyl group include a substituted alkyl group, a substituted aryl group and a substituted aralkyl group, respectively.

The unsubstituted alkyl group preferably has from 1 to 12 carbon atoms, more preferably from 4 to 10 carbon atoms, and it includes, for example, methyl, ethyl, n-propyl, isopropyl, n-butyl, isobutyl, t-butyl, n-amyl, isoamyl, n-hexyl cyclohexyl, n-heptyl, n-octyl, 2-ethylhexyl, n-nonyl, n-decyl and n-dodecyl groups. Example of the substituted alkyl group include an alkoxyalkyl group (e.g., methoxymethyl, methoxyethyl, methoxybutyl, ethoxyethyl, ethoxypropyl, methoxybutyl, butoxyethyl, butoxypropyl, butoxybutyl, vinyloxyethyl), a cyanoalkyl group (e.g., 2-cyanoethyl, 3-cyanopropyl, 4-cyanobutyl), a halogenated alkyl group (e.g., 2-fluoroethyl, 2-chloroethyl, 3-fluoropropyl), an alkoxycarbonylalkyl group (e.g., ethoxycarbonylmethyl), and an allyl group, a 2-butenyl group and a propargyl group.

The aryl group includes an unsubstituted aryl group (e.g., phenyl, naphthyl) and a substituted aryl group, for example, an alkylaryl group (e.g., 2-methylphenyl, 3-methylphenyl, 4-methylphenyl, 4-ethylphenyl, 4-isopropylphenyl, 4-tert-butylphenyl), an alkoxyaryl group (e.g., 4-methoxyphenyl, 3-methoxyphenyl, 4-ethoxyphenyl), and an aryloxyaryl group (e.g., 4-phenoxyphenyl). The aryl group preferably has from 6 to 14 carbon atoms, more preferably from 6 to 10 carbon atoms. It is especially preferably a phenyl group.

The aralkyl group includes an unsubstituted aralkyl group (e.g., benzyl, phenethyl, diphenylmethyl, naphthylmethyl) and a substituted aralkyl group, for example, an alkylaralkyl group (e.g., 4-methylbenzyl, 2,5-dimethylbenzyl, 4-isopropylbenzyl), an alkoxyaralkyl group (e.g., 4-methoxybenzyl, 4-ethoxybenzyl), a cyanoaralkyl group (e.g., 4-cyanobenzyl), a perfluoroalkoxyaralkyl group (e.g., 4-pentafluoropropoxybenzyl, 4-undecafluorohexyloxybenzyl) and a halogenated aralkyl group (e.g., 4-chlorobenzyl, 4-bromobenzyl, 3-chlorobenzyl). The aralkyl group preferably has from 7 to 15 carbon atoms, more preferably from 7 to 11 carbon atoms. Among them, a benzyl group or a phenethyl group is especially preferable.

X^{⊖} represents an anion, for example, a halide ion (e.g., chloride or bromide ion), an alkyl- or arylsulfonate ion (e.g., methanesulfonate, ethanesulfonate, benzenesulfonate, p-toluenesulfonate), an acetate ion, a sulfate ion or a nitrate ion. Especially, chloride ion, acetate ion and sulfate ion are preferred.

Any two or more of Q, R₂, R₃, and R₄, may be bonded together to form a cyclic structure together with the adjacent nitrogen atom. Preferable examples of the cyclic structure include pyrrolidine ring, piperidine ring, morpholine ring, pyridine ring, imidazole ring and quinuclidine ring. Especially preferred are pyrrolidine ring, morpholine ring, piperidine ring, imidazole ring and pyridine ring.

Any two or more of Q, R₅, R₆, R₇, R₈ and R₉ may be bonded together to form a cyclic structure together with the adjacent nitrogen atom, and the cyclic structure is especially preferably a 6 membered or 5-membered ring.

x indicates from 0 to 60 mol%, preferably from 0 to 40 mol%, more preferably from 0 to 30 mol%. y indicates from 0 to 60 mol%, preferably 0 to 40 mol%, more preferably from 0 to 30 mol%. z indicates from 30 to 100 mol%, preferably from 40 to 95 mol%, more preferably from 50 to 85 mol%.

In formula (I), G is preferably a basic residue having a pKa value of 4.5 or more, especially 7 or more, in an aqueous solution.

As the cationic polymer of the formula (I), a polymer latex is especially preferred from the view point of the film-forming quality thereof.

Specific examples of the compounds of the formula (I) and cationic polymers which are preferably used in the present invention are mentioned below.

In the formation of a dispersion of fine grains of the cationic polymer, a crosslinking monomer such as divinylbenzene is generally used as a monomer component. However, such a crosslinking monomer is not indispensable, depending upon the kind of the monomer to be used.

Of the compounds of the formula (I) for use in the present invention, those in which G represents
may be prepared by the method mentioned below.

The polymers of the formula (I) for use in the present invention are generally prepared by copolymerizing the above-mentioned copolymerizable monomer having at least two ethylenic unsaturated groups and ethylenic unsaturated monomer together with an unsaturated monomer of a formula:
in which R₁, R₂, R₃ and Q have the same meanings as defined above, for example, N,N-dimethylaminoethyl methacrylate, N,N-diethylaminoethyl methacrylate, N,N-dimethylaminoethyl acrylate, N,N-diethylaminoethyl acrylate, N-(N,N-dimethylaminopropyl)acrylamide, N-(N,N-dihexylaminomethyl)acrylamide, 3-(4-pyridyl)propyl acrylate, N,N-dimethylaminomethylstyrene, N,N-diethylaminomethyl styrene, N,N-dihexylaminomethylstyrene, 2-vinylpyridine or 4-vinylpyridine, especially preferably N,N-diethylaminoethyl methacrylate, N,N-dimethylaminomethylstyrene or N,N-diethylaminomethylstyrene, followed by reacting the resulting copolymer with a compound having a structure of R₄-X (where R₄ and X have the same meanings as defined above, for example, hydrochloric acid, sulfuric acid, nitric acid, acetic acid, p-toluenesulfonic acid) to give the corresponding ammonium salt.

The polymers of formula (I) for use in the present invention may also be prepared by copolymerizing the above-mentioned copolymerizable monomer having at least two ethylenic unsaturated groups and ethylenic unsaturated monomer together with an unsaturated monomer of a formula:
in which R₁, R₂, R₃, R₄, X and Q have the same meanings as defined above, for example, N,N dimethylaminoethyl methacrylate hydrochloride, N,N-diethyl aminoethyl methacrylate sulfate, N,N-dimethylaminoethyl acrylate hydrochloride, N,N-diethylaminoethyl acrylate acetate, N,N-dimethylaminostyrene hydrochloride, N,N-diethylaminomethylstyrene sulfate, 2-vinylpyridine hydrochloride or 4-vinylpyridine hydrochloride.

The polymers of formula (I) for use in the present invention may further be prepared by copolymerizing the above-mentioned copolymerizable monomer having at least two ethylenic unsaturated groups and an ethylenic unsaturated monomer together with an unsaturated monomer of the formula:
in which X represents a halogen atom (e.g., chlorine, bromine) or a sulfonic acid ester group (e.g., p-toluenesulfonyloxy) and R₁ and Q have the same meanings as defined above, for example, β-chloroethyl methacrylate, β-p-toluenesulfonyloxyethyl methacrylate or chloromethylstyrene, followed by reacting the resulting copolymer with an amine having a structure of
(where R₂, R₃ and R₄ have the same meanings as defined above), for example, dimethylamine, diethylamine, di-n-propylamine, di-n-butylamine, morpholine or piperidine, to give the corresponding ammonium salt.

Of the compounds of the formula (I) for use in the present invention, those where G represents
can be prepared by the method mentioned below.

Specifically, the polymers of the formula (I) for use in the present invention can be prepared by copolymerizing the above-mentioned copolymerizable monomer having at least two ethylenic unsaturated groups and ethylenic unsaturated monomer together with an unsaturated monomer of a formula:
in which R₁, R₅ and Q have the same meanings as defined above, for example, methyl vinyl ketone, methyl (1-methylvinyl) ketone, ethyl vinyl ketone, ethyl (1-methylvinyl) ketone, n-propyl vinyl ketone, diacetone acrylamide or diacetone acrylate, especially preferably methyl vinyl ketone, ethyl vinyl ketone, diacetone acrylamide or diacetone acrylate, followed by reacting the resulting copolymer with a compound of a formula:
in which R₆, R₇, R₈ and R₉ have the same meanings as defined above, for example, aminoguanidine bicarbonate, or N-amino-N′-methylguanidine bicarbonate, especially preferably aminoguanidine bicarbonate, and further with a compound H-X (where H-X has the same meaning as defined above, for example, hydrogen chloride, hydrogen bromide, sulfuric acid, acetic acid, nitric acid), to give the corresponding guanidium salt.

The above-mentioned polymerization reaction can be carried out by any conventional method of solution polymerization, emulsion polymerization, suspension polymerization, precipitation polymerization or dispersion polymerization. Solution polymerization and emulsion polymerization are preferred.

Of the above-mentioned polymerization reaction methods, for example, the emulsion polymerization can be carried out generally in the presence of at least one emulsifying agent selected from anionic surfactants (e.g., sodium dodecylsulfate, or Triton 770, a commercial product from Rhom & Haas), cationic surfactants (e.g., octadecyltrimethyl ammonium chloride), non-ionic surfactants (e.g., EMALEX NP-20, a commercial product from Nippon Emulsion), gelatin and polyvinyl alcohol, together with a radical polymerization initiator (e.g., combination of potassium persulfate and sodium hydrogen sulfite, a commercial product from Wako Pure Chemicals in the trade name of V-50), at a temperature of generally from about 30°C to about 100°C, preferably from about 40°C to about 80°C.

The above-mentioned reaction of forming the corresponding ammonium salt from the copolymer is carried out at a temperature of generally from about -10°C to about 40°C, especially preferably from about 0°C to about 30°C.

The copolymers for use in the present invention can be prepared in one reactor vessel throughout the complete manufacture process with ease.

Examples of production of some typical copolymers for use in the present invention are discussed below.

### PRODUCTION EXAMPLE 1

### Production of Poly(divinylbenzene-co-diethylaminomethylstyrene Sulfate) Polymer Dispersion (2):

1100 g of distilled water were put in a reactor vessel, which was then degassed using nitrogen gas. 16.6 g of sodium dodecylsulfate, 1.9 g of sodium hydroxide, 1.4 g of sodium sulfite, 33.6 g of divinyl benzene and 195.7 g of diethylaminomethylstyrene were added to the vessel and stirred.

After heating the vessel to 60°C, a solution of 0.9 g of potassium persulfate dissolved in 60 g of distilled water was added to the vessel every 1 h four times in all, and the whole was then continuously stirred for 2 h. Afterwards, it was cooled to room temperature, and a solution of 48.9 g of concentrated sulfuric acid dissolved in 313 g of distilled water was added thereto. The resulting mixture was filtered to obtain a polymer dispersion having a solid concentration of 15.4% by weight and an amine content of 5.29x10⁻⁴ eqv/g.

The polymer grains had a mean grain size of 0.054 »m and a fluctuation coefficient (standard deviation/mean grain size = 0.011/0.054) of about 0.20.

### PRODUCTION EXAMPLE 2

### Production of ethylglycol dimethacrylate-butyl methacrylate-diethylaminomethylstytene hydrochloride Coolymer Dispersion (6):

2.8 g of emulsifier (Nissan TRAX H-54, a commercial product from Nippon Fats and Oils), 75 g of distilled water, 5.95 g of ethylene glycol dimethacrylate, 4.98 g of butyl methacrylate and 5.34 g of chloromethylstyrene were put in a reactor vessel and stirred. After heating the vessel up to 60°C, 0.2 g of polymerization initiator V-50 (commercial product from Wako Pure Chemicals) were added and continuously stirred for 3 h. Afterwards, the reaction mixture was cooled to 40°C, and 108 g of distilled water and 62 g of isopropyl alcohol were dropwise added thereto over a period of 15 min. The whole was then continuously stirred for 2 h at 40°C and then filtered to obtain a polymer dispersion having a solid concentration of 8.16% by weight and an amine content of 1.31×10⁻⁴ eqv/g.

### PRODUCTION EXAMPLE 3

### Production of Poly(divinylbenzene-co-styrene-co-N,N-diethyl-N-methacryloyloxyethyl Ammonium Chloride) Polymer Dispersion (12):

108 g of distilled water were put in a reactor vessel, which was then degassed using nitrogen gas. The vessel was then heated to 60°C under a nitrogen stream, and 7.9 g of octadecyltrimethylammonium chloride (23%), 0.04 g of polyvinyl alcohol (saponification degree 95%), 0.78 g of styrene, 2.94 g of divinylbenzene and 20.63 g of N,N-diethylaminoethyl methacrylate were added thereto and stirred. A solution of 0.44 g of potassium persulfate and 0.14 g of sodium hydrogen sulfite was dissolved in 10.8 g of distilled water degassed with nitrogen gas, was added thereto and then continuously stirred for about 5 h. Afterwards, the resulting mixture was cooled to room temperature, and a solution of 10.6 g of concentrated hydrochloric acid dissolved in 100 g of distilled water was added thereto. The mixture was then filtered to obtain a polymer dispersion having a solid concentration of 14.0% by weight and an amine content of 4.59×10⁻⁴ eqv/g.

### PRODUCTION EXAMPLE 4

### Production of Poly(N,N-dimethyl-N-methacrylamidopropyl Ammonium Chloride) (Compound 17):

50.7 g of concentrated hydrochloric acid (hydrogen chloride content: 36% by weight) and 350 ml of distilled water were put in a reactor vessel, and 85 g of N,N-dimethylaminopropylmethacrylamide were gradually added thereto with stirring at room temperature.

The resulting solution was heated to 80°C under a nitrogen stream. A solution of 0.5 g of potassium persulfate dissolved in 20 ml of distilled water was added to the vessel and successively continuously stirred for 5 h. After cooling, 100 g of distilled water were added and the resulting mixture was filtered to obtain an aqueous polymer solution of Compound (17) having a solid content of 17.0% by weight and an amine concentration of 8.17×10⁻⁴ eqv/g.

Other polymers for use in the present invention can also be prepared in accordance with the production methods discussed above.

A hydrophilic protective colloid may be used as a binder for the colored layer used in the present invention. Such colloid includes, for example, gelatin, modified gelatins, gelatin derivatives and graft polymers of gelatin and other polymers. These may be used in combination with proteins such as albumin or casein; cellulose derivatives such as hydroxyethyl cellulose, carboxymethyl cellulose or cellulose sulfates; saccharide derivatives such as dextran, sodium alginate or starch derivatives; and homopolymers or copolymers such as polyvinyl alcohol, partially acetallized polyvinyl alcohol, poly-N-vinylpyrrolidone, polyacrylamide, acrylic acid or methacrylic acid copolymers or polyvinyl pyrazole. Especially preferably, gelatin is used as the hydrophilic colloid, and the gelatin may be a so-called lime-processed gelatin, acid-processed gelatin or enzyme-processed gelatin. The gelatin is especially preferably one having a narrow molecular weight distribution for the purpose of attaining rapid processing.

The molecular weight distribution of gelatin can be determined by, for example, the GPC method (gel permeation chromatography method). Gelatin having a proportion of high molecular content of 12% by weight or more, especially 14% by weight or more, is preferred for use in the present invention. The GPC method is described in detail in JP-A-62-87952 (main text and Example 1).

The colored layer used in the present invention and other hydrophilic colloid layers constituting the photographic material of the present invention are hardened with an inorganic or organic hardening agent. Suitable hardening agents include, for example, chromium salts, aldehydes (e.g., formaldehyde, glutaraldehyde), N-methylol compounds (e.g., dimethylolurea), active vinyl compounds (e.g., 1,3,5-triacryloyl-hexahydro-s-triazine, bis(vinylsulfonyl)methylether, N,N′-methylenebis(β-vinylsulfonyl)propionamide), active halogen compounds described in, for example, US-A-3,325,287 (e.g., 2,4-dichloro-6-hydroxy-s-triazine), mucohalogenic acids (e.g., mucochloric acid), N-carbamoylpyridinium salts (e.g., 1-morpholinocarbonyl-3-pyridinio)methanesulfonate), and haloamidinium salts (e.g., 1-(1-chloro-1-pyridinomethylene)pyrrolidinium, 2-naphthalenesulfonate). These can be used singly or in combination. In accordance with the present invention, hardening agents having two or more vinylsulfonyl groups (for example, those described in JP-B-47-24259, JP-B-49-13563 and JP-B-57-240902), hardening agents having two or more active vinyl groups (for example, those described in JP-A-53-41220, JP-A-53-57257, JP-A-59-162546 and JP-A-60-80846) as well as the compounds described in JP-A-62-222242, JP-A-62-245261 and JP-A-62-109050 and JP-A-62-295045 are especially preferably used, as these do not interfere with the cation site of the polymers to be used in the present invention.

The dyes to be used in accordance with the present invention are those having a selected light absorption in the spectral sensitivity range of the light-sensitive layer (to which the effect of irradiation inhibition or antihalation is intended to be provided) of the color photographic material of the present invention and especially those having a molar extinction coefficient of 10² l.mol.cm⁻¹ or more. In the color photographic materials having a reflective support, dyes which may be decolored by decoloration after development processings or which may be dissolved out of the photographic material during photographic processing are especially preferred as the dye.

The dye is preferably used in an amount of from 1 to 500 mg/m², and more preferably from 10 to 100 mg/m².

As the light absorbent for use in this invention, a dye which is substantially insoluble in an aqueous solution having pH of not higher than 7.0 is preferably used as a solid fine grain like dispersion thereof in a colloid together with a dispersion aid. The term "solid fine grain like" as used herein means a state that the dye grains having a mean grain size (projected, circle approximate) of not more than 1 »m, and preferably from 0.01 »m to 0.5 »m are dispersed in a colloid layer, said dye grains being substantially non-diffusible to other adjacent layer(s) and not aggregating coarser than about 3 »m.

As the dispersion aid, ordinary nonionic surface active agents, anionic surface active agents, and amphoteric surface active agents, such as the compounds described in patent publications cited in JP-A-62-215272, pages 649-668, and the compounds shown as practical compounds W-1 to W-99 in JP-A-62-215272, the surface active agents described in JP-B-56-36415 and 59-31688, and the surface active agents shown by formulae [VII], [VIII], and [IX] described in Japanese Patent Application No. 62-118519 can be used.

Specific examples thereof are as follows;

Also, as the dispersion aid, water-soluble organic solvents such as e.g. dimethylformamide, methanol, ethanol and dimethylsulfonylamide can be used. Furthermore, as the dispersion aid, hydrophilic colloids such as e.g. gelatin, casein, hydroxyethyl cellulose, poly-N-vinylpyrrolidone, polyacrylic acid and gelatin derivatives and also alkaline water can be used.

The solid fine grain dispersion of dye can be prepared by a method of dissolving dye solids in a water-soluble organic solvent and dispersing the solution in a neutral or acidic aqueous colloid solution, particularly preferably a method of wetting dye solids with water or an insoluble liquid, kneading the wet dye solids together with a dispersion aid, finely granulating the dye solids in a mill and dispersing them in an aqueous colloid solution, a method of fine-powdering dye solids using ultrasonic waves and dispersing the powdered dye in a colloid solution using a surface active agent as a dispersion aid, or a method of dissolving dye solids in alkaline water and dispersing the solution in an acidic aqueous colloid solution.

It is preferred that the dye or the aqueous colloid solution is used together with an organic acid such as e.g. citric acid, oxalic acid, acetic acid or tartaric acid.

The solid fine grains of dye for use in this invention may be fine crystals of the dye, micell-structural fine grains of the dye, or finely aggregated particles of the dye. The grains' size of the solid fine grains can be measured by observing the section of a colloid layer containing them using a transmission type electron microscope.

For dispersing solid fine grains of dye, a dye which is substantially insoluble in an aqueous solution having pH of not higher than 7 and which has a hydrophilic group substantially not causing proton-dissociation at pH 7 or less but causing the dissociation at pH of at least 9, such as e.g. a hydroxy group, a carboxy group, an amino group or a sulfamoyl group and thus is soluble in an aqueous solution having a pH of at least 9.0, is advantageously used in this invention. The term "substantially insoluble in an aqueous solution" as used herein means that the dispersed fine grains are insoluble to an extent capable of keeping the dispersed state in a hydrophilic colloid such as an aqueous gelatin solution having pH of not higher than 7.

A dye having a solubility in an aqueous solution of pH 7 or less at room temperature (24°C) of not more than 10% by weight, and preferably not more than 5% by weight is preferred.

The dyes can be selected from conventional known dyes, for example, arylidene dyes, styryl dyes, butadiene dyes, oxonole dyes, cyanine dyes, merocyanine dyes, hemicyanine dyes, diarylmethane dyes, triaryl dyes, azomethine dyes, azo dyes, metal-chelated dyes, anthraquinone dyes, stilbene dyes, chalcone dyes and indophenol dyes. In addition, they may also be selected from the dyes described in US-A-3,880,658, US-A-3,931,144, US-A-3,932,380, US-A-3,932,381 and US-A-3,942,987 and in J. Fabian & H. Hartmann, Light Absorption of Organic Colorants (published by Springer Verlag) as well as from non-diffusive analogues thereof.

The dyes for use in the present invention, which have the coincidence with the light absorption characteristic and which can be decolored after development processings, can be selected from the functional dyes described in JP-A-63-271351, the dyes of formula (I) described in JP-A-62-21527, JP-A-62-293243 (pages 109 to 117), JP-A-63-208846 and JP-A-63-316853 and the dyes of the formula (II) described in Japanese Patent Application No. 62-226131. For the antihalation purpose of the present invention, dyes having a light absorption in the spectral sensitivity wavelength range of the light-sensitive layer or layers, preferably the layer adjacent to the colored layer, to be provided on the colored layer are used; and for correction of the light-sensitivity range, dyes having a light absorption in the sensitivity wavelength range to be corrected are used. 80% or more of the dye to be used in the photographic emulsion layer or in other constitutional layers is preferably contained in the cationic polymer-containing layer. The amount of dye to be added is advantageously from 0.01 to 10, preferably from 0.2 to 1, as the number of the anion groups in the dye, per cation site of the cationic polymer.

Preferred dyes for use in the present invention, include the dyes described in JP-A-63-139947, JP-A-63-244034, JP-A-63-264745, Japanese Patent Application Nos. 61-314428, 62-226121, 62-277669 and 62-284448 for antihalation; and the dyes described in JP-A-63-200146, Japanese Patent Application Nos. 62-239032, 62-264396, 62-261052 and 62-247477 for correction of the spectral sensitivity.

Especially preferred dyes for use in the present invention, include the dyes described in JP-A-63-139949, JP-A-63-244034, JP-A-63-316853, Japanese Patent Application Nos. 62-226131, and 62-284448 and JP-A-62-123454.

Specific examples of the dyes which can be used in the present invention will be mentioned below .

Dye-18, Dye-37 and Dye-43 described above are suitable for the solid fine grain dispersion and furthermore, Dye-45 can be also used for the solid fine grain dispersion.

The dyes for use in this invention shown by formulae (II), (III), (IV), (V) and (VI) described below are particularly preferred for the solid fine grain dispersion. In particular, when the aforesaid dye is used for a colored layer (e.g., a colored layer utilizing colloidal silver and a layer colored by utilizing a cation polymer capable of providing cation site as a mordant), the following features can be obtained.
(1) Proper spectral absorption characteristics can be easily selected according to the using purpose of the colored layer, such as, for example, a filter layer and an antihalation layer.
(2) The dye is photochemically inactive and thus the dye does not chemically desensitize and fog an adjacent silver halide light-sensitive emulsion layer and does not fade latent images.
(3) The dye is easily dissolved off and decolored at photographic processing. Residual color or stain can not be seen.
(4) The solid fine grains of the dye do not diffuse into other layer(s). The solid fine grains have a high stability with the passage of time and further do not cause discoloring and fading.

These features are useful for the antihalation layer and the filter layer for correcting spectral sensitization distribution of color photographic materials for color print using a reflective support, such as color photographic papers, direct positive color photographic papers, and color reversal photographic papers. In the case of using the dye for the filter layer, it is preferred that the filter layer is properly formed while changing the layer construction of light-sensitive layers constituting the color photographic material, such as a blue-sensitive layer (BL), a green-sensitive layer (GL), and a red-sensitive layer (RL). Usually, a filter layer can be formed by incorporating the solid fine grains of the dye in an interlayer. Furthermore, it is preferred to use a combination of the solid fine grains of the dye and the aforesaid acidic dye.

Dyes which are used for preparing a solid fine grain dispersion can be selected from the compounds shown by following formulae (II), (III), (IV), (V) and (VI);

A₂ = L₁(̵L₂=L₃)̵ₙ A₂ (IV)

wherein A₂ (two A₂ groups may be the same or different) represents an acid nucleus having at least one substituent selected from a carboxyphenyl group, a sulfamoylphenyl group, a sulfonamidophenyl group, a carboxyalkyl group, and a hydroxyphenyl group (said acid nuclei may further have a substituent in addition to the aforesaid group), said acid nucleus being selected from 2-pyrazolin-5-one, rhodanine, hydantoin, thiohydantoin, 2,4-oxazolinedione, isoxazolinedinone, barbituric acid, thiobarbituric acid, indandione, and hydroxypyridone;

B₂ represents a basic nucleus having at least one substituent selected from a carboxy group, a sulfamoyl group, and a sulfonamido group (said basic nuclei may further have a substituent in addition to the aforesaid group), said basic nuclei being selected from pyridine, quinoline, indolenine, oxazole, benzoxazole, naphthoxazole, and pyrrole; R₄₀ represents a hydrogen atom or an alkyl group; R₄₁ and R₄₂ each represents a substituted or unsubstituted alkyl group, a substituted or unsubstituted aryl group, an acyl group, or a sulfonyl group, said R₄₁ and R₄₂ may combine with each other to form a 5- or 6-membered ring; R₄₃ and R₄₆ each represents a hydrogen atom, a hydroxy group, an alkyl group, an alkoxy group or a halogen atom; R₄₄ and R₄₅ each represents a hydrogen atom; or R₄₁ and R₄₄ or R₄₂ and R₄₅ form a non-metallic atomic group necessary for forming a 5- or 6-membered ring by the combination thereof; L₁, L₂, and L₃ each represents a substituted or unsubstituted methine group; X₃ and Y₃ each represents an electron attractive group, either X₃ or Y₃ having at least one carboxyphenyl group, sulfamoylphenyl group, sulfonamidophenyl group, carboxyalkyl group, or hydroxyphenyl group; m represents 0 or 1; n represents 0, 1, or 2; and p represents 0 or 1, when p is 0, said R₄₃ represents a hydroxy group or a carboxy group and said R₄₄ and R₄₅ represent a hydrogen atom.

Then, the formulae (II), (III), (IV), (V), and (VI) described above are explained in detail.

The carboxyphenyl group of the acidic nucleus shown by A₂ and the carboxyphenyl group of the electron attractive group shown by X₃ or Y₃ include not only a phenyl group having only one carboxy group but also a phenyl group having 2 or 3 carboxy groups. Also, the sulfamoylphenyl group, the sulfonamidophenyl group, and the hydroxyphenyl group of the acid nucleus shown by A₂ and of the electron attractive group shown by X₃ or Y₃ each includes not only a phenyl group having only one sulfamoyl group, sulfonamido group or hydroxy group but also a phenyl group having 2 or 3 sulfamoyl groups, sulfonamido groups, or hydroxy groups. The aforesaid carboxyphenyl group or the sulfamoylphenyl group, sulfonamidophenyl group and hydroxyphenyl group each may further have another substituent than the aforesaid groups [as to the substituent, there is no particular restriction if the substituent is a dissociative substituent having pKa (acid dissociation constant) in a solution of water and ethanol (1 : 1 by volume ratio) of at least 4 or a non-dissociative substituent].

Practical examples of these groups are 4-carboxyphenyl, 3,5-dicarboxyphenyl, 2,4-dicarboxyphenyl, 3-carboxyphenyl, 2-methyl-3-carboxyphenyl, 3-ethylsulfamoylphenyl, 4-phenylsulfamoylphenyl, 2-carboxyphenyl, 2,5-dicarboxyphenyl, 2,4,6-trihydroxyphenyl, 3-benzenesulfonamidophenyl, 4-(p-cyanobenzenesulfonamido)phenyl, 3-hydroxyphenyl, 2-hydroxyphenyl, 4-hydroxyphenyl, 2,4-dihydroxyphenyl, 3,4,5-trihydroxyphenyl, 2-hydroxy-4-carboxyphenyl, 3-methoxy-4-carboxyphenyl, and 2-methyl-4-phenylsulfamoylphenyl. Such a group may be bonded to the acidic nuclei or the electron attractive group directly or through a methylene group, an ethylene group, or a propylene group.

The carboxyalkyl group of the acidic nucleus shown by A₂ or of the electron attractive group shown by X₃ or Y₃ has preferably from 1 to 10 carbon atoms and specific examples thereof are carboxymethyl, 2-carboxyethyl, 3-carboxypropyl, 2-carboxypropyl, 4-carboxybutyl, and 8-carboxyoctyl.

The alkyl group shown by R₄₀, R₄₃, or R₄₆ has preferably from 1 to 10 carbon atoms and specific examples thereof are methyl, ethyl, n-propyl, isoamyl, and n-octyl.

The alkyl group shown by R₄₁ or R₄₂ has preferably from 1 to 20 carbon atoms and specific examples thereof are methyl, ethyl, n-propyl, n-butyl, n-octyl, n-octadecyl, isobutyl, and isopropyl. The alkyl group may have a substituent [such as a halogen atom (e.g., chlorine or bromine), a nitro group, a cyano group, a hydroxy group, a carboxy group, an alkoxy group (e.g., methoxy and ethoxy), an alkoxycarbonyl group (e.g., methoxycarbonyl and i-propoxycarbonyl), an aryloxy group (e.g., phenoxy), a phenyl group, and amido group (e.g., acetylamino and methanesulfonamido), a carbamoyl group (e.g., methylcarbamoyl and ethylcarbamoyl), and a sulfamoyl group (e.g., methylsulfamoyl and phenylsulfamoyl)].

The aryl group shown by R₄₁ or R₄₂ is preferably a phenyl group or a naphthyl group and may have a substituent such as the group illustrated above as the substituent for the alkyl group shown by R₄₁ or R₄₂ and an alkyl group (e.g., methyl and ethyl).

The acyl group shown by R₄₁ or R₄₂ has preferably from 2 to 10 carbon atoms and specific examples thereof are acetyl, propionyl, n-octanoyl, n-decanoyl, isobutanoyl, and benzoyl.

Examples of the alkylsulfonyl group and the arylsulfonyl group shown by R₄₁ and R₄₂ are methanesulfonyl, ethanesulfonyl, n-butanesulfonyl, n-octanesulfonyl, benzenesulfonyl, p-toluenesulfonyl and o-carboxybenzenesulfonyl.

The alkoxy group shown by R₄₃ or R₄₆ has preferably from 1 to 10 carbon atoms and specific examples thereof are methoxy, ethoxy, n-butoxy, n-octoxy, 2-ethylhexyloxy, isobutoxy, and isopropoxy.

As the halogen atom shown by R₄₃ or R₄₆, there are chlorine, bromine, and fluorine.

As the ring formed by R₄₁ and R₄₄ or by R₄₂ and R₄₅, there is, for example, a durolysine ring.

Also, examples of the 5- or 6-membered ring formed by R₄₁ and R₄₂ are, for example, a piperidine ring, a morpholine ring, and a pyrrolidine ring.

The methine group shown by L₁, L₂, and L₃ may have a substituent such as, e.g., methyl, ethyl, cyano, phenyl, hydroxypropyl and a chlorine atom.

The electron attractive group shown by X₃ and Y₃, which may be the same or different, each is a cyano group, a carboxy group, an alkylcarbonyl group which may be substituted (e.g., acetyl, propionyl, heptanoyl, dodecanoyl, hexadecanoyl, and 1-oxo-7-chloroheptyl), an arylcarbonyl group which may be substituted (e.g., benzoyl, 4-ethoxycarbonylbenzoyl, and 3-chlorobenzoyl), an alkoxycarbonyl group which may be substituted (e.g., methoxycarbonyl, ethoxycarbonyl, butoxycarbonyl, t-amyloxycarbonyl, hexyloxycarbonyl, 2-ethylhexyloxycarbonyl, octyloxycarbonyl, decyloxycarbonyl, dodecyloxycarbonyl, hexadecyloxycarbonyl, octadecyloxycarbonyl, 2-butoxyethoxycarbonyl, 2-methylsulfonylethoxycarbonyl, 2-cyanoethoxycarbonyl, 2-(2-chloroethoxy)ethoxycarbonyl, and 2-[2-(2-chloroethoxy)ethoxy]ethoxycarbonyl), an aryloxycarbonyl group which may be substituted (e.g., phenoxycarbonyl, 3-ethylphenoxycarbonyl, 4-ethylphenoxycarbonyl, 4-fluorophenoxycarbonyl, 4-nitrophenoxycarbonyl, 4-methoxyphenoxycarbonyl, and 2,4-di(t-amyl)phenoxycarbonyl), a carbamoyl group which may be substituted (e.g., carbamoyl, ethylcarbamoyl, dodecylcarbamoyl, phenylcarbamoyl, 4-methoxyphenylcarbamoyl, 2-bromophenylcarbamoyl, 4-chlorophenylcarbamoyl, 4-ethoxycarbonylphenylcarbamoyl, 4-propylsulfonylphenylcarbamoyl, 4-cyanophenylcarbamoyl, 3-methylphenylcarbamoyl, 4-hexyloxyphenylcarbamoyl, 2,4-di-(t-amyl)phenylcarbamoyl, 2-chloro-3-(dodecyloxycarbonyl)phenylcarbamoyl, and 3-(hexyloxycarbonyl)phenylcarbamoyl), a sulfonyl group (e.g., methylsulfonyl and phenylsulfonyl), or a sulfamoyl group which may be substituted (e.g., sulfamoyl and methylsulfamoyl).

Then, specific examples of the dyes which are particularly suitably used for the solid fine grain dispersion in this invention are illustrated below.

The aforesaid dyes for use in this invention can be easily synthesized by the methods described in WO 88/04794, EP-A-274,723, JP-A-52-92716, 55-155350, 55-155351, 61-205934, and 48-68623, US-A-2,527,583, US-A-3,486,897, US-A-3,746,539, US-A-3,933,798, US-A-4,130,429, and US-A-4,040,841 and by similar manners to the aforesaid methods.

In accordance with the present invention, the cationic polymer is dispersed in the hydrophilic colloid in the form of an aqueous solution or a latex. In the former case of a water-soluble cationic polymer, a dye may further be added to give a coating liquid for the colored layer. In the latter case of a cationic polymer latex, a master coating liquid to which previously a dye is added may be diluted and dispersed in the hydrophilic colloid to form a coating liquid. The dispersion containing a water-soluble cationic polymer would coagulate relatively easily, thus, a small amount of dye is used relative to the cationic polymer. The amount of the cationic polymer to be used is, although this can vary in accordance with the condition in the use thereof, preferably from about 1 g to about 100 g, more preferably from about 1 to about 50 g, especially preferably from about 1 to about 20 g, per 100 g of the hydrophilic protective colloid. The cationic polymer is used in an amount of 0.1 or more, preferably from 0.1 to 100, especially preferably from 1 to 5, as the number of the cation sites of the polymer, per one anionic group of the anionic compound of the dye to be used. The amount of the water-soluble cationic polymer to be used is preferably from 1 to 20 g per 100 g of the hydrophilic protective colloid, and it corresponds to from 5 to 30 cation sites of the polymer to one anionic group of an acidic dye.

The coating liquid for the colored layer contains a non-ionic, ampholytic or anionic surfactant, and preferably it contains a cationic surfactant. In the case of a water-soluble cationic polymer, it is preferably combined with a polymer latex dispersion, especially with a cationic polymer latex dispersion. The water soluble cationic polymer and the cationic polymer latex dispersion may be used in an optional proportion, however, it is preferable that the weight ratio of the amount of the polymer in the latex dispersion to the amount of the water soluble cationic polymer is not more than 1/2.

The mean grain size of the fine grains of the cationic polymer latex for use in the present invention is 1 »m or less, preferably from 1 to 0.001 »m, especially from 0.2 to 0.01 »m, and the grain size distribution of the grains is preferably narrow. Other polymer latexes as described in US-A-3,411,911 and US-A-3,411,912 and JP-B-45-5331 can also be co-used in the photographic constitutional layers. For instance, when an anionic compound such as an acidic dye is adsorbed on the polymer and dispersed, it is preferred that the anionic compound is previously adsorbed on the cation site of the polymer and then dispersed. By such a dispersion method, the anionic compound is prevented from being desorbed by the action of the co-existing anionic surfactant and the anionic group for the hydrophilic colloid itself.

The colored layer is coated on the support, and it may be directly coated on the white pigment-containing waterproof resin layer and dried thereon. It is preferred to provide an interlayer between the support and the colored layer. Any other silver halide light-sensitive layer may be inserted between the two layers. Two or more colored layers may be provided in a photographic material. The colored layer is provided between the support and the silver halide light-sensitive layer closest to the support. It is preferred that the colored layer is provided so that the spectral sensitivity distribution of the silver halide light-sensitive layer between the colored layer and the support may be corrected.

Depending on the position of the colored layers, dyes are usually included therein and preferably differ from each other.

When a blue sensitive layer, a green sensitive layer, a red sensitive layer and a protective layer, for example, are provided on a support in this order, the colored layer may be provided between the support and the blue sensitive layer. In this case the colored layer acts as an antihalation layer. The colored layer may also be provided between two emulsion layers, for example, between the green sensitive layer and the red sensitive layer. In this case the colored layer acts as an antihalation layer for the red sensitive layer and also acts as an irradiation inhibiting layer having light filtering effect for the green and blue sensitive layers (also acts as an antihalation layer).

The thickness of the colored layer is preferably from 0.1 to 10 »m, preferably from 0.2 to 5 »m. The maximum spectral reflection density thereof is preferably 0.2 or more, especially preferably from 0.3 to 1.5.

The silver halide emulsion to be used for preparing the photographic material of the present invention is preferably a silver chlorobromide emulsion, and it may be prepared in accordance with the methods described in P. Glafkides, Chimie et Physique Photographique (published by Paul Montel, 1967), G.F. Duffin, Photographic Emulsion Chemistry (published by Focal Press, 1966), V.L. Zelikman et al, Making and Coating Photographic Emulsion (published by Focal Press, 1964). Specifically, it may be prepared by any method including the acid method, neutral method and ammonia method, but it is preferably prepared by the acid method. The reaction of the soluble silver salt and soluble halide(s), can be carried out by methods including the single jet method, double jet method or combination thereof. The double jet method is especially preferred so as to obtain the monodispersed grains for use in the present invention. A so-called reverse mixing method where grains are formed under conditions of excess silver ions can also be employed. One type of the double jet method, i.e., a so-called controlled double jet method, where the silver ion concentration in the liquid phase to form silver chlorobromide is kept constant, may also be used. According to the method, a mono-dispersed silver chlorobromide emulsion which comprises grains having a regular crystal form and having a narrow grain size distribution and which is suited for use in the present invention can be obtained.

The above-mentioned grains which are preferably used in the present invention are desirably prepared on the basis of the double jet method. Suitable silver halide composition include compositions having a silver chloride content of 15 mol% or more. The silver chloride content is preferably 95 mol% or more, and more preferably 98 mol% or more for the photographic material which is required to have rapid processability. The composition of the silver halide may contain silver iodide in an amount not exceeding 1 mol%, but the photographic material which is required to have rapid processability desirably contains no silver iodide.

When the silver halide grains for use in the present invention are silver chlorobromide grains having a silver chloride content of 90 mol% or more, they are preferably hetero-structural grains having a "localized phase" where the silver bromide content is different from that in the adjacent phase.

The localized phase may be in the inside and/or on the surface of the silver halide grain. The localized phase may be on the surface of the grain non-uniformly or discontinuously or isolated from others on the surface Above all, the localized phase is preferably on the surface of the silver halide grain non-uniformly or is isolated from others. The silver bromide content in the localized phase is preferably at least 5 mol%, more preferably 10 mol% or more, esepcially preferably 20 mol% or more. The upper limit is preferably 70 mol%. If the silver bromide content is too high, the material would be desensitized under pressure, or the sensitivity or gradation would fluctuate in continuous development processing. The silver bromide content in the localized phase as well as the difference in the silver bromide content between the localized phase and the base phase (area other than the localized phase in the grain) is varied depending on the proportion of the silver bromide to the total silver halide, the molar ratio of the bromide used, the speed of feeding the water-soluble bromide to base grains and the pAg and pH of the reaction solution in forming the silver halide grains. For forming a localized phase in the silver halide grain as a layer, a silver nitrate solution and a halogen ion are added at a determined ratio, during the step of forming the base grain or after forming the same, while properly controlling the pAg and pH values in the reaction system. Alternatively, the silver chloride on the surface of the grain may be substituted by silver bromide by halogen substitution. The so-called CR-compounds described in, for example, EP-B-0273404, EP-B-0273429, EP-B-0274330, GB-B-2,206,974 and JP-A-63-235939 are used and a water-soluble bromide and silver nitrate are added to the base grains or fine silver bromide grains are added thereto for physical-ripening, whereby the nonuniform or isolated localized phase, which are especially advantageous for the silver halide grains for use in the present invention, is formed on the base grain.

The hetero-structual grains for use in the present invention advantageously contain a metal ion selected from metal ions of Group VIII in the Periodic Table, for example, an iron ion, rhodium ion, iridium ion or platinum ion. Especially, the metal ion is preferred to be incorporated into the localized phase or the base phase of the silver halide grains in a different concentration. For instance, it is preferred that iridium ion or iron ion is incorporated into the localized phase while a different metal ion selected form osmium, iridium, platinium, ruthenium, palladium, cobalt and nickel ions or a complex ion thereof is incorporated into the base phase in combination. Other metal ions of cadmium, zinc, lead, mercury and thallium ions may also be used. The amount of the metal ion to be incorporated into the silver halide grain is from 10⁻⁸ to 10⁻⁵ mol per mol of silver halide.

The silver bromide content in the localized phase can be analyzed by an X-ray diffraction method (for example, as described in "New Experimental Chemistry, Lecture VI, Analysis of Structure" (edited by Japan Chemical Society and published from Maruzen, Japan) or XPS method (for example, as described in "Surface Analysis - Application of IMA, Auger Electron and Photoelectronic Spectrography" (published by Kodansha, Japan).

The silver bromide content in the localized phase as existing non-uniformly or being isolated on the surface of the silver halide grain, especially in the edges or corners thereof, can be determined by the EDX (energy dispersive X-ray analysis) method (for example, described in H. Soejima, Electron Ray Microanalysis, published from Nikkan Kogyo Newspaper Co., 1987), with an EXD spectrometer as installed in a transmission type electron microscope, up to an accuracy of about 5 mol% with an aperture of from about 0.1 to about 0.2 »m diameter.

The silver halide grains for use in the present invention may be regular crystal grains, for example, cubic or 6-hedral or 14-hedral grains having (100) plane or 8-hedral grains having (111) plane, or may also be tabular grains. Such silver halide grains can selectively be formed by properly adjusting the pAg or pH value in the reaction solution for forming the silver halide grains, or by selectively using CR-compounds having a function of selectively adsorbing to (100) plane or (111) plane (for example, described in the above-mentioned patent specifications) or using any other appropriate organic compounds. In particular, 6-hedral or 14-hedral silver halide grains having (100) plane and having the localized phase in the corner parts of the surface thereof as well as tabular silver halide grains having the localized phase in the corner parts or edge parts of the surface thereof are preferred for use in the present invention.

The color photographic paper according to the present invention is processed by a "printer processor" as described in, for example, JP-A-62-184446 to form an image. It is first imagewise exposed, for example, with a CRT exposure system and then, generally, immediately subjected to color development. The color photographic paper according to the present invention which contains a silver chloride-rich silver halide emulsion is especially preferred to be rapidly processed.

The balance of the red-sensitivity (S_{R}), green-sensitivity (S_{G}) and blue-sensitivity (S_{B}) in general color photographic papers is low in the order of S_{B}, S_{G} and S_{R}. The light emitted from red-fluorescent bodies has a wavelength falling near the range of from 600 to 630 nm and near 700 nm, and therefore the bodies could hardly match with the red-sensitive wavelength for color photographic materials. In accordance with the present invention, elevation of the spectral sensitivity of the preferred reflection color photographic material as weel as improvement of the proper wavelength distribution of the spectral sensitivity thereof is especially important.

The characteristic aspects of the preferable reflection color photographic material of the present invention are as follows: First, a silver chlorobromide emulsion having a high silver chloride content is used for the purpose of attaining rapid processing of the material. Second, multi-layered silver halide grains (halogen composition distribution) are used and the grains are particularly chemically sensitized and spectrally sensitized, for the purpose of obtaining a sufficient spectral sensitivity necessary for compensating the sensitivity as lowered because of the dye added to the material so as to efficiently inhibit the diffusion of the luminous flux of the light applied to the material for exposure thereof. Third, an anti-halation layer is provided on a new support.

The silver chloride-rich silver chlorobromide emulsion for use in the present invention is preferably one which can form a latent image mainly on the surface of the silver chlorobromide grains.

The silver chlorobromide emulsion for use in a preferred reflection color photographic material of the present invention is one substantially comprising silver chloride or silver chlorobromide, and it has a silver iodide content of 2 mol% or less, preferably 1 mol% or less, especially preferably 0.1 mol% or less. It has a silver chloride content of at least 50 mol% or more, preferably 80 mol% or more, more preferably 90 mol% or more, especially preferably 95 mol% or more. The balance component may be silver bromide, silver iodide or silver rhodanide. The halogen components preferably form layers in the inside or surface of the silver halide grains, or are preferred to be differently and discontinuously isolated from others. Especially preferably, a silver bromide-localized phase which has a higher silver bromide content than the adjacent phases and is near the surface of the grain in layers or is discontinuously isolated from others, is used. The silver content in the localized phase is 5 mol% or more, preferably 10 mol% or more, especially preferably from 20 mol% to 70 mol%.

The silver halide grains to be contained in the silver halide emulsion for use in the reflection color photographic material of the present invention may have any crystal habit, but they are preferably regular crystal grains such as cubic, 14-hedral or 8-hedral grains or tabular grains rather than spherical grains or polymorphic grains. The silver halide grains are preferably multi-layered grains having different crystal structures in the inside of the grain or near the surface thereof. Especially preferred are grains having a layered structure composed of different halogen compositions or grains having a silver bromide-localized phase near the surface of the grain. When the grains are core/shell grains, it is preferred that the silver chloride content in the core part is higher than that in the shell part.

Silver halide grains having a high silver chloride content (hereinafter referred to as "high silver chloride grains") for use in the photographic material of the present invention are generally formed only in the form of cubic grains composed of (100) plane, but they may be obtained also in the form of 8-hedral grains having (111) plane or tabular grains, as the case may be, by any particular means. Preparation of 8-hedral grains having (111) plane is disclosed in JP-A-63-212932, JP-A-55-26589, Claes et al, Journal of Photographic Science, Vol. 21, page 39 (1973) and Wyrsh, International Congress of Photographic Science, III-13, page 122 (1978). The method described in JP-A-63-212932 is preferred.

For forming regular crystal grains having (111) plane, the compound as represented by the general formula (I) or (II) mentioned in JP-A-63-212932, or a compound of a formula:
where Z¹ represents an atomic group which comprises carbon, nitrogen, oxygen and/or sulfur atoms to form a 3-membered to 8-membered hetero ring together with the sulfur atom in the formula, or a compound of a formula:
where n represents an integer of from 1 to 3 and Z² represents an atomic group for forming a 3-membered to 8-membered ring together with the oxygen atom and the thiocarbonyl group in the formula, as described in JP-A-63-25643, pages 2 to 6, is preferably added during formation of the grains, especially preferably during the step of growing the grains after formation of the core grains, thereby to control the crystal habit of the grains to be formed. For formation of tabular grains for use in the present invention, the above-mentioned sulfur-containing heterocyclic compound or a compound of a formula:

R₁ - S - (X)ₘ - Y - R₂

where X represents a divalent group, including an alkylene, arylene, alkenylene, -SO₂-, -SO-, -O-, -S-, -CO- or -NR₃-, R₁ represents a hydrogen atom, an alkyl group, an aryl group or a heterocyclic group, R₂ represents a hydroxyl group, an alkyl group, an aryl group, a heterocyclic group, an amino group, an alkoxy group or an arylthio group, Y represents -CO- or -SO₂-, m represents 0 or 1, R₃ represents a hydrogen atom, an alkyl group or an aryl group, and the groups may optionally be further substituted, as described in JP-A-63-41845, is preferably added during the formation of the grains for the purpose of controlling the crystal habit of the grains to be formed. In particular, in formation of high silver chloride-tabular grains, the chloride concentration in the aqueous gelatin solution to be added during formation of the core grains is advantageously low, i.e., 0.15 mol/l or less. The chloride concentration during the step of growing the grains is preferably 5 mol/l or less, especially from 0.07 to 3 mol/l.

The silver chlorobromide grains for use in the preferred reflection color photographic material can be formed by growing grains after forming core grains by adding silver ion and a chloride or bromide or a mixture thereof thereto preferably in the presence of the above-mentioned crystal habit-controlling compound. Preferably, for forming the grains fine silver halide grains, for example fine silver bromide grains or fine silver chloride grains or a mixture thereof may be blended with a silver chloride, silver bromide or silver chlorobromide emulsion. By recrystallization or halogen-conversion of the silver halide, layer-structured grains or grains having an isolated and localized phase in the surface of the grain can be formed. Formation of the grains is preferably effected at 10 to 95°C, especially at 40 to 90°C.

Suitable silver halide solvents which can be used in formation of the grains include thiocyanates, thioethers and thioureas. Ammonia may also be used in an amount which does not badly interfere with the formation of the grains.

For instance, thiocyanates (for example, those described in US-A-2,222,264, US-A-2,448,534 and US-A-3,320,069), thioether compounds (for example, those described in US-A-3,271,157, US-A-3,574,628, US-A-3,704,130, US-A-4,297,439 and US-A-4,276,347), thione compounds (for example, those described in JP-A-53-144319, JP-A-53-82408 and JP-A-55-77737) and amine compounds (for example, those described in JP-A-100717) can be used for this purpose.

In the step of forming the silver halide grains or in the step of physical ripening of the grains formed, a cadmium salt, a zinc salt, a lead salt, a thallium salt, an indium salt or a complex salt thereof, a rhodium salt or a complex salt thereof, or an iron salt or a complex salt thereof may be added. In particular, use of an iridium salt, rhodium salt, iron salt or complex salt thereof is preferred.

In the step of preparing the silver halide grains for use in the present invention, a silver salt solution (for example, aqueous AgNO₃ solution) and a halide solution (for example, aqueous NaCl solution) are added for the purpose of accelerating the speed of grain formation. Preferably, the addition speed, the amount of the solutions to be added and the concentration of the solutions are elevated so as to accelerate the speed of grain formation.

Details of this method, for example, are disclosed in GB-B-1,335,925, US-A-3,672,900, US-A-3,650,757 and US-A-4,242,445 and JP-A-55-142329, JP-A-55-158124, JP-A-58-113297, JP-A-58-113928, JP-A-58-111934 and JP-A-58-111936.

The structure of the surface and near the surface of the high silver chloride grains used according to the present invention is important for the sensitivity, stability and reciprocity characteristics of the emulsions and for the stability of the latent images to be formed. In the final step of forming the silver halide grains, for example, after 85 mol% or more of the total silver halide grains have been grown up to the intended degree, the method of forming grains as well as CR-compounds (inhibitor for halogen conversion or chemical sensitization) described in Japanese Patent Application No.s 62-86252, 62-329265 and 62-152330 are preferably employed.

If a halide is added to the silver halide grains, after the CR-compound (discussed hereinafter) has been adsorbed thereto, the halide is preferably a halogen-donor which can control the feeding speed of chloride ion or bromide ion or control the amount of the ion to be fed. According to the method, a silver bromide-localized phase which has a silver bromide content different from the adjacent phase may be formed in the surface and/or near the surface of the silver halide grain.

The high silver chloride emulsion of the photographic material contains silver halide grains having a diameter preferably of from 0.1 to 3 »m as the diameter of a circle corresponding to the projected area of the grain, in an amount of 50% or more of the total grains as the projected area thereof. When the grains are tabular grains, the ratio of the circle-corresponding diameter to the grain thickness (hereinafter referred to as "aspect ratio") is preferably 2 or more, more preferably from 3 to 10, especially preferably from 5 to 8. The high silver chloride emulsion according to the present invention is preferably a monodispersed emulsion, and the emulsion preferably has a dispersion coefficient of the circle-corresponding diameter (ratio of the standard deviation of the circle-corresponding diameter to the mean grain size) of 0.15 or less.

Another preferred characteristic feature of the present invention resides in the method of chemical sensitization of the silver halide grains. Specifically, in accordance with the chemical sensitization according to the present invention, the emulsion containing high silver chloride grains having a localized phase is subjected to gold sensitization, especially to a combination of sulfur sensitization and gold sensitization, in the presence of a compound for controlling the chemical sensitization. This method is especially preferred to apply for production of the reflection colour photographic material.

The high silver chloride emulsion to be subjected to gold sensitization is especially a green-sensitive emulsion and a red-sensitive emulsion. Especially preferably, a red-sensitive emulsion is gold-sensitized.

The conditions (e.g., pH, pAg, temperature, time) for gold sensitization for the emulsions according to the present invention are not specifically limited, but the pH value is preferably from 3.0 to 8.5, especially from 5.0 to 7.5, the pAg value is preferably from 5.0 to 9.0, especially from 5.5 to 7.5, the temperature is preferably from 40 to 85°C, especially from 45 to 75°C, and the time is preferably from 10 to 200 min, especially from 30 to 120 min.

Preferred gold sensitizer compounds include the compounds described in US-A-2,399,083, US-A-2,540,085, US-A-2,540,086 and US-A-2,597,856. For example, suitable compounds include chloroauric acid and salts thereof, potassium gold cyanide, potassium gold thiocyanate and gold sulfide. Intensification of gold sensitization by the combined use of thiocyanates as well as the use of tetra-substituted thiourea compounds in combination with the gold sensitizer for gold sensitization, as described in JP-B-59-11892, is also advantageous.

Suitable sulfur sensitizers which can be used in combination with the gold sensitizers include, for example, thiosulfates, sulfinic acid salts, thioureas, thiazoles, rhodanines and other compounds described in US-A-1,574,944, US-A-2,410,689, US-A-2,728,668 and US-A-3,656,955. In addition, the sulfur-containing compounds described in US-A-3,857,711, US-A-4,266,018 and US-A-4,054,457 can also be used for the purpose.

The amount of the gold sensitizer to be used in accordance with the present invention is from about 10⁻⁸ mol to about 10⁻⁵ mol per mol of silver halide and is selected so that it may elevate sensitivity with low fog. By combination with a chemical sensitization-inhibitor, it may be used in a relatively small amount to attain a high sensitivity with low fog. Use of the gold sensitizer in a relatively small amount in accordance with the intended sensitivity is preferred.

Regarding the amount of the sulfur sensitizer to be used together with the gold sensitizer, an optimum amount may be selected in accordance with the grain size, temperature of chemical sensitization, and other conditions of pAg and pH. For instance, the sulfur sensitizer may be used in an amount of from 10⁻⁷ to 10⁻³ mol, preferably from 5×10⁻⁷ to 10⁻⁴ mol, more preferably from 5×10⁻⁷ to 10⁻⁵ mol, per mol of silver halide. When gold/sulfur sensitization is effected in combination, the chemical sensitization is preferably conducted in the presence of sulfur sensitizer and gold sensitizer in a ratio of at least 100/250 by mol%.

The silver halide emulsion used in the present invention can be processed with an oxidizing agent, after the formation of the grains. This method is discussed in JP-A-60-136736. Hydrogen peroxide can be used as the oxidizing agent.

At least one compound represented by anyone of the following formulae (S-I) to (S-III) is preferably added to the high silver chloride emulsion for use in the present invention, especially when a gold sensitizer is used, to noticeably effectively inhibit fog formation. It may be added to the emulsion at any time in the step of forming grains, the step of desalting, the step of chemical-ripening or immediately before coating. Especially preferably, it is added in the: step of forming grains, desalting or chemical-ripening, and particularly before the addition of the gold sensitizer to the emulsion. Compounds containing a thiosulfonyl group of formulae (S-I), (S-II) and (S-III) are mentioned below.

(S-I) Z-SO₂S-M

In these formulae, Z represents an alkyl group, an aryl group or a heterocyclic group, which are or are not further substituted. Y represents an atomic group necessary for forming an aromatic ring or hetero ring, which is or is not further substituted. M represents a metal atom or an organic cation. n represents an integer of from 2 to 10.

Substituents for the alkyl group, aryl group, aromatic ring or heterocyclic ring include a lower alkyl group such as methyl or ethyl group, an aryl group such as phenyl group, an alkoxy group having from 1 to 8 carbon atoms, a halogen atom such as chlorine, a nitro group, an amino group and a carboxyl group.

The alkyl group for Z has from 1 to 18 carbon atoms; and the aryl group and aromatic ring for Z and Y independently have from 6 to 18 carbon atoms.

The hetero ring represented by Z and that including Y include thiazole, benzothiazole, imidazole, benzimidazole and oxazole rings. When M is a metal cation, M preferably represents alkali metal cations such as sodium or potassium ions as well as organic cations such as ammonium or guanidinium ions.

Specific examples of the compounds of the formulae (S-I), (S-II) and (S-III) are mentioned below.

e H₃C·SO₂·SNa

- k: L-cysteine-disulfoxide
- ℓ: H₅C₂·SO₂·S·K
- m: H₁₇C₈·SO₂SNa

The compounds of the formulae (S-I), (S-II) and (S-III) can be used together with sulfites or sulfinic acid salts such as alkylsulfinic acid salts, arylsulfinic acid salts or heterocyclic sulfinic acid salts.

The silver halide emulsion for use in the present invention is preferably physically ripened in the presence of a known silver halide solvent (for example, ammonia, potassium thiocyanate or thioether or thione compounds described in US-A-3,271,157 and JP-A-51-12360, JP-A-53-82408, JP-A-53-144319, JP-A-54-100717 and JP-A-54-155828), whereby it may be converted into a monodispersed silver halide emulsion having a regular crystal shape and a narrow grain size distribution.

In order to remove soluble silver salts from the physically ripened emulsion, the emulsion may be subjected to noodle washing, flocculation precipitation or ultrafiltration.

The silver halide emulsion for use in the present invention can be chemically sensitized by sulfur sensitization, selenium sensitization, reduction sensitization and/or noble metal sensitization. Such chemical sensitization methods may be effected singly or in combination. Specifically, the emulsion may be treated by a sulfur sensitization method using a sulfur-containing compound capable of reacting with active gelatin or silver ion (e.g., thiosulfates, thiourea compounds, mercapto compounds, rhodanine compounds), reduction sensitization method using a reducing substance (e.g., stannous salts, amines, hydrazine derivatives, formamidinesulfinic acids, silane compounds) and/or noble metal sensitization method using a metal compound (e.g., gold complexes or complexes of metals of VIII group of the Periodic Table such as Pt, Ir, Pd, Rh or Fe). These methods can be used singly or in combination. A monodispersed silver chlorobromide emulsion is preferably sensitized by sulfur sensitization or selenium sensitization, advantageously in the presence of a hydroxyazaindene compound.

In accordance with the present invention, the monodispersed degree of the silver chlorobromide emulsion is preferably 0.15 or less, especially 0.1 or less, as the fluctuation coefficient thereof.

Chemical sensitization of the silver halide emulsion for use in the present invention can be effected by the conventional methods mentioned above. When the silver halide grains of the emulsion have a silver bromide-localized phase on the surface or sub-surface of the grains, the chemical sensitization of the emulsion is required to be properly controlled by providing the localized phase on the base grain. Control methods described in EP-A-0273404, EP-A-0273429 and EP-A-0273430 may be employed. In particular, the method using CR-compounds is helpful (a CR-compound is used at the final step of the grain formation to restrain the halogen conversion at the grain surface or is used to restrain chemical sensitization : see EP-A-273429 or EP-A-273430).

The photographic materials of the present invention can contain various stabilizer compounds. For instance, various known stabilizer compounds include, for example, azoles such as benzothiazolium salts, nitroindazoles, triazoles, benzotriazoles, benzimidazoles (especially nitro- or halogen-substituted derivatives); heterocyclic mercapto compounds such as mercaptothiazoles, mercaptobenzothiazoles, mercaptobenzimidazoles, mercaptothiadiazoles, mercaptotetrazoles (especially 1-phenyl-5-mercaptotetrazole), mercaptopyrimidines; the above-mentioned heterocyclic mercapto compounds having a water-soluble group such as a carboxyl group or a sulfone group; thioketo compounds such as oxazolinethione; azaindenes such as tetraazaindenes (especially 4-hydroxy substituted (1,3,3a,7)tetraazaindenes); benzenethiosulfonic acids; and benzenesulfinic acids.

In accordance with the present invention, conventional methine dyes can be used for spectral sensitization. Particular monomethine, trimethine or pentamethine dyes or merocyanine dyes as described in Japanese Patent Application Nos. 62-86252, 62-152330 and 62-329265 are advantageously adsorbed to the high silver chloride grains during the step of grain growth or the step of chemical sensitization thereof, as a chemical sensitization controlling agent.

The dyes to be used for spectrally sensitizing the silver halide emulsion for use in the present invention include cyanine dyes, merocyanine dyes, complex cyanine dyes, complex merocyanine dyes, homopolar cyanine dyes, hemicyanine dyes, styryl dyes and hemioxonole dyes. Cyanine dyes, merocyanine dyes and complex merocyanine dyes are especially useful. Any and every nuclei which are usually utilized for cyanine dyes as basic heterocyclic nuclei can be applied to these dyes. That is, such nuclei include pyrroline nuclei, oxazoline nuclei, thiazoline nuclei, pyrrole nuclei, oxazole nuclei, thiazole nuclei, selenazole nuclei, imidazole nuclei, tetrazole nuclei and pyridine nuclei; the nuclei obtained by fusing alicyclic hydrocarbon rings to these nuclei; and the nuclei obtained by fusing aromatic hydrocarbon rings to these nuclei, such as indolenine nuclei, benzindolenine nuclei, indole nuclei, benzoxazole nuclei, naphthoxazole nuclei, benzothiazole nuclei, naphthothiazole nuclei, benzoselenazole nuclei, benzimidazole nuclei and quinoline nuclei. These nuclei may be substituted on the carbon atom of the dye.

5-membered or 6-membered heterocyclic nuclei can be applied to the merocyanine dyes or complex merocyanine dyes. Suitable heterocyclic nuclei include pyrazolin-5-one nuclei, thiohydantoin nuclei, 2-thiooxazolidine-2,4-dione nuclei, thiazolidine-2,4-dione nuclei, rhodanine nuclei and thiobarbituric acid nuclei, as nuclei having a ketomethylene structure. Specific examples of such spectral sensitizing dyes include the compounds of the formulae (IIIa), (IIIb) and (IIIc) described in Japanese Patent Application No. 62-227338.

The amount of the dye to be added may be from 1×10⁻⁶ to 8×10⁻³ mol per mol of silver halide in the emulsion layer. When the silver halide grains have a preferred grain size of from 0.2 to 1.2 »m, the amount may be more effectively from about 5×10⁻⁵ to 2×10⁻³ mol per mol of the silver halide.

The tabular silver halide emulsion is preferred to be spectrally sensitized in a blue range and used in the blue-sensitive emulsion layer. "Spectral sensitization in a blue range" as referred to herein means that the emulsion contains a spectrally sensitizing dye which may give at least one absorption peak in the range of from 400 to 500 nm, preferably from 430 to 490 nm, more preferably from 445 to 490 nm, when adsorbed to the emulsion grains. Examples of such blue-spectrally sensitizing dye include the compounds of the formulae (IIIa) and (IIIc) where n₃₁ is 0 (zero) described in Japanese Patent Application No. 62-227338. Specific examples of the compounds include the compounds (III-1) to (III-8) and (III-29) to (III-32) described in Application No. 62-227338. High silver chloride-tabular grains formed in the presence of such dyes are preferably used in the present invention.

High silver chloride-tabular grains formed in the presence of the dye can be confirmed by the spectral sensitivity distribution of the grains. In general, it is difficult for high silver chloride emulsions to give a sharp spectral sensitivity distribution. However, when the grains are formed in the presence of the dye in accordance with the present invention, the resulting emulsion may give a sharp J-band for the methine dyes of the formulae (IIIa) and (IIIb), or the resulting emulsion may give a sharp monomer band (M-band) for the merocyanine dyes of the formula (IIIc). Anyway, the emulsion formed in the presence of the dye may give a sharp spectral sensitivity distribution.

Accordingly, formation of the grains in the presence of the dye can be confirmed by identification of the peak wavelength, the spectral sensitivity distribution and the kind of the dye used. The details of "J-band" and "M-band" are described in T.H. James, Theory of Photographic Processing, Chap. 8 (published by Macmillan, 1977).

The spectral sensitizing dyes can be used singly or in combination. They are preferably used in combination with supersensitizers. For instance, aminostilbene compounds (e.g., those described in US-A-2,933,390, US-A-3,635,721, US-A-3,615,613, US-A-3,615,641, US-A-3,617,295 and US-A-3,635,721, and JP-A-63-239449) as well as aromatic or heterocyclic mercapto compounds are preferably used as supersensitizers for the high silver chloride emulsion.

For red-spectral sensitization or spectral sensitization in the wavelength range of from 580 to 750 nm, sensitizing dyes having a reduction potential of -1.27 (V. vs SCE) or a value more anodic than the value are preferred since they give excellent sensitivity and high stability of sensitivity and latent images. Regarding the chemical structure of the compounds, pentamethinecyanine dyes having a ring-condensed structure via one or more methine chains as conjugated between nitrogen atoms, 4-quinoline nucleus-having trimethine-cyanine dyes, as well as tetramethine-merocyanine dyes and 4-quinoline nucleus-having dimethine-merocyanine dyes are preferred. Determination of reduction potential of the dyes can be effected by phase differentiation secondary higher harmonics alternate current polarography, where a dropping mercury electrode is used as the working electrode, a saturated calomel electrode as the reference electrode and a platinum as the counter electrode. Together with the sensitizing dyes, hydroquinone, catechol, aminophenol, silver halide-adsorbing formylhydrazine compounds or derivatives thereof are preferably used in combination. The details of the formhydrazine compounds are described in Japanese Patent Application No. 63-97905.

The high silver chloride emulsion used in the present invention has a lower intrinsic sensitivity in a visible ray range than any other high silver bromide emulsion. When the high silver chloride emulsion has a silver chloride content of 80 mol% or more, it may achieve the sensitivity substantially by spectral sensitization. On the other hand, since the spectral sensitivity in the blue wavelength of the silver halide emulsion used in the present invention is not mixed with the green-spectral sensitivity or red-spectral sensitivity, a method with ease of elevating the intrinsic sensitivity of the silver halide emulsion to substantially elevate the spectral sensitivity thereof, may be necessary.

Accordingly, it is extremely advantageous to combine gold sensitization for elevating the intrinsic sensitivity of the silver halide emulsion and the above-mentioned spectral sensitization, whereby the spectral sensitivity of the respective blue, green and red light-sensitive layers may well be balanced therebetween.

A compound having a mercapto group may preferably be added to the silver halide emulsion used in the present invention, whereby fog of the photographic material may be reduced, storage stability of the raw film may be improved and the storage stability of the emulsion coating composition before preparation of photographic materials may be improved.

For this purpose, tetrazaindenes are generally used, and it has heretofore been considered that mercapto-containing compounds should be added only in an extremely small amount (only in a determined amount) for this purpose. The mercapto compounds would be ineffective in an amount lower than the optimum range while they would noticeably cause desensitization when used in an amount higher than the optimum range. Unexpectedly, the addition of the mercapto compounds, which have heretofore been considered to have a strong adverse effect, to the emulsion of the preferred reflection color photographic material is preferred for the above-mentioned purpose, and the mercapto compounds do not cause desensitization and inhibition of development. For the high silver chloride emulsion, the compounds may be used together with sensitizing dyes to attain supersensitization.

Mercapto-containing compounds which are preferably used in the present invention are represented by the following general formula (S):
wherein M₁ represents a hydrogen atom, a cation or a protective group for mercapto group which may be cleaved by the action of an alkali; and Z₁ represents an atomic group necessary for forming a 5-membered or 6-membered hetero-ring. The hetero-ring may have substituent(s) or may also be condensed. Preferably, M₁ represents a hydrogen atom, a cation (for example, sodium ion, potassium ion, ammonium ion) or a protective group for mercapto group which may be cleaved by the action of an alkali (for example, -COR′, -COOR′ or -CH₂CH₂COR′, in which R′ represents a hydrogen atom, an alkyl group, an aralkyl group or an aryl group).

Z₁ represents an atomic group necessary for forming a 5-membered or 6-membered hetero-ring. The hetero-ring contains sulfur, selenium, nitrogen and/or oxygen atoms as a hetero atom, and this may be condensed and does or does not have substituent(s) on the hetero-ring or condensed-ring.

Examples of the hetero-ring including Z₁ include tetrazole, triazole, imidazole, oxazole, thiadiazole, pyridine, pyrimidine, triazine, azabenzimidazole, purine, tetrazaindene, triazaindene, pentazaindene, benzotriazole, benzimidazole, benzoxazole, benzothiazole, benzoselenazole and naphthoimidazole. Suitable substituents for the rings include an alkyl group (e.g., methyl, ethyl, n-hexyl, hydroxyethyl, carboxyethyl), an alkenyl group (e.g., allyl), an aralkyl group (e.g., benzyl, phenethyl), an aryl group (e.g., phenyl, naphthyl, p-acetamidophenyl, p-carboxyphenyl, m-hydroxyphenyl, p-sulfamoylphenyl, p-acetylphenyl, o-methoxyphenyl, 2,4-diethylaminophenyl, 2,4-dichlorophenyl), an alkylthio group (e.g., methylthio, ethylthio, n-butylthio), an arylthio group (e.g., phenylthio, naphthylthio), an aralkylthio group (e.g., benzylthio) and a mercapto group. The condensed rings may also have other substituents including a nitro group, an amino group, a halogen atom, a carboxyl group and a sulfo group, in addition to the aforesaid substituents.

The amount of the mercapto-containing compound to be added is preferably 10⁻³ mol or less, per mol of silver halide.

Specific examples of the mercapto group-having nitrogen-containing heterocyclic compounds which may be applied to the present invention include (A-374) to (A-827) described in JP-A-62-215272, pages 51 to 68.

Color couplers for use in the present invention will be mentioned hereunder.

Use of high active color couplers is preferred in the reflection color photographic material of the present invention. Specifically, the color couplers for use in the present invention are required to satisfy the general requirements for forming dyes having a sufficient color hue and a high extinction coefficient and are additionally required to have a sufficiently high activity to maintain a sufficient coupling coloring reaction with the oxidation product of a color developing agent such as paraphenylenediamine derivatives, since the developing speed of the emulsion used in the present invention is high. Use of couplers of the following formulae (Cup-1), (Cup-2), (Cup-3), (Cup-4) and (Cup-5) are preferred.

In these formulae, R₁, R₄ and R₅ each represent an aliphatic group, an aromatic group, a heterocyclic group, an aromatic amino group or a heterocyclic amino group;
R₂ represents an aliphatic group;
R₃ and R₆ each represent a hydrogen atom, a halogen atom, an aliphatic group, an aliphatic-oxy group or an acylamino group;
R₇ and R₉ each represents a substituted or unsubstituted phenyl group;
R₈ represents a hydrogen atom, an aliphatic or aromatic acyl group, or an aliphatic or aromatic sulfonyl group;
R₁₀ represents a hydrogen atom or a substituent;
Q represents a substituted or unsubstituted N-phenylcarbamoyl group;
Za and Zb each represents a methine group, a substituted methine group or =N-;
Y₁, Y₂ and Y₄ each represents a halogen atom or a group which can be released in coupling reaction with the oxidation product of a developing agent (hereinafter referred to as a "releasing group");
Y₃ represents a hydrogen atom or a releasing group; and
Y₅ represents a releasing group.

In formulae (Cup-1) and (Cup-2), R₂ and R₃, and R₅ and R₆ may be bonded to each other to form a 5-, 6- or 7-membered ring.

R₁, R₂, R₃ or Y₁; R₄, R₅, R₆ or Y₂; R₇ R₈ R₉ or Y₃; R₁₀, Za, Zb or Y₄; and Q or Y₅ may form a dimer or a higher polymer. R₅ and R₆ are preferably bonded to each other to form a 5-membered ring to give oxyindole or indazolin-2-one cyan couplers.

The details of R₁, R₂, R₃, R₄, R₅, R₆, R₇, R₈, R₉, R₁₀, Za, Zb, Q₁, Y₁, Y₂, Y₃ and Y₄ in formulae (Cup-1), (Cup-2), (Cup-3), (Cup-4) and (Cup-5) are the same as those in formulae (I), (II), (III), (IV) and (V) mentioned in JP-A-63-11939, pages 4 to 24.

Specific examples of the color couplers include compounds (C-1) to (C-40), (M-1) to (M-42) and (Y-1) to (Y-46) described in JP-A-63-11939, pages 11 to 24.

The standard amount of the color coupler to be used is from 0.001 to 1 mol per mol of the light-sensitive silver halide. Preferably, it is from 0.01 to 0.5 mol for yellow couplers, from 0.003 to 0.3 mol for magenta couplers, and from 0.002 to 0.3 mol for cyan couplers.

When the color coupler of the aforesaid formula (Cup-1), (Cup-2), (Cup-3), (Cup-4) or (Cup-5) is added to the photographic material, the preferred total amount of the silver halide in the material is from 0.1 g/m² to 1.5 g/m².

The color coupler can be incorporated into the emulsion layer, as dispersed in the layer together with at least one high boiling point organic solvent. The solvents preferably have a boiling point higher than 150°C, and more preferably higher than 170°C. Preferably, high boiling point solvents as represented by the following general formulae (A) to (E) are used for the purpose.

(B) W₁-COO-W₂

(E) W₁-O-W₂

In these formulae W₁, W₂ and W₃ each represent a substituted or unsubstituted alkyl, cycloalkyl alkenyl, aryl or heterocyclic group;
W₄ represents W₁, OW₁or S-W₁;
n represents an integer of from 1 to 5, and when n is 2 or more, plural W₄'s may be the same or different.

In the formula (E), W₁ and W₂ may form a condensed ring.

The photographic material of the present invention can contain, as a color-fogging inhibitor or a color mixing preventing agent, hydroquinone derivatives, aminophenol derivatives, amines, gallic acid derivatives, catechol derivatives, ascorbic acid derivatives, colorless couplers and sulfonamidophenol derivatives.

The photographic material of the present invention can contain a known anti-fading agent. Specific examples of organic anti-fading agents which can be used in the present invention include hindered phenols such as hydroquinones, 6-hydroxychromans, 5-hydroxycoumarans, spirochromans, p-alkoxyphenols and bisphenols, as well as gallic acid derivatives, dioxyphenylmethylenes, aminophenols and hindered amines and ether and ester derivatives of the compounds obtained by silylating or alkylating the phenolic hydroxyl group of the compound. In addition, metal complexes such as (bis-salicylaldoximato)nickel complexes and (bis-N,N-dialkyldithiocarbamato)nickel complexes may also be used.

For the protection of yellow dye images from heat, moisture and light, compounds having both the structures of a hindered amine and a hindered phenol in one molecule as described in US-A-4,268,593 are preferred. For the protection of magenta dye images especially from heat, spiroindanes described in JP-A-56-159644 and hydroquinone-diether or monoether-substituted chromans described in JP-A-55-89835 are preferred.

Image stabilizers described in JP-A-59-125732 are advantageous for the stabilization of magenta images formed from pyrazolotriazole magenta couplers.

In order to improve the storage stability, especially light-fastness, of cyan images, benzotriazole ultraviolet absorbents are preferably used. The ultraviolet absorbents can be co-emulsified with the cyan couplers.

The amount of the ultraviolet absorbent to be used is an amount that is sufficient for imparting light stability to the cyan dye images. If the absorbent is used in too large amount, it will cause yellowing in the non-exposed area (white background area) of the color photographic material. Accordingly, the amount is generally determined to fall within the range of from 1×10⁻⁴ mol/m² to 2×10⁻³ mol/m², especially from 5×10⁻⁴ mol/m² to 1.5×10⁻³ mol/m².

In the layers constituting conventional photographic color papers, any one of the both layers adjacent to the cyan coupler-containing red-sensitive emulsion layer, preferably both of them, contain(s) an ultraviolet absorbent. When the ultraviolet absorbent is incorporated into the interlayer between the green-sensitive layer and the red-sensitive layer, it may be co-emulsified with a color mixing preventing agent. When the ultraviolet absorbent is added to the protective layer, another protective layer may be formed thereon as an outermost layer. The outermost protective layer may contain a mat agent having any desired grain size or a latex having a different grain size in combination.

The photographic material of the present invention can contain an ultraviolet absorbent in the hydrophilic colloid layer.

In addition to the above-mentioned additives, the photographic material of the present invention can further contain various other compounds, including stabilizers, stain inhibitors, developing agents or precursors thereof, development accelerators or precursors thereof, lubricants, mordant agents, mat agents, antistatic agents, plasticizers, as well as other additives which are useful for photographic materials. Specific examples of such additives are described in Research Disclosure, Item 17643 (December 1978) and ibid., Item 18716 (November 1979).

The photographic material of the present invention can contain a brightening agent of stilbene, triazine, oxazole or coumarin compounds, in the photographic emulsion layers or in any other hydrophilic colloid layers. Water-soluble compounds can be used, or water-insoluble compounds can also be used in the form of a dispersion, as brightening agents.

The color photographic material of the present invention preferably has a yellow coupler-containing blue-sensitive silver halide light-sensitive layer, a magenta coupler-containing green-sensitive silver halide light-sensitive layer and a cyan coupler-containing red-sensitive silver halide light-sensitive layer formed on a support, and the order of the layers on the support may freely be varied in accordance with the object. Since the high silver chloride silver halide has only a slight intrinsic sensitivity in the blue-sensitive wavelength range (400 to 500 nm), the order of the layers on the support may be easily varied. For instance, red-sensitive layers, green-sensitive layers and blue-sensitive layers may be formed on a support in this order, or alternatively, a blue-sensitive layer, a red-sensitive layer and a green-sensitive layer may be formed thereon in this order.

The color sensitivity of the respective light-sensitive layers of the color photographic material of the present invention is selected in accordance with the light source for scanning exposure to be employed for the material, and the material is preferably exposed through the respective color separation filters. For instance, a combination of blue-sensitive, green-sensitive and red-sensitive layers or a combination of green-sensitive, red-sensitive and infrared-sensitive layers are mentioned.

The color photographic material of the present invention is preferably exposed by scanning exposure and then processed for color development.

The sensitizing dye for use in the present invention is preferably added during the step of chemical sensitization or before the same, or during the formation of the silver halide grains or after the formation of the same.

When the silver chlorobromide emulsion for use in the present invention contains high silver chloride-tabular grains as in the preferred reflection color photographic material, selection of the time of adding the dye is extremely important. Addition of the dye is to be effected prior to completion of formation of the silver halide precipitate, but the following method may also be employed. Generally, the dye is added after completion of the chemical sensitization but prior to coating. However, the dye may be added together with the chemical sensitizer for simultaneous spectral sensitization and chemical sensitization, as described in US-A-3,628,969 and US-A-4,225,666. Alternatively, the dye may be added prior to chemical sensitization, as described in JP-A-58-113298. Furthermore, the dye may be divided into parts, and a part thereof may be added prior to chemical sensitization and the remaining part thereof may be added after chemical sensitization, which is taught in US-A-4,225,666. The method as taught in US-A-4,183,756 may also be applied to the present invention. Anyway, the dye may be added to the silver halide grains in any stage of grain formation.

The cationic polymer for use in the present invention acts to capture the iodide ion to be dissolved out from the photographic material during development or fixation thereof, thereby accelerating the development processing speed.

In addition, the polymer acts to capture the bromide ion to be dissolved out from the photographic material during development processing thereof or the bromide ion as existing in the developer or to be carried thereinto from the outside, thereby stabilizing the color developing processing and elevating the development processing speed. In addition, in accordance with the present invention, the polymer noticeably acts to inhibit fluctuation of the photographic properties of the photographic material processed under variable processing conditions. In particular, the stability of the gradation of the toe or shoulder in the characteristic curve can be improved by the action of the polymer. The said effect of the polymer is especially noticeable when a high silver chloride emulsion having a localized silver bromide phase on the surface of the grain (preferably, silver chlorobromide emulsion having an AgCl content of 98 mol% or more) is used and the photographic material is rapidly processed at a higher temperature.

In the photographic material of the present invention, when the total amount of the silver halide is reduced to 0.9 g/m² or less, preferably 0.7 g/m² or less (not less than 0.4 g/m²) as silver, or when the light transmittance of the material is elevated by properly selecting the size and the shape of the silver halide grains, the improved image sharpness and color reproducibility due to the provision of the polymer-containing colored layer is more noticeable.

The color photographic material of the present invention generally contains yellow couplers, magenta couplers and cyan couplers which may form yellow, magenta and cyan colors, respectively, by coupling with the oxidation product of an aromatic amine color developing agent.

Preferred yellow couplers for use in the present invention include acylacetamide derivatives such as benzoylacetanilide or pivaloylacetanilide.

In particular, compounds of the following general formulae (Y-1) and (Y-2) are preferred as the yellow couplers for use in the present invention.

In these formulae, X represents a hydrogen atom or a coupling-releasing group; R₂₁ represents a non-diffusive group having a total carbon number of from 8 to 32; R₂₂ represents a halogen atom, a lower alkyl group, a lower alkoxy group or a non-diffusive group having a total carbon number of from 8 to 32; R₂₃ represents a substituent; and n and n′ represent 0 or an integer of from 1 to 4; and n′ represents 0 or an integer of from 1 to 5. When the formula (Y-1) or (Y-2) has two or more R₂₂ or R₂₃ groups, respectively, they may be the same or different. R₂₄ represents a halogen atom, an alkoxy group, a trifluoromethyl group or an aryl group; R₂₅ represents a hydrogen atom, a halogen atom or an alkoxy group; and R₂₆ represents -NHCOR₂₇, -NHSO₂R₂₇, -SO₂NHR₂₇, -COOR₂₇, and
(wherein R₂₇ and R₂₈ each represents an alkyl group, an aryl group or an acyl group).

The details of pivaloylacetanilide yellow couplers are described in US-A-4,622,287, from column 3, line 15, to column 8, line 39, and US-A-4,623,616, from column 14, line 50 to column 19, line 41.

The details of benzoylacetanilide yellow couplers are described in US-A-3,408,194, US-A-3,933,501, US-A-4,046,575, US-A-4,133,958 and US-A-4,401,752.

Specific examples of pivaloylacetanilide yellow couplers include compounds (Y-1) to (Y-39) described in the aforesaid US-A-4,622,287, columns 37 to 54. Above all, compounds (Y-1), (Y-4), (Y-6), (Y-7), (Y-15), (Y-21), (Y-22), (Y-23), (Y-26), (Y-35), (Y-36), (Y-37), (Y-38) and (Y-39) are especially preferred.

In addition, there are also mentioned compounds (Y-1) to (Y-23) described in the aforesaid US-A-4,623,616, columns 19 to 24. Above all, compounds (Y-2), (Y-7), (Y-8), (Y-12), (Y-20), (Y-21), (Y-23) and (Y-29) are preferred.

Other preferred couplers include compound (34) described in US-A-3,408,194, column 6, compounds (16) and (19) described in US-A-3,933,501, column 8, compound (9) described in US-A-4,046,575, columns 7 to 8, compound (1) described in US-A-4,133,958, columns 5 to 6, compound (1) described in US-A-4,401,752, column 5, and compounds (a) to (g) described in Japanese Patent Application No. 62-263318, pages 29 to 30.

Suitable magenta couplers for use in the present invention include oil-protect type indazolone or cyanoacetyl couplers, preferably 5-pyrazolone or pyrazoloazole couplers such as pyrazolotriazoles. 5-pyrazolone couplers wherein the 3-position is substituted by an arylamino or acylamino group are preferred from the view point of the hue and the density of the dyes to be formed therefrom. Specific examples of such couplers are described in US-A-2,311,082, US-A-2,343,703, US-A-2,600,788, US-A-2,908,573, US-A-3,062,653, US-A-3,152,896 and US-A-3,936,015. Preferred releasing groups in 2-equivalent 5-pyrazolone couplers include the nitrogen atom-releasing groups described in US-A-4,310,619 and the arylthio groups described in US-A-4,351,897. Ballast group-having 5-pyrazolone couplers described in EP-B-73,636 are preferred as they give a high color density.

Suitable pyrazoloazole couplers include pyrazolobenzimidazoles described in US-A-3,369,879, preferably pyrazolo[5,1-c][1,2,4]triazoles described in US-A-3,725,067, pyrazolotetrazoles described in Research Disclosure, Item 24220 (June, 1985) and pyrazolopyrazoles described in Research Disclosure, Item 24230 (June, 1984). The above-mentioned couplers may all be in the form of polymer couplers.

These compounds can typically be represented by the following general formula (M-1), (M-2) or (M-3):

In these formulae, R₃₁ represents a non-diffusive group having a total carbon number of from 8 to 32; R₃₂ represents a phenyl group or a substituted phenyl group. R₃₃ represents a hydrogen atom or a substituent. Z represents a non-metallic atomic group necessary for forming a 5-membered azole ring containing from 2 to 4 nitrogen atoms, and the azole ring may have substituent(s) including condensed ring(s). X₂ represents a hydrogen atom or a releasing group.

The details of the substituents for R₃₃ and the substituents for the azole ring are described in, for example, US-A-4,540,654, from column 2, line 41 to column 8, line 27.

Among the pyrazoloazole couplers, the imidazo[1,2-b]pyrazoles described in US-A-4,500,630 are preferred because of the small yellow side-absorption of the dye formed and the high light-fastness thereof. In particular, pyrazolo[1,5-b][1,2,4]triazoles described in US-A-4,540,654 are especially preferred.

In addition, pyrazolotriazole couplers where a branched alkyl group is directly bonded to the 2-, 3- or 6-position of the pyrazolotriazole ring described in JP-A-61-65245; pyrazoloazole couplers containing a sulfon-amido group in the molecule described in JP-A-61-65246; pyrazoloazole couplers having an alkoxyphenylsulfonamido ballast group described in JP-A-61-147254; and pyrazolotriazole couplers having an alkoxy group or an aryloxy group in the 6-position described in EP-B-226,849 are also preferably used in the present invention.

Typical cyan couplers for use in the present invention include phenol cyan couplers and naphthol cyan couplers.

Suitable phenol couplers include phenol compounds (including polymer couplers) having an acylamino group in the 2-position of the phenol nucleus and an alkyl group in the 5-position thereof described in US-A-2,369,929, US-A-4,518,687, US-A-4,511,647 and US-A-3,772,002. Typical examples of such compounds include the coupler of Example 2 of CA-A-625,822, compound (1) described in US-A-3,772,002, compounds (I-4) and (I-5) described in US-A-4,564,590, compounds (1), (2), (3) and (24) described in JP-A-61-39045, and compound (C-2) described in JP-A-62-70846.

Phenol cyan couplers include 2,5-diacylaminophenol couplers described in US-A-2,772,162, US-A-2,895,826, US-A-4,334,011 and US-A-4,500,653 and JP-A-59-164555. Specific examples of such couplers include compound (V) described in US-A-2,895,826, compound (17) described in US-A-4,557,999, compounds (2) and (12) described in US-A-4,565,777, compound (4) described in US-A-4,124,396 and compound (I-19) described in US-A-4,613,564.

Suitable phenol cyan couplers include condensed phenol couplers where a nitrogen-containing heterocyclic ring has been condensed to the phenol nucleus described in US-A-4,327,173, US-A-4,564,586 and US-A-4,430,423, JP-A-61-390441 and JP-A-62-257158. Specific examples of such couplers include couplers (1) and (3) described in US-A-4,327,173, compounds (3) and (16) described in US-A-4,564,586, compounds (1) and (3) described in US-A-4,430,423 and the following compounds .

Further phenol cyan couplers for use in the present invention include ureido couplers described in US-A-4,333,999, US-A-4,451,559, US-A-4,444,872, US-A-4,427,767 and US-A-4,579,813 and EP-B-067,689. Specific examples of such couplers include coupler (7) described in US-A-4,333,999, coupler (1) described in US-A-4,451,559, coupler (14) described in US-A-4,444,872, coupler (3) described in US-A-4,427,767, couplers (6) and (24) described in US-A-4,609,619, couplers (1) and (11) described in US-A-4,579,813, couplers (45) and (50) described in EP-B-067,689, and coupler (3) described in JP-A-61-42658.

Suitable naphthol cyan couplers for use in the present invention include naphthol compounds having an N-alkyl-N-arylcarbamoyl group at the 2-position of the naphthol nucleus (for example, those described in US-A-2,313,586), those having an alkylcarbamoyl group at the 2-position (for example, those described in US-A-2,474,293 and US-A-4,282,312), those having an arylcarbamoyl group at the 2-position (for example, those described in JP-B-50-14523), those having a carbonamido or sulfonamido group at the 5-position (for example, those described in JP-A-60-237448, JP-A-61-145557, JP-A-61-153640), those having an aryloxy-releasing group (for example, those described in US-A-3,476,563), those having a substituted alkoxy-releasing group (for example, those described in US-A-4,296,199), and those having a glycolic acid-releasing group (for example, those described in JP-B-60-39217).

Diphenylimidazole cyan couplers described in EP-A-0,249,453 can also be used in the present invention singly or in combination with the aforesaid cyan couplers.

Specific examples of the compounds are mentioned below.

The photographic material of the present invention can contain hydroquinone derivatives, aminophenol derivatives, gallic acid derivatives and ascorbic acid derivatives as color-fogging inhibitors.

In addition, they may also contain catechol derivatives, for example, those described in JP-A-59-125732 and JP-A-60-262159, as color image stabilizers.

The photographic material of the present invention can contain an ultraviolet absorbent in the hydrophilic colloid layer. For instance, aryl group-substituted benzotriazole compounds (for example, those described in US-A-3,533,794), 4-thiazolidone compounds (for example, those described in US-A-3,314,794 and US-A-3,352,681), benzophenone compounds (for example, those described in JP-A-46-2784), cinnamic acid ester compounds (for example, those described in US-A-3,705,805 and US-A-3,707,375), butadiene compounds (for example, those described in US-A-4,045,229) or benzoxidol compounds (for example, those described in US-A-3,700,455) can be used for this purpose. Ultraviolet-absorbing couplers (for example, α-naphthol cyan dye-forming couplers) and ultraviolet-absorbing polymers may also be used. The ultraviolet absorbent can be mordanted in a particular layer.

The color photographic material of the present invention preferably has plural layers of a subbing layer, at least three silver halide light-sensitive layers, an inter-layer, an ultraviolet absorbing layer and a protective layer, coated on the reflective support, and therefore the improved effect of the antihalation layer is noticeable.

On the other hand, in the multi-layered color photographic material of the present invention, the cationic polymer-containing layer can be provided without layer condition problems by forming the inter-layer (substantially not containing light-sensitive silver halide grains) adjacent to the polymer-containing layer. In particular, when the silver halide light-sensitive layer is combined with the cationic polymer-containing layer, an interlayer not containing light-sensitive silver halide grains is preferably provided between the two layers. The interlayer comprises a hydrophilic colloid which may contain a color mixing inhibiting agent, an ultraviolet absorbing agent, a coupler for preventing color mixing, a stain inhibiting agent, a polymer latex and/or a dye. The thickness of the interlayer is preferably from 0.1 »m to 3 »m, and more preferably from 0.1 »m to 2 »m.

The photographic material of the present invention can contain, if desired, various surfactants as coating aids, an emulsifying and dispersing agent or an anti-blocking agent to improve photographic properties (for example, acceleration of developability, elevation of contrast and elevation of sensitivity), for static charge prevention and for the improvement of slide properties.

For instance, such surfactants include non-ionic surfactants, for example, saponins (steroid type), alkyleneoxide derivatives (e.g., polyethylene glycol, polyethylene glycol/polypropylene glycol condensed product, polyethylene glycol alkylethers or polyethylene glycol alkylarylethers, polyethylene glycol esters, polyethylene glycol sorbitan esters, polyalkylene glycol alkylamides or amides, siliconepolyethyleneoxide adducts), glycidol derivatives (e.g., alkenylsuccinic acid polyglyceride, alkylphenol polyglyceride), fatty acid esters of polyhydric alcohols, and alkyl esters of saccharides; anionic surfactants containing an acid group such as a carboxyl, sulfo, phospho, sulfate or phosphate group, for example, alkylcarboxylic acid salts, alkylsulfonic acid salts, alkylbenzenesulfonic acid salts, alkylnaphthalenesulfonic acid salts, alkylsulfuric acid esters, alkylphosphoric acid esters, N-acyl-N-alkyltauric acids, sulfosuccinic acid esters, sulfoalkylpolyoxyethylene alkylphenylethers, polyoxyethylene alkylphosphoric acid esters; ampholytic surfactants, for example, amino acids, aminoalkylsulfonic acids, aminoalkylsulfuric acid esters or phosphoric acid esters, alkylbetaines, amineoxides; and cationic surfactants, for example, alkylamine salts, aliphatic or aromatic quaternary ammonium salts, heterocyclic quaternary ammonium salts such as pyridinium or imidazoliums, and aliphatic or heterocyclic phosphonium or sulfonium salts. Among these surfactants, polyoxyethylene surfactants and fluorine-containing surfactants are especially preferably used.

In particular, combinations of the cationic polymer dispersion used in the present invention and the above-mentioned cationic surfactants are effective for improving layer properties, film quality and adhesiveness to the adjacent layer.

The color photographic material of the present invention can contain various other additives. Additives which can be used in the present invention are described in Research Disclosure, Item 17643 (December, 1978) and Item 18716 (November, 1979). The relevant parts of the foregoing references are discussed below.

The present invention is suited for color photographic materials, especially printing color photographic materials.

A color developer is used for development of the photographic material of the present invention. The color developer for use in the present invention is preferably an alkaline aqueous solution comprising essentially an aromatic primary amine color developing agent. Preferably, color developing agents for the developer are phenylenediamine compounds, although aminophenol compounds are useful. Specific examples of the compounds include 3-methyl-4-amino-N,N-diethylaniline, 3-methyl-4-amino-N-ethyl-N-β-hydroxyethylaniline, 3-methyl-4-amino-N-ethyl-N-β-methanesulfonamidoethyl-aniline, 3-methyl-4-amino-N-ethyl-N-β-methoxyethylaniline and sulfates, hydrochlorides and p-toluenesulfonates thereof. Two or more of these compounds may be used in combination, in accordance with the object thereof.

"Scanning exposure system" as referred to herein means an image exposure performed by a scanning system. A "Scanning system" means a system of restructuring an image to be reproduced on a plane by combining image elements as resolved in accordance with a determined rule into a time-dependent sequence in accordance with a reversely determined rule. Details of the system are described in, for example, Image Electronics Handbook (edited by Image Electronics Association of Japan), Introduction, 3rd Chap., pages 45 to 55. A laser ray, CRT or LED (luminescence emitting diode) can be used for image exposure.

In accordance with the present invention, the use of a scanning exposure system by CRT is preferred

Preferably, the color photographic paper has at least three silver halide light-sensitive layers on a support, such as, the preferred reflection color photographic material, and the emitted wavelength of maximum strength from CRT is matched with the respective maximum wavelength of the different spectral sensitivities of each silver halide compound in the layers, in scanning exposure of the paper. For instance, at least three laser rays selected from e.g. He-Cd laser, Ar-gas laser, He-Ne gas laser and GaAs, GaAsxPrx and InP semiconductor lasers are preferably used. In scanning exposure, since the light emission of the respective image elements comprises repetition of light emission of from several ms to several »s, a sufficiently high quantity of light can be obtained from CRT of a relatively low output. The apparatus for the system is compact and inexpensive. In the present invention, a high quality color CRT and black-and-white CRT are advantageougly used. For example, a suitable CRT has a high resolving power, little strain, is able to obtain a picture on the whole fluorescent surface and has little spot halo. A black-and-white CRT which has a fluorescent body capable of emitting in blue, green and red wavelength ranges so as to elevate the density of the image elements, is especially preferred. In the system, image elements are inputted from a memory means of already inputted digital information, for example, a floppy disk, or are directly inputted without such means and the thus inputted information is displayed on a black-and-white CRT as photographic images, CG images, line images and/or character images, whereupon the images are formed on the surface of the light-sensitive layer of a color photographic paper via an optical lens and a shutter through blue, green and red filters in order.

Because of the necessity of short time exposure, the fluorescent body to be used is one which intensely emits fluorescent light under high voltage and high current density conditions and which has excellent current saturation characteristics and temperature stability. The fluorescent body can be selected from those used for projection tubes. Suitable industrially stable available fluorescent bodies which can be employed in the present invention include, Y₂O₃:Eu and Y₂O₂S:Eu for red, Zn₂SiO₄:Mn and Gd₂O₂S:Tb, in particular, Y₂SiGeO₅:Tb and Y₂Al₅O₁₂:Tb for blue, and ZnS:Ag and Cl or ZnS:Ag or Al for blue.

The exposure time for the respective blue image, green image and red image obtainable through the blue, green and red filters is inversely proportional to the spectral sensitivity of the respective light-sensitive layers of the color photographic paper by high-intensity and short-time multi-exposure. In accordance with the CRT to be applied to the method of the present invention, the number of image elements is generally from about (500 to 1000) × (500 to 1500), the emitting time for one image element is from about 1×10⁻³ to 1×10⁻⁷ s, and from 10 to 100 emissions are effected for one exposure to the respective light-sensitive layers. The beam diameter of the emission for one image element is from about 20 to 100 »m.

Exposure may also be effected by the use of the abovesaid FOT or CRT. In such case, a particular means for color separation between blue, green and red colors, for example, a liquid crystal filter can be used for contact exposure. Preferably the color photographic material is imagewise exposed by a combination of a black-and-white CRT exposure system and a photographic image exposure system as combined by light path changing-over switch means.

A flow sheet illustrating a process for forming prints by a CRT exposure system of the present invention is illustrated in Fig. 1.

Character image-inputting means (12) is composed of a console having a CRT and a keyboard. Character information is inputted by operating the keyboard and watching the CRT. The inputted character information can be memorized in a memory medium (for example, a floppy disk). Initiation of CRT exposure can be indicated by the means (12). Figure image-inputting means (13) comprises a digitizer, by which line images and computer graphics (CG) images can be inputted. The data of the inputted figure images can be memorized in a floppy disk. Initiation of CRT exposure can be indicated by means (13). In portrait image-inputting means (10), a photographic image may be exposed by a separate photographic image-exposing system, or alternatively, information or a photographic image inputted by an electronic steel camera can be inputted by means of a digitizer.

Picture-synthesizing means (11) is composed of a microcomputer, where the data is read out in a determined order from the portrait image-inputting means (10), character image-inputting means (12) and/or figure image-inputting means (13) and they are laid out in a determined position and are thereafter inputted into the CRT controller (14). The CRT controller (14) functions to control the color monitor (15) and the black-and-white CRT (16) for exposure. Before the initiation of exposure, the synthesized image data is outputted in only the color monitor (15) and a positive image is displayed on the display surface. In exposure, the synthesized image is reversed to a negative image and outputted to the black-and-white CRT (16). Then, electron beams are shifted to the direction opposite to the normal direction so that the synthesized image is reversed (turned right to left).

The black-and-white CRT image is inserted by synchronizing optical filters B, G and R with the emission on the black-and-white CRT display surface through optical lens (18), whereupon the filters are also synchronized with shutter (17). Accordingly, the color photographic paper (19) is printed for a determined period of time by a three-color face-ordered exposure system. Afterwards, the thus printed paper is subjected to a determined color development process through the photographic processing device (20).

Preferably, the fluorescent body used for the black-and-white CRT is one having a wavelength of maximum luminance which corresponds to the main wavelength of the spectral sensitivity of the respective three light-sensitive layers of the color photographic paper to be processed. Preferably, the fluorescent body also has a short afterimage time or has no afterimage and has a small flare on the display surface.

In accordance with the present invention, a CRT exposure system can be combined with a photographic exposure system to give synthesized images comprising photographic picture images and CG images, line images and character images. The luminous flux as emitted from image elements by the fluorescent body on the CRT surface is hardly focused. The color photographic paper to be employed in the system has plural light-sensitive layers on a reflective support, the layers each containing a dispersion of different couplers and silver halide grains. The degree of diffusion of the luminous flux to be emitted from the image elements of CRT frequently differs in the respective light-sensitive layers. Japanese letters have more edges and thinner lines than alphabet letters so that the reproduction of the former letters is generally difficult. Accordingly, a special means is required for elevating the resolving power and edge contrast and for inhibiting color bleeding in the edges of letters, in the reproduction of Japanese letters.

The color photographic paper according to the present invention has been improved with respect to the said requirements. The color photographic paper is therefore especially suited for use in cards and post cards.

When a post card is prepared from the printed image of the photographic paper according to the present invention, the paper preferably has a conventional support having a thickness of 220 »m or less. The post card print preferably has a weight of 6 g or less, a length of from 140 to 150 mm and a width of from 90 to 100 mm. Using the apparatus as described in, for example, JP-A-63-34545 and JP-A-63-70858 a print obtained from the color photographic paper according to the present invention is cut to have a weight of 6 g or less, and it is attached to a post card support with an adhesive. The thus attached sheet may be cut into a determined size for the post card.

A seal print may also be obtained from the color photographic paper according to the present invention, for example, in accordance with the techniques of Japanese Patent Application Nos. 61-231481 and 62-4765. The color photographic paper according to the present invention may also be processed into cards, in accordance with the technique described in, for example, JP-A-62-58248.

The color developer generally contains a pH buffer such as alkali metal carbonates, borates or phosphates, and development inhibitors or an anti-foggant such as bromides, iodides, benzimidazoles, benzothiazoles or mercapto compounds. In addition, the developer may further contain, if desired, various kinds of preservatives, such as hydroxylamine, diethylhydroxylamine, sulfates, hydrazines, hydrazides, phenylsemicarbazides, triethanolamine, catecholsulfonic acids, triethylenediamine (1,4-diazabicyclo[2,2,2]-octanes).

Above all, the use of hydrazines and hydrazides is preferred. These compounds correspond to those of the formula (II) described in Japanese Patent Application No. 63-11295. Specific examples thereof include the compounds shown in the same Application No. 62-11295, pages 27 to 47. The amount of the compound to be added is preferably from 0.01 to 50 g, especially from 0.1 to 30 g, per liter of developer. The amount of hydroxylamines to be added is preferably from 0 to 10 g, especially from 0 to 5 g, per liter of the developer. The amount of compound added is preferably small, provided that the stability of the color developer can be maintained.

Another compound may be added to the color developer for use in the present invention including ethylene glycol or diethylene glycol; a development accelerator such as benzyl alcohol, polyethylene glycol, quaternary ammonium salts or amines; dye-forming couplers; competing couplers; a foggant such as sodium boronhydride; an auxiliary developing agent such as 1-phenyl-3-pyrazolidone; a thickener; as well as various kinds of chelating agents such as aminopolycarboxylic acids, aminopolyphosphonic acids, alkylphosphonic acids or phosphonocarboxylic acids, e.g., ethylenediamine-tetraacetic acid, nitrilo-triacetic acid, diethylenetriamine-pentaacetic acid, cyclohexanediamine-tetraacetic acid, hydroxyethylimino-diacetic acid, 1-hydroxyethylidene-1,1-diphosphonic acid, nitrilo-N,N,N-trimethylenephosphonic acid, ethylenediamine-N,N,N′,N′-tetramethylenephosphonic acid, ethylenediamine-di(o-hydroxyphenylacetic acid) and salts thereof.

The processing temperature of the material of the present invention with the color developer is preferably from 30°C to 50°c, more preferably from 33°C to 42°C. The amount of the replenisher used in processing is 2000 ml or less, preferably 1500 ml or less, per m² of the photographic material being processed. The amount of the replenisher is preferably small in order to decrease the water liquid to be drained.

The photographic material of the present invention is preferably developed with a color developer substantially not containing benzyl alcohol. The inclusion of benzyl alcohol is disadvantageous since it causes environmental pollution, deterioration of storage stability of color images formed and increases staining of the material processed by a rapid development procedure. Thus, the color developing system preferably contains a restoring agent for the oxidation product of the color developing agent and a capturing agent for the oxidation product of the restoring agent, as described in JP-A-63-113537.

The color developer to be used for processing the photographic material of the present invention preferably does not substantially contain iodide ion. The "color developer substantially not containing iodide ion" means that the content of the iodide ion in the developer is less than 1 mg/l. The color developer for use in the present invention also preferably does not substantially contain sulfite ion. The "color developer substantially not containing a sulfite ion" means that the sulfite ion content in the developer is 0.02 mol/l or less.

The color developer generally has a pH value of from 9 to 12, preferably from 10 to 11. The amount of the replenisher to the developer is generally 3 l or less per m² of the material being processed. By lowering the bromide ion concentration in the replenisher, the amount may be 500 ml or lower. When the amount of the replenisher to be added is lowered, it is desirable to prevent the evaporation and aerial oxidation of the processing solution by reducing the contact surface area of the processing tank with air. In addition, the amount of the replenisher to be added may also be reduced by suppressing the accumulation of bromide ion in the developer.

After being color developed, the photographic emulsion layer is generally bleached. Bleaching may be carried out simultaneously with fixation (bleach-fixation) or separately from the latter. In order to accelerate the photographic processing, bleaching may be followed by bleach-fixation. In addition, bleach-fixation in two continuous processing tanks, fixation prior to bleach-fixation or bleaching followed by bleach-fixation may also be used to process the photographic material of the present invention, in accordance with the object thereof. Suitable bleaching agents include, for example, compounds of polyvalent metals such as iron (III), cobalt(III), chromium (VI) or copper(II), as well as peracids, quinones and nitro compounds. Specific examples of the bleaching agent include ferricyanides; bichromates; organic complexes of iron(III) or cobalt (III), for example, complexes with aminopolycarboxylic acids such as ethylenediaminetetraacetic acid, diethylenetriamine-pentaacetic acid, cyclohexanediamine-tetraacetic acid, methylimino-diacetic acid, 1,3-diaminopropane-tetraacetic acid or glycolether-diamine-tetraacetic acid, as well as with citric acid, tartaric acid or malic acid; persulfates; bromates; permanganates; and nitrobenzenes. Among them, aminopolycarboxylic acid iron(III) complexes such as ethylenediamine-tetraacetic acid/iron (III) complex as well as persulfates are preferred in view of the rapid processability thereof and of the prevention of environmental pollution. The aminopolycarboxylic acid/iron(III) complexes are especially useful both in a bleaching solution and in a bleach-fixing solution. The bleaching solution or bleach-fixing solution containing such bleaching agents generally has a pH value of from 5.5 to 8, but the solution may have a lower pH value for rapid processing.

Specific examples of advantageous bleaching accelerators for use in the present invention include compounds containing a mercapto group or a disulfide group such as those described in US-A-3,893,858, DE-B-1,290,812, JP-A-53-95630 and Research Disclosure, Item 17129 (July 1978); thiazolidine derivatives described in JP-A-50-140129; thiourea derivatives described in US-A-3,706,561; iodides described in JP-A-58-16235; polyoxyethylene compounds described in DE-B-2,748,430; and polyamine compounds described in JP-B-45-8836. Above all, mercapto group- or disulfide group-containing compounds are preferred as having sufficient accelerating effect, and in particular, the compounds described in US-A-3,893,858, DE-B-1,290,812 and JP-A-53-95630 are especially preferred. In addition, the compounds described in US-A-4,552,834 are also preferred. The bleaching accelerator can be incorporated into the photographic material. The bleaching accelerators are especially advantageously used for bleach-fixation of picture-taking color photographic materials.

Suitable fixing agents include thiosulfates, thiocyanates, thioether compounds, thioureas and a large amount of iodides. Among them, thiosulfates are generally used, and in particular, ammonium thiosulfate is most widely used. Preferred preservatives for the bleach-fixing solution include sulfites, bisulfites and carbonyl-bisulfite adducts.

The silver halide color photographic material of the present invention is generally rinsed with water and/or stabilized, after being desilvered. The amount of the water to be used in the rinsing step can be set in a broad range, in accordance with the characteristics of the photographic material being processed (for example, depending upon the raw material components, such as the coupler) or the use of the material, as well as the temperature of the rinsing water, the number of the rinsing tanks (the number of the rinsing stages), the replenishment system of normal current or countercurrent and other various kinds of conditions. Among these conditions, the relationship between the number of the rinsing tanks and the amount of the rinsing water in a multi-stage countercurrent rinsing system can be determined by the method described in Journal of the Society of Motion Picture and Television Engineers, Vol. 64, pages 248 to 253 (May, 1955).

According to the multi-stage countercurrent system described in the above-reference, the amount of the rinsing water to be used can be reduced noticeably, but because of the prolongation of the residence time of the water in the rinsing tank, bacteria would propagate in the tank so that the floating substances generated by the propagation of bacteria would adhere to the surface of the material as it was processed. The method of reducing calcium and magnesium ions, which is described in Japanese Patent Application No. 62-288838, can be effectively used for overcoming the foregoing problem during the processing the photographic material of the present invention. In addition, the isothiazolone compounds and thiabendazoles described in JP-A-57-8542; chlorine-containing bactericides such as chlorinated sodium isocyanurates; and benzotriazoles and other bactericides described in H. Horiguchi, Chemistry of Bactericidal and Fungicidal Agents, and Bactericidal and Fungicidal Techniques to Microorganisms, edited by Association of Sanitary Technique, Japan, and Encyclopedia of Bactericidal and Fungicidal Agents, edited by Nippon Bactericide and Fungicide Association, can also be used.

The pH value of the rinsing water to be used for processing the photographic material of the present invention is from 4 to 9, preferably from 5 to 8. The temperature of the rinsing water and the rinsing time can be variably set in accordance with the characteristics of the photographic material being processed as well as the use thereof. In general, the temperature is from 15 to 45°C and the time is from 20 s to 10 min, and preferably the temperature is from 25 to 40°C and the time is from 30 s to 5 min. Alternatively, the photographic material of the present invention may also be processed directly with a stabilizing solution in place of being rinsed with water. Suitable stabilization methods include, for example, those described in JP-A-57-8543, JP-A-58-14834 and JP-A-60-220345.

In addition, the material can also be stabilized, following the rinsing step. For example, a stabilizing bath containing formalin and a surfactant, can be used as a final bath for color photographic materials. The stabilizing bath may also contain various chelating agents and fungicides.

The overflow from the rinsing and/or stabilizing solutions because of addition of replenishers thereto may be re-used in the other steps such as the desilvering step.

The silver halide color photographic material of the present invention can contain a color developing agent for the purpose of simplifying and accelerating the processing of the material. For incorporation of color developing agents into the photographic material, various precursors of the agents are preferably used. For example, suitable precursors include the indoaniline compounds described in US-A-3,342,597, the Schiff base compounds described in US-A-3,342,599 and Research Disclosure Items 14850 and 15159, the aldole compounds described in Research Disclosure Item 13924, the metal complexes described in US-A-3,719,492 and the urethane compounds described in JP-A-53-135628.

The silver halide color photographic material of the present invention can contain various kinds of 1-phenyl-3-pyrazolidones, if desired, for the purpose of accelerating the color developability thereof. Specific examples of these compounds are described in JP-A-56-64339, JP-A-57-144547 and JP-A-58-115438.

The processing solutions for the photographic material of the invention are used at 10°C to 50°C. In general, a processing temperature of from 35°C to 38°C is standard, but the temperature may be made higher so as to accelerate the processing or to shorten the processing time, or on the contrary, the temperature may be made lower so as to improve the quality of images formed and to improve the stability of the processing solutions used. For the purpose of economization of silver in the photographic material, the cobalt intensification or hydrogen peroxide intensification described in DE-B-2,226,770 and US-A-3,674,499 may be employed in processing the photographic material of the present invention.

In order to optimize the excellent characteristics of the silver halide photographic material of the present invention, the materials are processed with a color developer which does not substantially contain benzyl alcohol and which contains bromide ion in an amount of 0.002 mol/l or less, within a development time of 2 min 30 s or less. The complete process from color development to drying via desilvering and rinsing can be effected within 120 s, in the photographic processing procedure for the preferred reflection color photographic material of the present invention.

The "color developer which does not substantially contain benzyl alcohol" means that it contains benzyl alcohol in an amount of 2 ml/l or less, preferably 0.5 ml/l or less, and most preferably, it contains no benzyl alcohol.

The following examples are intended to illustrate the present invention in more detail.

### EXAMPLE A-1

A waterproof titanium oxide-containing white pigment resin layer comprising the composition mentioned below was formed on the surface of a white raw paper made of 100% LBKP for photographic paper (hardwood, bleached sulfate pulp) (weight 175 g/m², thickness about 180 »m), to prepare supports (A) and (A-I) to (A-VI).

### Support (A):

10 parts by weight of titanium oxide white pigment were surface-treated with silicon oxide and aluminium oxide was added to 90 parts by weight of polyethylene composition (i) (density 0.920 g/ml melt index (MI) 5.0 g/10 min) and kneaded. The resulting blend was coated on the raw paper by melt-extrusion coating to form a 30 »m waterproof resin layer thereon. On the other hand, the back surface of the white raw paper was coated with only a polyethylene composition (ii) (density 0.950 g/ml, MI 8.0 g/10 min) to form a 20 »m waterproof resin layer thereon.

### Support A-I:

11 parts by weight of anatase-type titanium oxide white pigment (surface-treated as indicated in Table 1 below) were added to 89 parts by weight of the polyethylene composition (i) used in preparation of support (A) and blended analogously. The resulting blend was coated on the raw paper by melt-extrusion coating to form a 30 »m waterproof resin layer thereon.

The same titanium oxide powder as that used in the preparation of support (A) was dipped in an ethanol solution of 2,4-dihydroxy-2-methylpentane and then heated. After the evaporation of ethanol, a surface-treated titanium oxide white pigment was obtained. The alcohol adhered to the titanium oxide in an amount of about 1% by weight to coat the surface of the grains. The back surface of the white raw paper was coated with the same polyethylene composition (ii) as that used for the preparation of support (A) to form a waterproof resin layer thereon.

Supports (A-II) and (A-V) were prepared in the same manner as above, but using the compositions indicated in Table A-1 below.

### Support A-VI:

A composition comprising 50 parts by weight of dipentaerythritol propyleneoxide (12 mols)-hexaacrylate ester adduct and 50 parts by weight of rutile-type titanium oxide was blended and dispersed in a ball mill for 20 h or more and the resulting blend was coated and dried on the raw paper mentioned below in a dry film thickness of 20 »m. The raw paper used here was prepared by coating a 20 »m polyethylene composition layer on the same white raw paper as that used in the preparation of support (A), the back surface of the paper being coated with a 20 »m polyethylene layer (density 0.960 g/ml, MI 25 g/10 min).

The thus coated layer was treated by irradiation with an electron ray in an amount corresponding to an absorption dose of 5 M.rad under an accelerated voltage of 200 kV, to prepare support (A-VI).

The surface of the waterproof resin layer as coated on each of the supports thus prepared was etched to a depth of about 0.05 »m from the surface thereof by ion-sputtering, and the white pigment grains thus exposed were observed with an electron microscope so as to evaluate the degree of dispersion of the white pigment grains in the layer. The projected area ratio (Ri) of each grain was determined for the continuous six unit areas (each having a size of 6 »m x 6 »m), and the standard deviation (s) as well as the mean grain possessory area ratio (%) (R̅) were obtained from the following formulae:

The results are shown in Table A-1-a below.

As is obvious from the results in Table A-1-a, the degree of dispersion of white pigment in supports (A-I) to (A-VI) was superior to that in support (A). In particular, it is noted that the white pigment grains were substantially uniformly dispersed in supports (A-I), (A-VI) and (A-VI).

Each of supports (A) and (A-I) to (A-V) was subjected to corona discharge and a subbing layer (gelatin layer) was provided thereon. Next, a colored layer, silver halide light-sensitive layers, interlayers and a protective layer were formed on the support, as mentioned below. Color photographic paper samples (A-a) to (A-g) and (A-1) to (A-6) were thus prepared.

The numeral for the amount coated is expressed by the unit of g/m². The silver halide emulsion is expressed by the amount of silver therein.

### First Layer: Colored Layer

See Table A-3 below.

### Second Layer: Blue-sensitive Silver Halide Emulsion Layer

### Third Layer: Color Mixing Preventing Layer

### Fourth Layer: Green-sensitive Silver Halide Emulsion Layer

### Fifth Layer: Ultraviolet Absorbing Layer

### Sixth Layer: Red-sensitive Silver Halide Emulsion Layer

### Seventh Layer: Ultraviolet Absorbing Layer

### Eighth Layer: Protective Layer

The details of the silver halide emulsions used in preparing the above-mentioned samples are shown in Table 2 below.

The definition of the above-mentioned fluctuation coefficient and the method for determining the same are described in T.H. James, "The Theory of the Photographic Process", (published by Macmillan Company), 3rd Ed. (1966), page 39.

The compounds used in preparing the above-mentioned photographic material samples are mentioned below.

### (Sen-1) 6×10⁻⁴ mol/Ag-mol

### (Sen-2) 4×10⁻⁴ mol/Ag-mol

### (Sen-3) 8×10⁻⁴ mol/Ag-mol

### (Sen-4) 1.8×10⁻⁴ mol/Ag-mol

### (Sen-5) 3×10⁻⁴ mol/Ag-mol

(Solv-2) O = P(̵OC₉H₁₉(iso))₃

Each sample thus prepared was sensitometrically wedgewise exposed with a commercial sensitometer (color temperature in light source 3,200°K), using blue, green and red filters. On the other hand, each sample was exposed for determination of its resolving power (CTF) and then processed by the process mentioned below.

The density was obtained from the strip thus developed, and Dmin (minimum density in non-image area) was obtained. The whiteness was evaluated by visual observation and on the basis of Dmin (yellow) as obtained from the blue filter density. The results are shown in Table 4 below.

The photographic processing process employed here comprised the following steps:

The processing solutions used in the steps had the following compositions.

### Color Developer:

### Bleach-fixing Solution:

As is obvious from the results in Table 4, the color photographic paper samples (Samples (c) to (g) and Samples (1) to (7)) having the support according to the present invention have improved whiteness and resolving power, as compared with comparative samples having the conventional support. In addition, the color photographic paper samples (Samples (1) to (7)) having the colored layer according to the present invention have a synergetically improved resolving power. Above all, Sample (6) is noted to have a sufficient resolving power and an excellent whiteness, as it has a support containing a large amount of titanium oxide grains with a small fluctuation coefficient and it has a colored layer containing a cationic latex polymer having at least one hydrogen-having ammonium group at the cation site.

When ExC-2, ExC-3 or ExC-4 was used as the cyan coupler in place of ExC-1, the same results were obtained.

### EXAMPLE A-2

Samples (h) and (8) to (10) were prepared in the same manner as in Example 1, using supports (A), (A-I), (A-III) and (A-VI). The layer constitution of the samples was as follows. Unless otherwise specifically indicated, the amount coated is expressed by the unit of g/m². The silver halide is expressed by the amount of silver therein.

### First Layer: Blue-colored Layer

### Second Layer: Blue-sensitive Silver Halide Emulsion Layer

### Third Layer: Color Mixing Preventing Layer

### Fourth Layer: Green-sensitive Silver Halide Emulsion Layer

### Fifth Layer: Ultraviolet Absorbing Layer

### Sixth Layer: Interlayer

### Seventh Layer: Red-sensitive Silver Halide Emulsion Layer

### Eighth Layer: Ultraviolet Absorbing Layer

### Ninth Layer: Protective Layer

The additives used above were the same as those used in Example A-1, except for the following compounds.

The details of the silver halide emulsions used in preparing the above-mentioned samples are shown in Table A-5 below.

(Cpd-1) and (Cpd-9) used in Example 1 were added to the above-mentioned emulsions (EM-7) to (EM-9).

Each of these samples was wedgewise exposed for sensitometry and further exposed for determination of the resolving power, in the same manner as in Example A-1. In addition, color negative originals formed by photographing a person image, a Mackbeth Color Chart or a living flower on Fuji Color SUPER HR-100 were printed on each sample.

The samples were then processed by the rapid processing procedure mentioned below, and the density of the image formed was determined. The results are shown in Table A-6 below.

As is obvious from the results in Table A-6 above, the silver halide color photographic materials of the present invention (Samples 8 to 10) had improved image sharpness without lowering the degree of the whiteness thereof.

By observation of the characteristic curve of each sample processed, it is noted that Sample (10) had a lower Dmin than Sample (h) and the gradation of the toe was sharply cut and extended in the former Sample (10). By visual observation of the printed photograph, it is noted that the detail gradation of the highlight area was excellently reproduced in the samples of the present invention.

When a bluish colorant such as ultramarine is applied to the support according to the present invention, the apparent whiteness (visual whiteness degree) may be further strengthened.

The above-mentioned samples were processed by the following processing procedure.

(Stabilization was effected by a four-tank counter-current system from tank (4) to tank (1).)

Processing solutions used in the steps of the procedure had the following compositions.

### Color Developer:

### Bleach-Fixing Solution:

### Stabilizing Solution:

### EXAMPLE A-3

### Support A-VII (Acid Paper Support):

Wood pulp comprising 20 parts of LBSP (hard wood bleached sulfurous acid pulp) and 80 parts of LBKP (hard wood bleached sulfate pulp) was beaten with a disc refiner to a Canadian freeness of 300 ml. 1.0 part of sodium stearate, 1.0 part of anion polyacrylamide, 1.5 parts of aluminum sulfate and 0.5 part of polyamidepolyamine-epichlorohydrin were added thereto. (The "part" is by absolute dry weight to wood pulp.) The resulting mixture was made into a paper (weight: 180 g/m²) by the use of a Fourdrinier machine, whereupon polyvinyl alcohol (PVA) was added as a sizing agent in an amount of 1 g/m². The density of the paper made was adjusted to be 1.0 g/m² by the use of a machine calender. The paper made to have a pH value of 4.3.

The acid paper thus formed was used as a paper substrate, and a waterproof resin layer (25 »m thick) containing 15% by weight of trimethylolethane-surface-treated anatase-type titanium oxide was formed on the substrate in accordance with the method used to prepare the above-mentioned support (A-II), to prepare support (A-VII).

### Support A-VIII (Neutral Paper Support):

Wood pulp comprising 20 parts of LBSP and 80 parts of LBKP was beaten with a disc refiner to a Canadian freeness of 300 ml. Polyamide-polyamine-epichlorohydrin (fixing agent KYMENE 557, commercial product of DIC-HERCULES CHEMICALS Inc.) was added to the foregoing in an amount of 0.5% (by weight to absolute dry pulp - the same shall apply hereunder) and then cationic polyacrylamide (POLYSTRON 705, commercial product of Arakawa Chemical) and anionic polyacrylamide (POLYACRON ST-13, commercial product of Hamano Industries) each in an amount of 0.5% were added. Further, alkylketene dimer (AQUAPEL, commercial product of DIC-HERCULES CHEMICALS Inc.) was added thereto in an amount of 0.5%. The resulting mixture was made into a paper(weight: 180 g/m²) by the use of a Fourdrinier machine, whereupon PVA was added as a sizing agent in an amount of 1 g/m². The density of the paper was adjusted to be 1.0 g/cm³ by the use of a machine calender. The paper made to have a pH value of 5.5.

The neutral paper thus formed was used as a paper substrate, and a waterproof white pigment-containing resin layer was formed thereon by the same method used in preparing the above-mentioned support (A-VII).

Each of supports (A-VII) and (A-VIII) was subjected to corona discharge, and a colored layer having the composition mentioned below was formed thereon.

### Composition of Colored Layer (First Layer):

Next, the same second to ninth layers as those in Example A-2 were formed on the first layer and dried to prepare color photographic material Samples (11) and (12), where 1,2-bis(vinylsulfonyl)ethane was used as the hardening agent.

Each sample was cut into 12 cm wide strips and rolled. Each sample was then imagewise exposed and rolled, and the cut edge was rubbed under the same condition. Next, each sample was color-developed in the same manner as in Example A-2. Each rolled print thus obtained was stored for 5 days at 40°C, and the cut edge was observed to determine whether or not it was stained. (That is, the side edge of the rolled sample was visually observed and checked.) The results are shown in Table A-7 below.

Sample (i) was prepared as follows: Support (B) was prepared in the same manner as Support (A-VII), except that the same waterproof white pigment-containing resin layer as that used for preparing the above-mentioned Sample (A) was formed. Sample (i) was prepared in the same manner as Sample (11), except that Support (B) was used in place of Support (A-VII).

The results of Table A-7 above indicate that neutral paper is more advantageous than is acid paper as the support substrate for obtaining a higher degree of whiteness in the color photographic material of the present invention. From the results, therefore, it is presumed that the additives and sizing agent added to the support substrate as well as the pH value of the substrate have some influence on the degree of whiteness of the photographic material formed on the support.

The photographic material of the present invention gives photographic prints having excellent whiteness, image sharpness and highlight detail color tone reproducibility. In addition, the prints obtained from the photographic material of the present invention are hardly stained by photographic processing.

### Example A-4

Dispersion Method for Fine Grains of Dyes:

### Dispersion Method A

The dye crystal composition shown below was kneaded and ground by a sand mill.

Furthermore, the ground mixture was dispersed in 25 ml of an aqueous solution of 10% lime-processed gelatin containing 1 g of citric acid dissolved therein and sands used for the sand mill were removed using a glass filter. The dyes adsorbed to the sands on the glass filter were recovered by using warm water and added to the dispersion to provide 100 ml of the dispersion containing 7% gelatin with the addition of water.

Each of the supports as used in Example A-1 and Example A-3 was subjected to a corona discharging treatment, and after forming thereon a gelatin subbing layer, a first layer (colored layer) shown in Table A-8 below was formed and then the second layer to the ninth layer as in Example A-2 were formed thereon to provide Samples 13 to 16.

The cross section of a piece of Sample 13 was observed using a transmission type electron microscope. The mean grain size of the fine dye powder in Sample 13 was about 0.3 »m. Also, the fine dye powder existed in the first layer and was not observed in the adjacent layers.

According to the methods shown in Example A-1, each of the samples was subjected to the sensitometric stage exposure and the exposure for measuring the resolving power and then subjected to quick processing as shown in Example A-2. The occurrence of residual color and yellow stain in each sample was less than that of Samples 11 and 12 in Example 3. The results obtained are shown in Table A-9.

Also, when the samples having the subbing layer and the first layer only in Samples 13 to 16 were immersed in the color developer, it was observed that the dyes in the first layer were quickly (from about 15 s to 20 s) decolored and dissolved off.

### Example A-5

Each of the compositions of the dye crystals shown below was kneaded with a dispersion aid, ground by a ball mill, and the ground composition was dispersed in 25 ml of an aqueous solution of 10% lime-processed bone gelatin containing 1 g of citric acid dissolved therein. The beads used for grinding were removed from the mixture using a filter, the dyes adsorbed to the beads and the filter were recovered by warm water and added to the dispersion to provide 100 ml of the aqueous dispersion containing 7% gelatin.

### Dispersion Method B

### Dispersion Method C

### Dispersion Method D

### Dispersion Method E

The mean grain sizes of the fine crystal grains of the dyes in Dispersion Methods B, C, D and E were 0.1 »m, 0.3 »m, 0.15 »m, 0.2 »m, respectively. That is, the mean grain sizes were all 0.3 »m or less and haze was slight or absent.

Each of the first layers having the compositions shown in Table A-10 below was formed on each of the supports shown in Table A-10. In this example, Samples 17 and 18 each contained the dispersion of the fine dye grains according to this invention prepared by Dispersion Methods B and C, respectively. Furthermore, the second layer to the ninth layer as in Example A-2 were also formed thereon. In this case, however, the ninth layer of Sample 19 contained fine grains of Dye IV-24 formed by Dispersion Method D.

Each of the samples thus prepared was subjected to the sensitometric stage exposure and the exposure for measuring the resolving power as in Example A-2 and then subjected to quick color photographic processing as in Example A-2. The density of each sample thus processed was measured and the results obtained are shown in Table A-10 below.

As is clear from the results shown in the above table, Samples 17, 18, and 19 give less Dₘᵢₙ, give neither residual color nor stain, and are excellent in whiteness (visual observation) and resolving power as compared with other samples.

### Sensitization Test by Safelight

Two pieces of each of Samples 9, 16, 17, and 19 were subjected to a stage exposure (200 CMS, 0.1 s) through a sensitometric red filter and one of the two pieces of each sample was subjected to a sensitization test by safelight, another piece being used as a comparison contrast.

That is, a commercial Safelight Filter for color paper was mounted on an electric bulb of 10 W (100 V) and after irradiating one piece of each sample by the electric bulb in the direction perpendicular to the light-sensitive surface thereof for 20 min, the piece of the sample was subjected to color photographic processing together with another piece of the sample.

After processing, the density of each sample was measured and the increased density of each sample at the point of the image exposure amount corresponding to 0.5 in the reflection cyan image density of the contrast sample was compared with those of other samples and the results obtained are shown in Table A-11 below. The value is a measure of the resistivity to the safelight.

From the results shown in Table A-11 above, it can be seen that Sample 19 has a strong resistivity to safelight and gives low background density after processing.

### EXAMPLES B-1 to 7

For easy understanding of the total process of the methods as illustrated in the examples to follow, the steps constituting the process of each example are summarized in the following Table B-1.

In the following examples, reference is made to Table B-1 above.

A waterproof titanium oxide-containing white pigment resin layer comprising the composition mentioned below was formed on the surface of a white raw paper made of 100% LBKP for photographic paper (hardwood, bleached sulfate pulp) (weight 175 g/m², thickness about 180 »m), to prepare supports (B-I).

### Support (B-1):

10 parts by weight of titanium oxide white pigment were surface-treated with silicon oxide and aluminium oxide was added to 90 parts by weight of polyethylene composition (i) (density 0.920 g/ml, melt index (MI) 5.0 g/10 min) and kneaded. The resulting blend was coated on the raw paper by melt-extrusion coating to form a 30 »m waterproof resin layer thereon. On the other hand, the back surface of the white raw paper was coated with only a polyethylene composition (ii) (density 0.950 g/ml, MI 8.0 g/10 min) to form a 20 »m waterproof resin layer thereon.

### Support B-II:

15 parts by weight of anatase-type titanium oxide white pigment (surface-treated as indicated in Table 1 below) were added to 85 parts by weight of the polyethylene composition (i) used in preparation of support (B-I) and blended analogously. The resulting blend was coated on the raw paper by melt-extrusion coating to form a 30 »m waterproof resin layer thereon.

The same titanium oxide powder as that used in preparation of support (B-1) was dipped in an ethanol solution of 2,4-dihydroxy-2-methylpentane and then heated. After the evaporation of ethanol, a surface-treated titanium oxide white pigment was obtained. The alcohol adhered to the titanium oxide in an amount of about 1% by weight to coat the surface of the grains. The back surface of the white raw paper was coated with the same polyethylene composition (ii) as that used for the preparation of support (B-I) to form a waterproof resin layer thereon.

### Support B-III:

Support B-III was prepared in the same manner as support B-II, except that titanium oxide containing 3% by weight of zinc oxide was used in an amount of 12 parts by weight to 88 parts by weight of the polyethylene composition, in place of the anatase-type titanium oxide white pigment in support B-II.

### Support B-VI:

A composition comprising 50 parts by weight of dipentaerythritol propyleneoxide (12 mols)-hexaacrylate ester adduct and 50 parts by weight of rutile-type titanium oxide was blended and dispersed in a ball mill for 20 h or more and the resulting blend was coated and dried on the raw paper mentioned below in a dry film thickness of 20 »m. The raw paper used here was prepared by coating a 20 »m polyethylene composition layer on the same white raw paper as that used in preparation of support (B-I), the back surface of the paper being coated with a 20 »m polyethylene layer (density 0.960 g/ml, MI 25 g/10 min).

The thus coated layer was treated by irradiation with an electron ray in an amount corresponding to an absorption dose of 5 (M.rad) under an accelerated voltage of 200 kV, to prepare support (B-IV).

S/R̅ of each sample was determined in the same manner as in Example A-1 and shown in Table B-2.

As is obvious from the results in Table B-2, the degree of dispersion of the white pigment in support samples (B-II) to (B-VI) was superior to that in support sample (B-I). In particular, it is noted that the white pigment grains were substantially uniformly dispersed in samples (B-II), (B-III) and (B-IV).

Using supports (B-I) to (B-IV) color photographic paper samples (A) to (G) were prepared in the same manner as in Example A-1.

### First Layer: Colored Layer

See Table B-3 below, with reference to the item for the first layer as indicated in Table B-1 above.

The second to eighth layers include two kinds of (a) and (b) as indicated in Table B-1 above. Sample (a) is a silver bromide-rich material, and sample (b) is a silver chloride-rich material. The compositions of sample (a) and sample (b) are mentioned below.

### Sample (a):

The same as the second to eighth layer in Example A-1.

### Sample (b):

Following the above-mentioned sample (a), plural layers having the compositions mentioned below were formed on support (B-II) to prepare photographic material sample (E). Unless otherwise specifically indicated, the numeral for the amount coated is expressed by the unit g/m². The silver halide emulsion is expressed by the amount of silver therein.

### First Layer: Mordant Layer

### Second Layer: Blue-sensitive Silver Halide Emulsion Layer

### Third Layer: Color Mixing Preventing Layer

### Fourth Layer: Green-sensitive Silver Halide Emulsion Layer

### Fifth Layer: Ultraviolet Absorbing Layer

### Sixth Layer: Interlayer

### Seventh Layer: Red-sensitive Silver Halide Emulsion Layer

### Eighth Layer: Ultraviolet Absorbing Layer

### Ninth Layer: Protective Layer

The same additives as those used in the preparation of sample (a) were used for sample (b), except the compounds (Sen-6) and (Sen-7) which were as follows.

The details of the silver halide emulsions used in preparing sample (b) are shown in Table B-4 below.

(Cpd-1) and (Cpd-9) used in the preparation of sample (a) were added to the above-mentioned emulsions (EM-7) to (EM-9).

Processing conditions for processing (i) and (ii) indicated in Table 1 above are as follows.

### Processing (i):

The same as in Example A-1.

### Processing (ii):

Sample (E) as exposed in a commercial video printer was taken out therefrom before the development step, without being fogged with light, and processed in accordance with the following procedure.

(Stabilization was effected by a four-tank counter-current system from tank (4) to tank (1).)

The processing solutions used in the steps of the above-mentioned procedure had the following compositions.

### Color Developer:

### Bleach-fixing Solution:

### Stabilizing Solution:

The samples of Table B-1 were tested in accordance with the procedure mentioned below. Each of samples (A) to (G) was set in a commercial video printer and color name cards were prepared. The flow sheet of the equipment is same as that shown in Fig. 1. Precisely, a portrait image signal and a character image signal were introduced from the respective inputting means and these were outputted in the cathode ray tube (CRT) screen in the video printer and were printed to the sample through the lens system. All the samples thus printed, except sample (E), were developed, fixed and dried in the processing device as equipped in the machine, in accordance with the processing conditions mentioned above. The exposure time for each sample is shown in Table B-5 below. As the optinum exposure time varies for every sample, the exposure amount was varied in the level of high exposure, middle exposure and low exposure.

The sharpness of the thus finished samples (A) to (G) was evaluated by determining the density profile of the character as printed in each sample with a microdensitometer. The microdensitometer used was a reflection mode of a commercial FMP-S Type transmission-reflection microdensitometer. The measurement conditions were as follows. The objective lens had five magnifications. Fiber illumination with incident angle of 45 degrees was used. Two different filters each for visual ray and red ray were used. The size of the measurement slit was 10 »m × 100 »m. The object to be printed was a Japanese character of 13th degree Ming-style type. This was scanned in the position and direction as indicated in Fig. 2. From the density profile thus obtained, acutance "Ac" which will be explained hereunder is calculated out, and this was used as the value for evaluating the sharpness. "Ac" is defined as follows, for example, in accordance with the description of The Theory of the Photographic Process (by T.H. James) (published by the Macmillan Company), 4th Ed., 1967, page 602. In Fig. 7 "L" means the transition width of the stepwise image having a density difference "Ds". The transition width "L" is a criterion of the blurred degree of the edge of the image and is obtained from the mean density gradient G of the transition area, in accordance with the following formula:$\text{L =} \frac{\text{Ds}}{\text{G}}$
"Ac" is defined as follows:$\text{Ac =} \frac{\text{Ds}}{\text{L²}}$
Accordingly, the value "Ac" becomes higher when the blurred degree of "L" is smaller and the effective density difference "Ds" of image is larger.

The accurate definition of "Ac" is applied to the image where the hemi-planes of each of the low density side and the high density side are stepwise connected to each other. Although the character as examined in the present examples does not always satisfy the said condition, it could be interpreted that the definition of "Ac" as defined by formula (2) be applied to the both edges of the lines with a limited width of the character-constituting elements. Accordingly, since the actual "Ac" depends upon the line width, comparison between the characters with the same line width can be effected accurately.

In general, the resolving power and response function may be used as a criterion of sharpness, but the acutance as employed herein was the optimum function in the present case because of the following two reasons. The first is that the evaluation value can be expressed by one numeral. The second is that the acutance can be calculated by measuring the object itself to be examined, and printing of any other particular pattern for evaluation is unnecessary.

Samples (A) to (G) were thus evaluated, and the results obtained are shown in Table B-5 below.

The cyan couplers ExC-2, ExC-3 or ExC-4 were used in the preparation of samples (A) to (G) in place of ExC-1, and the same results were also obtained.

As is obvious from the results in Table B-5 above, samples (B) to (G) were superior to the comparative sample (A) with respect to the actuance (Ac). The actuance (Ac) somewhat differed in accordance with the exposure amount and in the parts of the image. The values shown in Table B-5 were mean values obtained in the optimum exposure range of the respective samples. That is, in the exposure range of giving "Ds" of from 1.5 to 2.5. The profiles of the third edge and that of the fifth edge of the character as shown in Fig. 2 were evaluated, and the mean values obtained were employed for the results in Table B-5.

As is noted from the results in Table B-5, "Ac" by the red filter was generally inferior to that by the visual filter. In particular, the difference therebetween in samples (A) to (C) and samples (D) to (G) was great. This may be because of the synergistic action of the exposure blur by so-called halation to be directed to the direction of the incident ray from the support and the blur caused by the light-scattering in viewing the finished print. The great difference means that the two blurs are especially great for red light. This could be understood from the fact that the red-sensitive layer is positioned in the uppermost layer which is most remote from the support in constituting the color light-sensitive layers of the present color photographic paper. In fact, sample (A) had noticeable bleeding of the cyan color around the character, while such bleeding was small in samples (B), (C), (D), (E), (F) and (G). Such bleeding could not be seen in samples (D) to (G).

### EXAMPLE B-8

Sample (E) of Example B-5 and Sample (F) of Example B-6 were prepared. Using a printer comprising a combination of the CRT exposure system of Fig. 1 and the portrait exposure system with light path switch-over means as described in JP-A-62-184446, a portrait was combined with Japanese characters. The characters were inputted from the character-inputting means and were displayed on the black-and-white CRT through the CRT controller, and printed on each of samples (E) and (F) to prepare a New Year's Card. The spectral sensitivity curve of sample (F) is shown in Fig. 4-a; and that of sample (E) in Fig. 4-b. In the black-and-white CRT in the CRT exposure system as used in the present example, a mixture of fluorescent substances of P-22R and P45 (code numbers of EIA; Electronic Industries Association) were used, and the relative emission strength is shown in Fig. 5. Fig. 6 shows spectral transmittance curves of B, G, R and Y filters used in the present example. After printing, sample (F) was developed with the developer (for processing (i) mentioned above) as filled in a commercial Video Printer. On the other hand, sample (E) was, after printing, developed with the processing solutions (for processing (ii) mentioned above) as filled in a modified Video Printer where the rack and other parts had been reformed so as to be suited for the processing (ii).

The thus obtained print having both portrait and characters was cut into a size of about 150 mm (length) × about 100 mm (width). An aqueous adhesive was applied to the back surface of the resulting print and this was attached to a postal card (as described in the Example of JP-A-63-104050). This was cut into a size of 145 m×98 mm to give a print-attached postcard having a dry weight of 5.8 g.

Sample (A) of Example B-1 was also processed in the same manner as Sample (F) to obtain a print-attached postcard. As compared with the postcard obtained from sample (A), those obtained from samples (F) and (E) exhibited excellent image quality of the character images. The latter postcards from samples (F) and (E) had a combination of a portrait photograph and character images which were comparable to the character images obtained by offset printing using lith film and a PS plate. These print-attached postcards from samples (F) and (E) had a high quality appearance.

In accordance with the method of the present invention, character-combined photograph prints can be provided, which have excellent image sharpness and excellent tone reproducibility of highlight details.

### EXAMPLE B-9

Dispersion method for Solid Fine Grains of Dyes:

### Dispersion Method A

The dye crystal composition shown below was kneaded and finely ground by a sand mill.

The ground composition was dispersed in 25 ml of an aqueous solution of 10% lime-processed gelatin containing 1 g of citric acid dissolved therein and sands used for grinding were removed using a glass filter. The dyes adsorbed to sands on the glass filter were recovered using warm water and added to the dispersion to provide 100 ml of the solid fine grain dispersion of the dyes containing 7% gelatin.

After applying a corona discharging treatment onto the support as Support B-II in Example B-3 and forming thereon a subbing layer, a colored layer was formed thereon using the aforesaid solid fine grain dispersion of the dyes as the first layer in Example B-2. In this case 2,4-dichloro-5-hydroxy-1,3,4-triazine sodium salt was used as a hardening agent.

The composition of the first layer was as follows.

The mean grain size of the solid fine grains of the dyes observed by a transmission type electron microscope (200 kV) was about 0.25 »m and aggregates having grain sizes of larger than about 3 »m were not observed.

Also, when the sample having the aforesaid colored layer was subjected to process (a) described in Example B-1, the colored layer formed was almost completely decolored.

Furthermore, the second layer to the eighth layer as in Examples B-2, B-4, and B-6 were formed thereon to provide Sample H. Sample H was subjected to the sensitometry as in Example B-2 and also the printing time for printing CRT images was determined using the aforesaid video printer as in Example 6 and the Ac value was determined as in Example B-6. The results obtained are shown in Table B-11 below.

It can be seen that Sample H shows the excellent Ac value as compared with Sample F at the same exposure time.

### EXAMPLES B-10 to 13

Using each of Supports B-I, B-II, and B-IV described above, the first layer (colored layer) containing the solid fine grain dispersion was formed using the solid fine grain dispersion of the dyes shown in Example B-9. Then, the second layer to the eighth layer of Sample (b) as in Example B-5 were formed thereon to provide Samples I, J, K and L, respectively.

Then, each sample was processed by Processing (ii) as shown in Example B-5, the exposure time for printing in the aforesaid video printer was determined as Example B-5 and the Ac value was determined as in Example B-5. The results obtained are shown in Table B-12 below.

In Samples I to L, the colored layers were almost completely decolored in spite of quick processing. Also, the colored layers have a tendency of giving the higher Ac value as compared with colored layers (1), (2) and (3).

Also, when the cross section of a piece of Sample J was observed by a transmission type electron microscope (200 KV), it was confirmed that the solid fine grain dispersion of the dyes was not diffused into the adjacent layers.

As described above, the method of the present invention can provide a silver halide photographic material capable of giving photographic prints having less stain by processing, having excellent whiteness, having excellent sharpness of images, and being excellent in tone reproducibility of details of the highlight.

### EXAMPLE C-1

A waterproof titanium oxide-containing white pigment resin layer comprising the composition mentioned below was formed on the surface of a white raw paper made of 100% LBKP for photographic paper (hardwood, bleached sulfate pulp) (weight 175 g/m², thickness about 180 »m), to prepare support (C-I).

### Support (C-1):

10 parts by weight of titanium oxide white pigment were surface-treated with silicon oxide, and aluminium oxide was added to 90 parts by weight of polyethylene composition (i) (density 0.920 g/ml, melt index (MI) 5.0 g/10 min) and kneaded. The resulting blend was coated on the raw paper by melt-extrusion coating to form a 30 »m waterproof resin layer thereon. On the other hand, the back surface of the white raw paper was coated with only a polyethylene composition (ii) (density 0.950 g/ml, MI 8.0 g/10 min) to form a 20 »m waterproof resin layer thereon.

### Support C-II:

12 parts by weight of anatase-type titanium oxide white pigment (surface-treated as indicated in Table C-1 below) were added to 88 parts by weight of the polyethylene composition (i) used in preparation of support (C-I) and blended analogously. The resulting blend was coated on the raw paper by melt-extrusion coating to form a 30 »m waterproof resin layer thereon.

The same titanium oxide powder as that used in preparation of support (C-I) was dipped in an ethanol solution of trimethylol ethane and then heated. After the evaporation of ethanol, a surface-treated titanium oxide white pigment was obtained. The alcohol adhered to the titanium oxide in an amount of about 1% by weight to coat the surface of the grains. The back surface of the white raw paper was coated with the same polyethylene composition (ii) as that used for the preparation of support (C-I) to form a waterproof resin layer thereon.

### Support C-III:

Support C-III was prepared in the same manner as support C-II, except that titanium oxide containing 3% by weight of zinc oxide was used in an amount of 12 parts by weight to 80 parts by weight of the polyethylene composition, in place of the anatase-type titanium oxide white pigment in support C-II.

### Support C-VI:

A composition comprising 50 parts by weight of dipentaerythritol propyleneoxide (12 mols)-hexaacrylate ester adduct and 50 parts by weight of rutile-type titanium oxide was blended and dispersed in a ball mill for 20 h or more and the resulting blend was coated and dried on the raw paper mentioned below in a dry film thickness of 20 »m. The raw paper used here was prepared by coating a 20 »m polyethylene composition layer on the same white raw paper as that used in preparation of support (C-I), the back surface of the paper being coated with a 20 »m polyethylene layer (density 0.960 g/ml, MI 25 g/10 min).

The thus coated layer was treated by irradiation with an electron ray in an amount corresponding to an absorption dose of 5 M.rad under an accelerated voltage of 200 kV, to prepare support (C-VI).

Supports (C-I), (C-II) and (C-III) contained ultramarine in an amount of about 0.3% by weight to the total of the polyethylene and white pigment grains; and support (C-IV) contained the same in an amount of about 0.15% by weight.

S/R̅ of each support was obtained in the same manner as described hereinbefore and the results are shown in Table C-1.

As is obvious from the results in Table C-1, the degree of dispersion of white pigment grains in each of Supports (C-II) to (C-IV) was superior to that in Support (C-I). In particular, it is noted that the grains were substantially uniformly dispersed in Supports (C-III) and (C-IV).

### EXAMPLE C-2

Silver halide emulsions (1) to (6) were prepared as mentioned below.

### (Solution-1)

### (Solution-2)

### (Solution-3)

### (Solution-4)

### (Solution-5)

### (Solution-6)

(Solution-1) was heated to 55°C, and (solution-2) was added thereto. Next, (solution-3) and (solution-4) were simultaneously added over a period of 10 min. After 10 min, (solution-5) and (solution-6) were simultaneously added over a period of 35 min. 5 min after completion of the addition, the temperature was lowered for desalting.

Water and gelatin for dispersion were added to the above-obtained resultant and the pH value was adjusted at 6.2. A monodispersed cubic silver chlorobromide emulsion (i) having a mean grain size of 0.70 »m and a fluctuation coefficient (value obtained by dividing the standard deviation by the mean grain size) of 0.13 was obtained.

Next, Ex DyeB( as CR-compound) was added to the emulsion (i) in an amount of 2.3×10⁻⁴ mol per mol of the silver halide at 58°C, and then sodium thiosulfate, chloroauric acid and ammonium rhodanide were added for optimum chemical sensitization for obtaining a surface latent image type emulsion. Afterwards, 4-hydroxy-6-methyl-1,3,3a,7-tetrazaindene (as stabilizer) was added. The resulting emulsion was called emulsion (1).

Emulsions (2) to (6) were prepared in the same manner as emulsion (1), whereupon the temperature for the grain formation and the CR-compound were varied as indicated in Table C-2 below. When silver bromide was added, the amount of the chloroauric acid was halved for effecting the optimum chemical sensitization.

Plural layers each having the composition mentioned below were formed on a paper support both surfaces of which were coated with polyethylene (support C-II) to prepare a multilayer color photographic paper sample.

The coating compositions were prepared by blending a silver halide emulsion, chemicals and a coupler-containing emulsion. The method of preparing the compositions is discussed below.

### Preparation of Coupler-Containing Emulsion:

27.2 ml of ethyl acetate and 7.7 ml of solvent (Solv-1) were added to 19.1 g of yellow coupler (Ex Y) and 4.4 g of color image stabilizer (Cpd-1). The resulting solution was dispersed by emulsification in 185 ml of an aqueous 10% gelatin solution containing 8 ml of 10% sodium dodecylbenzenesulfonate.

Other magenta, cyan and interlayer emulsions were prepared in the same manner.

Stabilizer (Ex-3d) was added to the blue-sensitive emulsion layer in an amount of 2.5×10⁻⁴ mol per mol of the silver halide.

The gelatin hardening agent used for each layer was 1-hydroxy-3,5-dichloro-s-triazine sodium salt.

Dyes (Ex-3a) and (Ex-3b) were added to the emulsion layers for anti-irradiation.

Further, compound (Ex-3c) was added to the red-sensitive emulsion layer in an amount of 2.6×10⁻³ mol per mol of the silver halide.

The coating compositions were coated on the support in accordance with the combinations as indicated in Table C-3 below. Samples (1), (2), (3) and (4) were thus obtained.

### Layer Constitution:

The compositions of the layers constituting each of samples (1) to (4) are mentioned below. The numeral indicates the amount coated by the unit g/m². The silver halide coated is expressed by the amount of silver therein.

### Support:

Polyethylene-Coated Paper (Support (C-II) (This contained white pigment (TiO₂) and bluish dye (ultramarine) in the polyethylene in the side coated with the first layer.)

### First Layer: Colored Layer

### Second Layer: Blue-sensitive Layer

### Third Layer: Color Mixing Preventing Agent

### Fourth layer: Green-sensitive Layer

### Fifth Layer: Ultraviolet Absorbing Layer

### Sixth Layer: Red-sensitive Layer

### Seventh layer: Ultraviolet Absorbing Layer

### Eighth Layer: Protective Layer

In order to examine the photographic characteristics of the thus prepared photographic material samples, the samples were subjected to the following tests.

First, each of the samples was sensitometrically wedgewise exposed with a commercial sensitometer (color temperature of light source 3200°K) through a green filter. The exposure time was 1/10 s, and the exposure amount was 250 CMS.

The thus exposed samples were processed for color development in accordance with the procedure mentioned below.

The processing solutions used in the steps were as follows.

### Color Developer:

### Bleach-fixing Solution:

The density of each of the thus processed photographic material samples (1) to (4) was determined, with red light, green light or blue light, and the relative sensitivity and fog of each light-sensitive layer were obtained. The results are shown in Table C-4 below.

As is obvious from the results in Table C-4, the relative sensitivity of sample (2) was noticeably lower than that of sample (1) because the anti-halation colored layer was provided on the support. In particular, B-sensitivity and G-sensitivity were relatively noticeably lowered. In sample (3), the sensitivity of the emulsions used was elevated and the fog thereof was suppressed, whereby the sensitivity of sample (3) was kept almost the same as that of sample (1) while the fog of sample (3) was also suppressed.

Sample (4) is noted to be superior to sample (1), as the blue-sensitivity, green-sensitivity and red-sensitivity were well balanced at a high level and the fog was suppressed.

For determination of the resolving power of each sample, a rectangular wave pattern for CTF determination was attached to the surface of each sample. Each sample was then exposed with the photometer. Subsequently, the thus exposed sample was processed as mentioned above, and the density of the processed sample was determined with a microdensitometer. The results obtained are shown in Table C-5 below.

As is obvious from the results in Table C-5, samples (3) and (4) are superior to sample (1) with respect to the resolving power.

Other samples were prepared, following samples (3) and (4), except that ExM2, ExM3 or ExM4 was used in place of ExM1 in the fourth layer, and ExC3, ExC4 or ExC5 was used in place of the blend of ExC1 and ExC2 in the sixth layer. These samples were also found to have the same properties.

In addition, ExDyeR in emulsion (6) was replaced by ExDyeR-1, and the same result was also obtained.

The compounds used in preparation of the above-mentioned samples are mentioned below.

### Yellow Coupler:

Magenta Couplers:

### Cyan Couplers:

### (Cpd-2): Color Image Stabilizer

### (Cpd-11): Color Mixing Preventing Agent

### (Cpd-4): Color Mixing Preventing Agent

### (Cpd-13): Color Image Stabilizer

(5/8/9 by weight mixture of the following compounds)

### (Cpd-12): Polymer

(mean molecular weight: 80,000)

### (UV-5): Ultraviolet Absorbent

(2/9/8 by weight mixture of the following compounds)

### (Solv-4): Solvent

### (Solv-2): Solvent

O=P(̵O-C₉H₁₉(ISO))₃

### (Solv-3): Solvent

### Compound Ex-3a:

### Compound Ex-3b

### Compound Ex-3c

### Compound Ex-3d

### Compound Ex-3e

### Compound Ex-3f

### ExDyeB

### (Cpd-14) Color Image Stabilizer:

### (Cpd-15) Color Image Stabilizer:

### (Solv-2) Solvent

(1/1 by volume mixture of the following compounds)

### EXAMPLE C-3

Using supports (C-I), (C-III) and (C-IV) in place of support (C-II), color photographic paper samples (5), (6) and (7) were prepared in the same manner as the photographic material of sample (3) prepared in Example C-1. These samples were subjected to the same sensitometry as that carried out in Example C-2. In addition, the same rectangular wave pattern for CTF determination used in Example C-2 was applied to the surface of each of samples (5), (6) and (7) and the resolving power of each sample was determined in the same manner as in Example C-2. The results obtained are shown in Table C-6 below.

The results in Table C-6 demonstrate that the color photographic paper samples (6) and (7) having support (C-III) and (C-IV), respectively are superior to sample (5) having support (C-I) with respect to the sensitivity and resolving power.

### EXAMPLE C-4

Emulsions (8) and (9) were prepared as follows: First, emulsion (i) was prepared in the same manner as in Example C-2, and the above-mentioned ExDyeR-1 (as CR-compound) was added thereto in an amount of 1.5×10⁻⁴ mol/mol-Ag at 42°C. Next, fine silver halide grains were added and heated and then sodium thiosulfate, chloroauric acid and ammonium rhodanide were added following the process of preparing emulsion (6) in Example C-2. Further, 10 mg/mol-Ag of the aforesaid thiosulfonyl group-containing compound (g) or 15 mg/mol-Ag of compound (i) were added for optimum chemical sensitization to obtain a surface latent-image type emulsion. Last, 4-hydroxy-6-methyl-1,3,3a,7-tetrazaindene and compound (Ex-3f) mentioned in Example C-3 were added to obtain emulsions (7) and (8).

Using emulsion (7) or emulsion (8) in place of emulsion (6) in sample (4) in Example C-2, sample (8) and sample (9) were prepared, respectively.

Samples (8) and (9) thus prepared were subjected to the same sensitometry as that in Example C-2. The results obtained are shown in Table C-7 below.

Samples (8) and (9) had the same resolving power as sample (4). As is obvious from the results in Table C-7, the red-sensitive layer (RL) containing the conpound having the thiosulfonyl group containing emulsion (7) or (8) had an extremely elevated sensitivity with noticeably lowered fog in samples (8) or (9), respectively.

### EXAMPLE C-5

Photographic material samples (1) to (4) prepared in Example C-2 and samples (8) and (9) prepared in Example C-4 were tested in accordance with the procedure mentioned below.

Each of the six kinds of samples was set in a commercial video printer and color name cards composed of a portrait image, a CG image and a character image were prepared. The flow sheet of the videoprinter is shown in Fig. 1. Precisely, the portrait image is displayed in the color monitor and the black-and-white CRT as digital information, while the CG image and the character image are synthesized in the image synthesizing means and are also displayed in the color monitor and the black-and-white CRT through the CRT controller. The yellow image, green image and red image as displayed in the black-and-white CRT were passed through the lens system and printed on the sample via the three color filters of (B+Y) filter, G filter and R filter which have the spectral transmittance as shown in Fig. 6 and which are synchronized with the color images. A blend of the fluorescent bodies (P-22R and P-45) which gave the spectral emission intensity as shown in Fig. 5 was used in the black-and-white CRT. The printing time for the respective blue, green and red lights were previously determined in accordance with the spectral sensitivity of BL, GL and RL of each sample. The printing time is shown in Table C-8 below.

It is noted from the results in Table C-8, that the printing time for samples (8) and (9) was reduced to 0.3 to 0.7 time of that for samples (1) to (4).

The image quality of the character images obtained from samples (2) to (4) and samples (8) and (9) was superior to that of the character images obtained from sample (1), especially with respect to the sharpness and the edge contrast.

Each of samples (3) and (4) was cut into a roll having a width of 102 mm. The resulting roll was charged in a printer equipped with CRT exposure system and photographic image exposure system, following the description of JP-A-62-184446. A portrait image was printed on the roll by a photographic image exposure system while character images were simultaneously printed thereon by a CRT exposure system.

Subsequently, the thus printed roll was passed through the photographic processing device to complete the color development mentioned in Example C-2, whereby a photographic print with written characters was obtained. This was cut to a size of 98 mm×148 mm to obtain a print for a postcard. The image quality of the character images printed was comparable to that obtained by conventional lithographic printing.

The thus prepared print was attached to a lottery postal card to form a print-attached lottery postal card, following the description of JP-A-63-70858.

### Example C-6

### Dispersion Method for Fine Grains of Dyes:

### Dispersion Method A

The dye crystal composition shown below was kneaded and finely ground by a sand mill.

Furthermore, the ground mixture was dispersed in 25 ml of an aqueous solution of 10% lime-processed gelatin containing 1 g of citric acid dissolved therein and sands used for the sand mill were removed using a glass filter. The dyes adsorbed to the sands on the glass filter were recovered using warm water and added to the dispersion to provide 100 ml of the solid fine grain dispersion of dyes containing 7% gelatin.

After applying a corona discharging treatment onto the support C-II as in Example C-2 and forming thereon a gelatin subbing layer, a colored layer was formed thereon the first layer having the composition shown below as in Example C-2. In this case, 2,4-dichloro-5-hydroxy-1,3,4-triazine sodium salt was used as a hardening agent.

### First Layer:

### Dispersion Method A

The mean grain size of the solid fine grains of the dyes by a transmission type electron microscopic observation was about 0.25 »m and aggregates of larger than about 3 »m were not observed.

When the sample was immersed in a color developer as used in Example C-2, the dyes were decolored within about 15 s and when the sample was immersed in a bleach-fixation solution as in Example C-2, decoloring was observed to a considerable extent.

Furthermore, the second layer to eighth layer as shown in Example C-2 were formed on the first layer of the sample to provide Sample 10. The sample was subjected to the sensitometric exposure and CTF measurement as Samples 1 to 4 in Example C-2 and the results obtained are shown in Table C-9.

From the results shown in Table C-9, it can be seen in the comparison with the results shown in Table C-4 and Table C-5 described above that the application of the solid fine grain dispersion method according to this invention gives a higher resolving power and lower fog.

### Example C-7

According to the Dispersion Method A shown in Example C-6, dye crystals shown in Table C-10 below and a dispersion aid were kneaded, the dye crystals were ground by a ball mill, and the ground crystals were dispersed in 25 ml of an aqueous solution of 10% lime-processed bone gelatin containing 1 g of citric acid dissolved therein. The beads used for grinding were removed by filtration, and the dyes adsorbed to the filter and the beads were recovered and added to the dispersion to provide 100 ml of the solid fine grain dispersion of dyes containing 7% gelatin.

On each of the supports Support C-III and C-IV in Example C-3 was formed a first layer using the aforesaid solid fine grain (fine crystal) dispersion prepared above. Furthermore, the second layer to the eighth layer as in Samples 6 and 7 in Example C-2 were formed thereon to provide Samples 11 to 15, respectively.

Each of the samples was subjected to the sensitometry and CTF measurement as in Example C-2. The results obtained are shown in Table C-10 below.

As is clear from the comparison of the results shown in Table 10 below with the results shown in Tables C-4 and C-5 in Example C-2 described above, the samples using the solid fine grain dispersions of the dyes according to this invention show less desensitization and give sufficiently high resolving power as compared with the samples (Samples 2 and 3) each having a colored layer using black colloid silver. In particular, it can be seen that in Sample 15, the color separation between the green-sensitive layer and the red-sensitive layer is improved and the resistivity to safelight is improved.

Then, the cross section of each piece of Samples 11 to 15 was observed by a transmission type electron microscope (200 kV). The solid fine crystal dispersion of the dyes contained in the colored layer (first layer) or the eighth layer was not diffused into adjacent layers and also aggregates having a mean grain size of larger than about 3 »m were not observed.

### Example C-8

By following the same procedure as in the preparation of Sample 11 in Example C-7 using the support C-III and the first layer (colored layer) as in Sample 11 and forming the second layer to the eighth layer as in Sample 9 in Example C-4, Sample 16 was prepared.

Sample 16 was subjected to the sensitometry as applied to Sample 9 in Examples C-4 and C-5 and also the printing times at blue light, green light, and red light were determined using a commercial video printer. The results obtained are shown in Table C-11 below.

As is clear from the results shown in Table C-11 above, the printing times for Sample 16 are the same as or faster than those for Sample 9. Also, the fog in Sample 16 was 0.08 less in the blue-sensitive layer, the green-sensitive layer, and the red-sensitive layer.

Using the preferred reflection color photographic material of the present invention, a color print having not only photographic picture images with excellent image sharpness but also line images and character images with high edge contrast can be obtained rapidly and easily. In particular, a so-called mini-laboratory system composed of a CRT exposure system printer and a photographic processing device can efficiently be used for processing the photographic material of the invention, and a print having not only photographic picture images with excellent image quality but also CG images, line images and/or character images with improved image sharpness can be formed easily in a short period of time of about 4 min or less. The photographic material of the invention is therefore especially convenient for forming printed postal cards.

## Claims

1. A color photographic material comprising: at least one silver halide light-sensitive layer provided on a reflective support containing white pigment grains in a waterproof resin layer, wherein said pigment grains are present in said waterproof resin layer in a density of from 10% by weight or more, and a colored layer which can be decolored by photographic processing located between said support and said silver halide light-sensitive layer, characterized in that the degree of dispersion of the white pigment grains in the layer is from 0.20 or less as the fluctuation coefficient (s/R̅) of the possessory area ratio (%) per unit area of 6 »m x 6 »m, where R̅ means the mean possessory area ratio per unit area and s means the standard deviation of the possessory area ratio per the unit area.

2. The color photographic material as in claim 1, wherein said waterproof resin layer is coated on a support base.

3. The color photographic material as in claim 2, wherein said support base is a neutral paper.

4. The color photographic material as in claim 1, wherein said white pigment grains are or are not surface-treated, and are fine grains selected from the group consisting of titanium oxide, barium sulfate, calcium sulfate, silicon oxide, zinc oxide, titanium phosphate and aluminium oxide.

5. The color photographic material as in claim 1, wherein said white pigment grains are present in the waterproof resin layer in a density of up to 60% by weight.

6. The color photographic material as in claim 1, wherein said white pigment grains are dispersed in the surface of the waterproof resin layer or in a thickness up to 10 »m from the surface of the layer.

7. The color photographic material as in claim 1, wherein said white pigment grains are incorporated into the waterproof resin layer in the presence of a surfactant to control the fluctuation coefficient of the possessory surface area of the grains.

8. The color photographic material as in claim 1, wherein said colored layer contains at least one of a dye and colloidal silver.

9. The color photographic material as in claim 1, wherein said colored layer contains a dye and a cationic polymer.

10. The color photographic material as in claim 9, wherein said cationic polymer is a non-coloring polymer having at least one hydrogen-containing ammonium base in the cation site which functions as an anion exchange polymer.

11. The color photographic material as in claim 10, wherein said cationic polymer is represented by formula (I): wherein A represents a monomer unit derived from copolymerization of a copolymerizable monomer having at least two copolymerizable ethylenically unsaturated groups, one of which is in the side chain moiety of the monomer; B represents a monomer unit derived from copolymerization of a copolymerizable ethylenically unsaturated monomer; R₁ represents a hydrogen atom, a lower alkyl group or an aralkyl group; Q represents a single bond or an alkylene group, an arylene group, an aralkylene group, L represents an alkylene group, an arylene group or an aralkylene group; R represents an alkyl group; G represents or R₂, R₃, R₄, R₅, R₆, R₇, R₈ and R₉ are the same or different and each represents a hydrogen atom, an alkyl group, an aryl group or an aralkyl group; X^{⊖} represents an anion; any two or more of Q, R₂, R₃, and R₄ or Q, R₅, R₆, R₇, R₈ and R₉ may be bonded to each other to form a ring structure together with the adjacent nitrogen atom; in the group of formula at least one of R₂, R₃, and R₄ must be a hydrogen atom; x, y and z each represent a molar percentage, and x is from 0 to 60, y is from 0 to 60 and z is from 30 to 100; and all said groups are or are not substituted and the following polymers:

12. The color photographic material as in claim 1, wherein said colored layer contains a solid grain dispersion of a dye which is insoluble in an aqueous solution having a pH of not higher than 7.0 to an extent capable of keeping the dispersed state in a hydrophilic colloid and soluble in an aqueous solution having a pH of at least 9.0

13. The color photographic material as in claim 12, wherein said dye is at least one dye selected from the group consisting of compounds shown by the following formulae (II), (III), (IV), (V) or (VI);
A₂ = L₁(̵L₂=L₃)̵ₙ A₂ (IV)
wherein A₂ (two A₂ groups being either the same or different) represents an acid nucleus having at least one substituent selected from a carboxyphenyl group, a sulfamoylphenyl group, a sulfonamidophenyl group, a carboxyalkyl group, and a hydroxyphenyl group (said acid nuclei may further have a substituent in addition to the aforesaid group), said acid nucleus being selected from 2-pyrazolin-5-one, rhodanine, hydantoin, thiohydantoin, 2,4-oxazolinedione, isoxazolinedinone, barbituric acid, thiobarbituric acid, indandione, and hydroxypyridone B₂ represents a basic nucleus having at least one substituent selected from a carboxy group, a sulfamoyl group, and a sulfonamido group (said basic nuclei may further have a substituent in addition to the aforesaid group), said basic nuclei being selected from pyridine, quinoline, indolenine, oxazole, benzoxazole, naphthoxazole, and pyrrole; R₄₀ represents a hydrogen atom or an alkyl group; R₄₁ and R₄₂ each represents a substituted or unsubstituted alkyl group, a substituted or unsubstituted aryl group, an acyl group, or a sulfonyl group, said R₄₁ and R₄₂ may combine with each other to form a 5- or 6-membered ring; R₄₃ and R₄₆ each represents a hydrogen atom, a hydroxy group, an alkyl group, an alkoxy group or a halogen atom; R₄₄ and R₄₅ each represents a hydrogen atom; or R₄₁ and R₄₄ or R₄₂ and R₄₅ form a non-metallic atomic group necessary for forming a 5- or 6-membered ring by the combination thereof; L₁, L₂, and L₃ each represents a substituted or unsubstituted methine group; X₃ and Y₃ each represents an electron attractive group, either X₃ or Y₃ having at least one carboxyphenyl group, sulfamoylphenyl group, sulfonamidophenyl group, carboxyalkyl group, or hydroxyphenyl group; m represents 0 or 1; n represents 0, 1, or 2; and p represents 0 or 1, when p is 0, said R₄₃ represents a hydroxy group or a carboxy group and said R₄₄ and R₄₅ represent a hydrogen atom and the following dyes:

14. The color photographic material as in claim 1, wherein said silver halide layer is the closest silver halide layer to the support.

15. The color photographic material as in claim 8, wherein the amount of the dye is from 1 to 500 mg/m².

16. The color photographic material as in claim 8, wherein the amount of the colloidal silver is from 0.01 to 0.5 g/m².

17. The color photographic material as in claim 1, wherein the thickness of the colored layer is from 0.1 to 10 »m.

18. The color photographic material as in claim 1, wherein the thickness of the waterproof resin layer is from 5 to 200 »m.

19. The color photographic material as in claim 1, wherein said silver halide light sensitive layer contains silver halide containing 15 mol% or more of silver chloride.

20. The color photographic material as in claim 1, wherein said silver halide light sensitive layer contains silver halide containing 98 mol% or more of silver chloride.

21. The color photographic material as in claim 1, wherein said silver halide light sensitive layer contains silver halide containing not more than 1 mol% of silver iodide.

22. The colour photographic material according to claim 1 wherein said colour photographic material is a reflection colour photographic material, the at least one silver halide light-sensitive layer contains a colour coupler, the waterproof resin layer is located on the side of the support coated with said silver halide light-sensitive layer, and said silver halide light-sensitive layer contains an emulsion of silver chlorobromide having a mean silver chloride content of 90 mol% or more and having a silver bromide-localized phase in the inside and/or surface of the emulsion grain.

23. The color photographic material as in claim 22, wherein the surface of the emulsion grain is gold-sensitized.

24. The color photographic material as in claim 22, wherein said reflective support contains white pigment grains in a waterproof resin layer in an amount of 12% by weight or more and the degree of dispersion of the white pigment grains is 0.15 or less as the fluctuation coefficient (s/R̅) of the projected possessory area ratio (%) per unit area of 6 »m x 6 »m, where R̅ means mean possessory area ratio per unit area and s means standard deviation of the possessory area ratio.

25. The color photographic material as in claim 23, wherein a compound having a thiosulfonyl group is added to said silver chlorobromide emulsion before, during or after gold-sensitization of the emulsion.

26. The color photographic material as in claim 22, wherein said silver halide light sensitive layer contains silver halide containing 98 mol% or more of silver chloride.

27. The color photographic material as in claim 22, wherein said silver halide light sensitive layer contains silver halide containing not more than 1 mol% of silver iodide.

28. A method of forming a color image, characterized in that the color photographic material as set forth in claim 1 or claim 22 is printed by a scanning exposure system and then subjected to color development processing.

29. A method of forming a color image comprising the step of:
imagewise exposing a color photographic material having at least one light-sensitive layer provided on a waterproof resin-containing reflective support by a scanning exposure system, wherein the reflective support contains white pigment grains in the waterproof resin layer located on the side coated with said light-sensitive layer in a density of 10% by weight or more, characterized in that the degree of dispersion of the white pigment grains in the waterproof resin layer is 0.20 or less as the fluctuation coefficient (s/R̅) of the projected possessory area ratio (%) per unit area of 6 »m x 6 »m, where R̅ means the mean. projected possessory area ratio per unit area and s means the standard deviation of the projected possessory area ratio per unit area.

30. The method of forming a color image as in claim 29, wherein said color photographic material comprises:
at least three kinds of silver halide light-sensitive layers each containing a color coupler selected from a cyan coupler, a magenta coupler and a yellow coupler, respectively, formed on said support; and
a colored layer which can be decolored during color development process and said colored layer is provided between the support and the silver halide light-sensitive layer unit.

31. The method of forming a color image as in claim 29, wherein image-exposure of the line original or character original is conducted by a CRT exposure system.

32. The method of forming a color image as in claim 29, wherein said color photographic material is imagewise exposed by a combination of a black-and-white CRT exposure system and a photographic image exposure system as combined by light path changing-over switch means.

33. The method of forming a color image as in claim 29, wherein said light-sensitive layer is a hydrophilic colloid layer containing silver halide grains forming a latent image mainly on the surface of the grain.

34. The method of forming a color image as in claim 29, wherein said light-sensitive layer is a hydrophilic colloid layer containing silver chloride or silver chlorobromide.

35. The method of forming a color image as in claim 29, wherein said silver halide light sensitive layer contains silver halide containing 15 mol% or more of silver chloride.

36. The method of forming a color image as in claim 29, wherein said silver halide light sensitive layer contains silver halide containing 98 mol% or more of silver chloride.

37. The method of forming a color image as in claim 29, wherein said silver halide light sensitive layer contains silver halide containing not more than 1 mol% of silver iodide.

38. The method of forming a color image as in claim 30, wherein said colored layer contains a dye.

39. The method of forming a color image as in claim 30, wherein said colored layer contains a solid dispersion of a dye which is insoluble in an aqueous solution to an extent capable of keeping the dispersed state in a hydrophilic colloid having a pH of not higher than 7.0 and soluble in an aqueous solution having a pH of at least 9.0.

## Patentansprüche

1. Farbphotographisches Material, das umfaßt mindestens eine lichtempfindliche Silberhalogenidschicht, die auf einem reflektierenden Träger angeordnet ist, der weiße pigmentkörnchen in einer wasserundurchlässigen Harzschicht enthält, wobei die pigmentkörnchen in der wasserundurchlässigen Harzschicht in einer Dichte von 10 Gew.-% oder mehr vorliegen, und eine gefärbte Schicht, die durch photographische Behandlung (Entwicklung) entfärbt werden kann, die zwischen dem Träger und der lichtempfindlichen Silberhalogenidschicht angeordnet ist,
dadurch gekennzeichnet, daß der Dispersionsgrad der weißen pigmentkörnchen in der Schicht 0,20 oder weniger beträgt, bestimmt als Fluktuations-Koeffizient (s/R̅) des possessorischen Flächenanteils (%) pro Einheitsfläche von 6 »m x 6 »m, worin R̅ für den mittleren possessorischen Flächenanteil pro Einheitsfläche und s für die Standardabweichung des possessorischen Flächenanteils pro Einheitsfläche stehen.

2. Farbphotographisches Material nach Anspruch 1, worin die wasserundurchlässige Harzschicht auf eine Trägerbasis aufgebracht ist.

3. Farbphotographisches Material nach Anspruch 2, worin die Trägerbasis ein neutrales Papier ist.

4. Farbphotographisches Material nach Anspruch 1, worin die weißen Pigmentkörnchen oberflächenbehandelt oder nicht oberflächenbehandelt und feine Körnchen sind, ausgewählt aus der Gruppe, die besteht aus Titanoxid, Bariumsulfat, Calciumsulfat, Siliciumoxid, Zinkoxid, Titanphosphat und Aluminiumoxid.

5. Farbphotographisches Material nach Anspruch 1, worin die weißen Pigmentkörnchen in der wasserundurchlässigen Harzschicht in einer Dichte von bis zu 60 Gew.-% vorliegen.

6. Farbphotographisches Material nach Anspruch 1, worin die weißen Pigmentkörnchen in der Oberfläche der wasserundurchlässigen Harzschicht oder in einer Dicke von bis zu 10 »m ab der Oberfläche der Schicht dispergiert sind.

7. Farbphotographisches Material nach Anspruch 1, worin die weißen Pigmentkörnchen der wasserundurchlässigen Harzschicht in Gegenwart eines oberflächenaktiven Agens einverleibt wurden, um den Fluktuationskoeffizient des possessorischen Oberflächenanteils der Körnchen zu kontrollieren (zu steuern).

8. Farbphotographisches Material nach Anspruch 1, worin die gefärbte Schicht mindestens einen Vertreter aus der Gruppe Farbstoff und kolloidales Silber enthält.

9. Farbphotographisches Material nach Anspruch 1, worin die gefärbte Schicht einen Farbstoff und ein kationisches Polymer enthält.

10. Farbphotographisches Material nach Anspruch 9, worin das kationische Polymer ein nicht-färbendes Polymer ist, das mindestens eine Wasserstoff enthaltende Ammoniumbase in dem Kationen-Anteil aufweist, die als Anionenaustausch-Polymer fungiert.

11. Farbphotographisches Material nach Anspruch 10, worin das kationische Polymer dargestellt wird durch die Formel (I) worin bedeuten:
A eine Monomereinheit, abgeleitet aus der Copolymerisation eines copolymerisierbaren Monomers, das mindestens zwei copolymerisierbare ethylenisch ungesättigte Gruppen aufweist, von denen eine in der Seitenketten-Gruppe des Monomers vorliegt;
B eine Monomereinheit, abgeleitet aus der Copolymerisation eines copolymerisierbaren ethylenisch ungesättigten Monomers;
R₁ ein Wasserstoffatom, eine niedere Alkylgruppe oder eine Aralkylgruppe;
Q eine Einfachbindung oder eine Alkylengruppe, eine Arylengruppe, eine Aralkylengruppe, worin L für eine Alkylengruppe, eine Arylengruppe, eine Aralkylengruppe und R für eine Alkylgruppe stehen;
G worin R₂, R₃, R₄, R₅, R₆, R₇, R₈ und R₉, die gleich oder verschieden sind, jeweils stehen für ein Wasserstoffatom, eine Alkylgruppe, eine Arylgruppe oder eine Aralkylgruppe und X^{⊖} ein Anion darstellt;
wobei jeweils zwei oder mehr der Reste Q, R₂, R₃ und R₄ oder Q, R₅, R₆, R₇, R₈ und R₉ miteinander verbunden sein können unter Bildung einer Ringstruktur zusammen mit dem benachbarten Stickstoffatom; wobei in der Gruppe der Formel mindestens einer der Reste R₂, R₃ und R₄ ein Wasserstoffatom sein muß; und
x, y und z jeweils einen Molprozentsatz, wobei x 0 bis 60 beträgt, y 0 bis 60 beträgt und z 30 bis 100 beträgt;
und wobei alle die genannten Gruppen substituiert oder unsubstituiert sind, und
die folgenden Polymeren:

12. Farbphotographisches Material nach Anspruch 1, worin die gefärbte Schicht eine Festkorn-Dispersion eines Farbstoffes enthält, der in einer wäßrigen Lösung mit einem pH-Wert von nicht höher als 7,0 bis zu einem solchen Grade unlöslich ist, daß der dispergierte Zustand in einem hydrophilen Kolloid aufrechterhalten werden kann, und der in einer wäßrigen Lösung mit einem pH-Wert von mindestens 9,0 löslich ist.

13. Farbphotographisches Material nach Anspruch 12, dadurch gekennzeichnet, daß der Farbstoff mindestens ein Farbstoff ist, der ausgewählt wird aus der Gruppe, die besteht aus Verbindungen der folgenden Formeln (II), (III), (IV), (V) oder (VI);
A₂ = L₁(̵L₂=L₃)̵ₙ A₂ (IV)
worin bedeuten:
A₂ (wobei zwei A₂-Gruppen gleich oder verschieden sind), einen sauren Kern (Ring) mit mindestens einem Substituenten, ausgewählt aus einer Carboxyphenylgruppe, einer Sulfamoylphenylgruppe, einer Sulfonamidophenylgruppe, einer Carboxyalkylgruppe und einer Hydroxyphenylgruppe (wobei die sauren Kerne(Ringe) außerdem einen weiteren Substituenten zusätzlich zu der obengenannten Gruppe aufweisen können), wobei der saure Kern(Ring) ausgewählt wird aus der Gruppe 2-Pyrazolin-5-on, Rhodanin, Hydantoin, Thiohydantoin, 2,4-Oxazolindion, Isoxazolindinon, Barbitursäure, Thiobarbitursäure, Indandion und Hydroxypyridon;
B₂ einen basischen Kern(Ring), der mindestens einen Substituenten aufweist, ausgewählt aus einer Carboxygruppe, einer Sulfamoylgruppe und einer Sulfonamidogruppe (wobei die basischen Kerne(Ringe) außerdem einen weiteren Substituenten zusätzlich zu der obengenannten Gruppe aufweisen können), wobei die basischen Kerne(Ringe) ausgewählt werden aus der Gruppe Pyridin, Chinolin, Indolenin, Oxazol, Benzoxazol, Naphthoxazol und Pyrrol;
R₄₀ ein Wasserstoffatom oder eine Alkylgruppe;
R₄₁ und R₄₂ jeweils eine substituierte oder unsubstituierte Alkylgruppe, eine substituierte oder unsubstituierte Arylgruppe, eine Acylgruppe oder eine Sulfonylgruppe, wobei R₄₁ und R₄₂ miteinander kombiniert sein können unter Bildung eines 5- oder 6-gliedrigen Ringes;
R₄₃ und R₄₆ jeweils ein Wasserstoffatom, eine Hydroxygruppe, eine Alkylgruppe, eine Alkoxygruppe oder ein Halogenatom;
R₄₄ und R₄₅ jeweils ein Wasserstoffatom; oder
R₄₁ und R₄₄ oder R₄₂ und R₄₅ eine Nicht-Metallatomgruppe bilden, die für die Bildung eines 5- oder 6-gliedrigen Ringes durch die Kombination derselben erforderlich ist;
L₁, L₂ und L₃ jeweils eine substituierte oder unsubstituierte Methingruppe;
X₃ und Y₃ jeweils eine Elektronen anziehende Gruppe, wobei entweder X₃ oder Y₃ mindestens eine Carboxyphenylgruppe, Sulfamoylphenylgruppe, Sulfonamidophenylgruppe, Carboxyalkylgruppe oder Hydroxyphenylgruppe aufweist;
m die Zahl 0 oder 1;
n die Zahl 0, 1 oder 2; und
p die Zahl 0 oder 1, wobei dann, wenn p = 0, R₄₃ eine Hydroxygruppe oder eine Carboxygruppe darstellt und R₄₄ und R₄₅ ein Wasserstoffatom und die folgenden Farbstoffe darstellen:

14. Farbphotographisches Material nach Anspruch 1, worin die Silberhalogenidschicht die dem Träger am nächsten angeordnete Silberhalogenidschicht ist.

15. Farbphotographisches Material nach Anspruch 8, worin die Menge des Farbstoffs 1 bis 500 mg/m² beträgt.

16. Farbphotographisches Material nach Anspruch 8, worin die Menge des kolloidalen Silbers 0,01 bis 0,5 g/m² beträgt.

17. Farbphotographisches Material nach Anspruch 1, worin die Dicke der gefärbten Schicht 0,1 bis 10 »m beträgt.

18. Farbphotographisches Material nach Anspruch 1, worin die Dicke der wasserundurchlässigen Harzschicht 5 bis 200 »m beträgt.

19. Farbphotographisches Material nach Anspruch 1, worin die lichtempfindliche Silberhalogenidemulsionsschicht ein Silberhalogenid enthält, das 15 Mol-% oder mehr Silberchlorid enthält.

20. Farbphotographisches Material nach Anspruch 1, worin die lichtempfindliche Silberhalogenidschicht ein Silberhalogenid enthält, das 98 Mol-% oder mehr Silberchlorid enthält.

21. Farbphotographisches Material nach Anspruch 1, worin die lichtempfindliche Silberhalogenidschicht ein Silberhalogenid enthält, die nicht mehr als 1 Mol-% Silberjodid enthält.

22. Farbphotographisches Material nach Anspruch 1, worin das farbphotographische Material ein farbphotographisches Reflexions-Material ist, bei dem mindestens eine lichtempfindliche Silberhalogenidschicht einen Farbkuppler enthält, die wasserundurchlässige Harzschicht auf der Seite des Trägers angeordnet ist, der mit der lichtempfindlichen Silberhalogenidschicht beschichtet ist, und die lichtempfindliche Silberhalogenidschicht eine Emulsion von Silberchloridbromid enthält, das einen mittleren Silberchloridgehalt von 90 Mol-% oder mehr und eine im Innern und/oder auf der Oberfläche des Emulsionskorns angeordnete Silberbromidphase aufweist.

23. Farbphotographisches Material nach Anspruch 22, worin die Oberfläche des Emulsionskorns goldsensibilisiert ist.

24. Farbphotographisches Material nach Anspruch 22, worin der reflektierende Träger weiße Pigmentkörnchen in einer wasserundurchlässigen Harzschicht in einer Menge von 12 Gew.-% oder mehr enthält und der Dispersionsgrad der weißen Pigmentkörnchen 0,15 oder weniger beträgt, bestimmt als Fluktuationskoeffizeint (s/R̅) des projizierten possessorischen Flächenanteils (%) pro Einheitsfläche von 6 »m x 6 »m, wobei R̅ für den mittleren possessorischen Flächenanteil pro Einheitsfläche und s für die Standardabweichung des possessorischen Flächenanteils stehen.

25. Farbphotographisches Material nach Anspruch 23, worin eine Verbindung, die eine Thiosulfonylgruppe aufweist, der Silberchloridbromidemulsion vor, während oder nach der Goldsensibilisierung der Emulsion zugesetzt worden ist.

26. Farbphotographisches Material nach Anspruch 22, worin die lichtempfindliche Silberhalogenidschicht ein Silberhalogenid enthält, das 98 Mol-% oder mehr Silberchlorid enthält.

27. Farbphotographisches Material nach Anspruch 22, worin die lichtempfindliche Silberhalogenidschicht ein Silberhalogenid enthält, das nicht mehr als 1 Mol-% Silberjodid enthält.

28. Verfahren zur Erzeugung eines Farbbildes, dadurch gekennzeichnet, daß das farbphotographische Material nach Anspruch 1 oder 22 vervielfältigt (kopiert) wird unter Verwendung eines Abtastbelichtungssystems und dann einer Farbentwicklungsbehandlung unterworfen wird.

29. Verfahren zur Erzeugung eines Farbbildes, das die Stufe umfaßt: bildmäßiges Belichten eines farbphotographischen Materials, das mindestens eine lichtempfindliche Schicht aufweist, die auf einem ein wasserdichtes Harz enthaltenden reflektierenden Träger vorgesehen ist, unter Verwendung eines Abtastbelichtungssystems, wobei der reflektierende Träger weiße Pigmentkörnchen in der wasserundurchlässigen Harzschicht, die auf der Seite angeordnet ist, die mit der lichtempfindlichen Schicht beschichtet ist, in einer Dichte von 10 Gew.-% oder mehr enthält, dadurch gekennzeichnet, daß der Dispersionsgrad der weißen Pigmentkörnchen in der wasserundurchlässigen Harzschicht 0,20 oder weniger beträgt, bestimmt als Fluktuations-Koeffizient (s/R̅) des projizierten possessorischen Flächenanteils (%) pro Einheitsfläche von 6 »m x 6 »m, worin R̅ für den mittleren projizierten possessorischen Flächenanteil pro Einheitsfläche und s für die Standardabweichung des projizierten possessorischen Flächenanteils pro Einheitsfläche stehen.

30. Verfahren zur Erzeugung eines Farbbildes nach Anspruch 29, worin das farbphotographische Material umfaßt:
mindestens drei Arten von lichtempfindlichen Silberhalogenidschichten, die jeweils einen Farbkuppler enthalten, ausgewählt aus einem Blaugrünkuppler, einem Purpurrotkuppler und einem Gelbkuppler, die auf dem Träger angeordnet sind, und
eine gefärbte Schicht, die während des Farbentwicklungsprozesses entfärbt werden kann und die zwischen dem Träger und der lichtempfindlichen Silberhalogenidschicht-Einheit angeordnet ist.

31. Verfahren zur Erzeugung eines Farbbildes nach Anspruch 29, worin die bildmäßige Belichtung eines Strich-Originals oder eines Zeichen (Buchstaben)-Originals unter Verwendung eines CRT-Belichtungssystems durchgeführt wird.

32. Verfahren zur Erzeugung eines Farbbildes nach Anspruch 29, worin das farbphotographische Material bildmäßig belichtet wird durch Verwendung einer Kombination aus einem Schwarz-Weiß-CRT-Belichtungssystem und einem photographischen Bild-Belichtungssystem in Kombination mit einer Lichtdurchgangs-Umschalteinrichtung.

33. Verfahren zur Erzeugung eines Farbbildes nach Anspruch 29, worin die lichtempfindliche Schicht eine hydrophile Kolloidschicht ist, die Silberhalogenidkörnchen enthält, die hauptsächlich auf der Oberfläche des Korns ein latentes Bild erzeugen.

34. Verfahren zur Erzeugung eines Farbbildes nach Anspruch 29, worin die lichtempfindliche Schicht eine hydrophile Kolloidschicht ist, die Silberchlorid oder Silberchloridbromid enthält.

35. Verfahren zur Erzeugung eines Farbbildes nach Anspruch 29, worin die lichtempfindliche Silberhalogenidschicht ein Silberhalogenid enthält, das 15 Mol-% oder mehr Silberchlorid enthält.

36. Verfahren zur Erzeugung eines Farbbildes nach Anspruch 29, worin die lichtempfindliche Silberhalogenidschicht ein Silberhalogenid enthält, das 98 Mol-% oder mehr Silberchlorid enthält.

37. Verfahren zur Erzeugung eines Farbbildes nach Anspruch 29, worin die lichtempfindliche Silberhalogenidschicht ein Silberhalogenid enthält, das nicht mehr als 1 Mol-% Silberjodid enthält.

38. Verfahren zur Erzeugung eines Farbbildes nach Anspruch 30, worin die gefärbte Schicht einen Farbstoff enthält.

39. Verfahren zur Erzeugung eines Farbbildes nach Anspruch 30, worin die gefärbte Schicht eine Feststoffdispersion eines Farbstoffes enthält, der in einer wäßrigen Lösung bis zu einem solchen Grad unlöslich ist, daß der dispergierte Zustand in einem hydrophilen Kolloid mit einem pH-Wert von nicht höher als 7,0 aufrechterhalten werden kann, und der in einer wäßrigen Lösung mit einem pH-Wert von mindestens 9,0 löslich ist.

## Revendications

1. Matériau photographique couleur comprenant : au moins une couche photosensible à l'halogénure d'argent disposée sur un support réfléchissant contenant des grains de pigment blanc dans une couche de résine imperméable à l'eau, dans laquelle lesdits grains de pigment sont présents dans ladite couche de résine imperméable à l'eau à une densité de 10 % en poids ou plus, et une couche colorée, qui peut être décolorée par traitement photographique, disposée entre ledit support et ladite couche photosensible à l'halogénure d'argent, caractérisé en ce que le degré de dispersion des grains de pigment blanc dans la couche est de 0,20 ou moins, exprimé par le coefficient de fluctuation (s/R̅) du rapport de surface occupée (%) rapporté à une surface unitaire de 6 »m x 6 »m, dans lequel R̅ représente le rapport de surface occupée moyen d'une surface unitaire et s représente l'écart-type du rapport de surface occupée par surface unitaire.

2. Matériau photographique couleur selon la revendication 1, dans lequel ladite couche de résine imperméable à l'eau est appliquée sur une base de support.

3. Matériau photographique couleur selon la revendication 2, dans lequel ladite base de support est un papier neutre.

4. Matériau photographique couleur selon la revendication 1, dans lequel lesdits grains de pigment blanc sont ou non traités en surface et sont des grains fins choisis parmi l'oxyde de titane, le sulfate de baryum, le sulfate de calcium, l'oxyde de silicium, l'oxyde de zinc, le phosphate de titane et l'oxyde d'aluminium.

5. Matériau photographique couleur selon la revendication 1, dans lequel lesdits grains de pigment blanc sont présents dans la couche de résine imperméable à l'eau jusqu'à une densité de 60 % en poids.

6. Matériau photographique couleur selon la revendication 1, dans lequel lesdits grains de pigment blanc sont dispersés dans la surface de la couche de résine imperméable à l'eau ou jusqu'à une épaisseur de 10 »m à partir de la surface de la couche.

7. Matériau photographique couleur selon la revendication 1, dans lequel lesdits grains de pigment blanc sont incorporés dans la couche de résine imperméable à l'eau en présence d'un tensioactif pour contrôler le coefficient de fluctuation de la surface occupée des grains.

8. Matériau photographique couleur selon la revendication 1, dans lequel ladite couche colorée contient au moins un colorant et/ou de l'argent colloïdal.

9. Matériau photographique couleur selon la revendication 1, dans lequel ladite couche colorée contient un colorant et un polymère cationique.

10. Matériau photographique couleur selon la revendication 9, dans lequel ledit polymère cationique est un polymère non colorant ayant au moins une base ammonium contenant de l'hydrogène dans un site cationique, qui agit comme polymère échangeur d'anions.

11. Matériau photographique couleur selon la revendication 10, dans lequel ledit polymère cationique est représenté par la formule (I) : dans laquelle A représente un motif monomère dérivé de la copolymérisation d'un monomère copolymérisable ayant au moins deux groupes éthyléniques insatures copolymérisables, dont l'un est dans le reste de chaîne latérale du monomère ; B représente un motif monomère dérivé de la copolymérisation d'un monomère éthylénique insature copolymérisable; R₁ représente un atome d'hydrogène, un groupe alkyle inférieur ou un groupe aralkyle, Q représente une liaison simple ou un groupe alkylène, un groupe arylène, un groupe aralkylène, L représente un groupe alkylène, un groupe arylène ou un groupe aralkylène ; R représente un groupe alkyle ; G représente R₂, R₃, R₄, R₅, R₆, R₇, R₈ et R₉ sont identiques ou différents et représentent chacun un atome d'hydrogène, un groupe alkyle, un groupe aryle ou un groupe aralkyle ; X^{⊖} représente un anion ; 2 quelconques ou plus des restes Q, R₂, R₃ et R₄ ou Q, R₅, R₆, R₇, R₈ et R₉ peuvent être reliés entre eux pour former une structure cyclique avec l'atome d'azote voisin;
dans le groupe de formule l'un au moins des restes R₂, R₃ et R₄ doit être un atome d'hydrogène ; x, y et z représentent chacun un pourcentage molaire et x est de 0 à 60, y est de 0 à 60 et z est de 30 à 100 ; et tous lesdits groupes sont substitués ou non
et les polymères suivants :

12. Matériau photographique couleur selon la revendication 1, dans lequel ladite couche colorée contient une dispersion de grains solides d'un colorant qui est insoluble dans une solution aqueuse ayant un pH de pas plus de 7,0 à un degré capable de maintenir l'état dispersé dans un milieu colloïdal hydrophile et soluble dans une solution aqueuse ayant un pH d'au moins 9,0.

13. Matériau photographique couleur selon la revendication 12, dans lequel ledit colorant est au moins un colorant choisi parmi les composés représentés par les formules (II), (III), (IV), (V) et (VI) suivantes :
A₂ = L₁ (̵L₂=L₃)̵ₙ A₂ (IV)
dans lesquelles A₂ (2 groupes A₂ pouvant être soit identiques ou soit différents) représente un noyau d'acide ayant au moins un substituant choisi parmi un groupe carboxyphényle, un groupe sulfamoylphényle, un groupe sulfonamidophényle, un groupe carboxyalkyle et un groupe hydroxyphényle (lesdits noyaux d'acides pouvant avoir encore un substituant en plus du groupe précité), ledit noyau d'acide étant choisi parmi la 2-pyrazoline-5-one, la rhodanine, l'hydantoïne, la thiohydantoïne, la 2,4-oxazolinedione, l'isoxazolinedinone, l'acide barbiturique, l'acide thiobarbiturique, l'indanedione et l'hydroxypyridone ; B₂ représente un noyau basique ayant au moins un substituant choisi parmi un groupe carboxyle, un groupe sulfamoyle et un groupe sulfonamido (lesdits noyaux basiques pouvant encore avoir un substituant en plus du groupe précité), lesdits noyaux basiques étant choisis parmi la pyridine, la quinoléine, l'indolénine, l'oxazole, le benzoxazole, le naphtoxazole et le pyrrole ; R₄₀ représente un atome d'hydrogène ou un groupe alkyle ; R₄₁ et R₄₂ représentent chacun un groupe alkyle substitué ou non, un groupe aryle substitué ou non, un groupe acyle ou un groupe sulfonyle, lesdits restes R₄₁ et R₄₂ pouvant se combiner l'un avec l'autre pour former un noyau à 5 ou 6 chaînons ; R₄₃ et R₄₆ représentent chacun un atome d'hydrogène, un groupe hydroxyle, un groupe alkyle, un groupe alcoxy ou un atome d'halogène ; R₄₄ et R₄₅ représentent chacun un atome d'hydrogène ; ou bien R₄₁ et R₄₄ ou R₄₂ et R₄₅ sont combinés en formant un groupe atomique non métallique nécessaire pour former un cycle à 5 ou 6 chaînons ; L₁, L₂ et L₃ représentent chacun un groupe méthine substitué ou non ; X₃ et Y₃ représentent chacun un groupe attracteur d'électrons, X₃ ou Y₃ ayant au moins un groupe carboxyphényle, un groupe sulfamoylphényle, un groupe sulfonamidophényle, un groupe carboxyalkyle ou un groupe hydroxyphényle ; m représente 0 ou 1 ; n représente 0, 1 ou 2 ; et p représente 0 ou 1 et lorsque p est égal à 0, ledit reste R₄₃ représente un groupe hydroxyle ou un groupe carboxyle et lesdits restes R₄₄ et R₄₅ représentent des atomes d'hydrogène
et les colorants suivants :

14. Matériau photographique couleur selon la revendication 1, dans lequel ladite couche à halogénure d'argent est la couche à halogénure d'argent la plus proche du support.

15. Matériau photographique couleur selon la revendication 8, dans lequel la quantité du colorant est de 1 à 500 mg/m².

16. Matériau photographique couleur selon la revendication 8, dans lequel la quantité d'argent colloïdal est de 0,01 à 0,5 g/m².

17. Matériau photographique couleur selon la revendication 1, dans lequel l'épaisseur de la couche colorée est de 0,1 à 10 »m.

18. Matériau photographique couleur selon la revendication 1, dans lequel l'épaisseur de la couche de résine imperméable à l'eau est de 5 à 200 »m.

19. Matériau photographique couleur selon la revendication 1, dans lequel ladite couche photosensible à l'halogénure d'argent contient un halogénure d'argent contenant 15 mol % ou plus de chlorure d'argent.

20. Matériau photographique couleur selon la revendication 1, dans lequel ladite couche photosensible à l'halogénure d'argent contient un halogénure d'argent contenant 98 mol % ou plus de chlorure d'argent.

21. Matériau photographique couleur selon la revendication 1, dans lequel ladite couche photosensible à l'halogénure d'argent contient un halogénure d'argent contenant pas plus de 1 mol % d'iodure d'argent.

22. Matériau photographique couleur selon la revendication 1, dans lequel ledit matériau photographique couleur est un matériau photographique couleur par réflexion, une couche photosensible à l'halogénure d'argent au moins contient un coupleur chromogène, la couche de résine imperméable à l'eau est située du côté du support revêtu avec ladite couche photosensible à l'halogénure d'argent, ladite couche photosensible à l'halogénure d'argent contient une émulsion de chlorobromure d'argent ayant une teneur moyenne en chlorure d'argent de 90 mol % ou plus et ayant une phase localisée de bromure d'argent à l'intérieur et/ou à la surface des grains d'émulsion.

23. Matériau photographique couleur selon la revendication 22, dans lequel la surface des grains d'émulsion est sensibilisée par l'or.

24. Matériau photographique couleur selon la revendication 22, dans lequel ledit support réfléchissant contient des grains de pigment blanc dans une couche de résine imperméable à l'eau en quantité de 12 % en poids ou plus et le degré de dispersion des grains de pigment blanc est de 0,15 ou moins, exprimé par le coefficient de fluctuation (s/R̅) du rapport de surface occupé projeté (%) rapporté à une surface unitaire de 6 »m x 6 »m, dans lequel R̅ représente le rapport de surface occupée moyen rapporté à la surface unitaire et s représente l'écart-type du rapport de surface occupée.

25. Matériau photographique couleur selon la revendication 23, dans lequel un composé ayant un groupe thiosulfonyle est ajouté à ladite émulsion de chlorobromure d'argent avant, pendant ou après la sensibilisation par l'or de l'émulsion.

26. Matériau photographique couleur selon la revendication 22, dans lequel ladite couche photosensible à l'halogénure d'argent contient un halogénure d'argent contenant 98 mol % ou plus de chlorure d'argent.

27. Matériau photographique couleur selon la revendication 22, dans lequel ladite couche photosensible à l'halogénure d'argent contient un halogénure d'argent contenant pas plus de 1 mol % d'iodure d'argent.

28. Procédé pour former une image en couleur, caractérisé en ce que le matériau photographique couleur selon la revendication 1 ou la revendication 22 est exposé par un système d'exposition par balayage et ensuite soumis à un traitement de développement chromogène.

29. Procédé de formation d'une image en couleur comprenant l'étape d'exposition suivant une image d'un matériau photographique couleur ayant au moins une couche photosensible disposée sur un support réfléchissant contenant une résine imperméable à l'eau par un système d'exposition par balayage, dans lequel le support réfléchissant contient des grains de pigment blanc dans la couche de résine imperméable à l'eau disposée du côté revêtu avec ladite couche photosensible jusqu'à une densité de 10 % en poids ou plus, caractérisé en ce que le degré de dispersion des grains de pigment blanc dans la couche de résine imperméable à l'eau est de 0,20 ou moins, exprimé par le coefficient de fluctuation (s/R̅) du rapport de surface occupée projetée (%) rapporté à une surface unitaire de 6 »m x 6 »m, dans lequel R̅ représente le rapport de surface occupée projetée moyen dans une surface unitaire et s représente l'écart-type du rapport de surface occupée projetée de la surface unitaire.

30. Procédé de formation d'une image en couleur selon la revendication 29, dans lequel ledit matériau photographique couleur comprend :
au moins trois types de couches photosensibles à l'halogénure d'argent contenant chacune un coupleur chromogène choisi parmi un coupleur pour cyan, un coupleur pour magenta et un coupleur pour jaune, respectivement, formées sur ledit support ; et
une couche colorée qui peut être décolorée pendant le procédé de développement chromogène, ladite couche colorée étant disposée entre le support et l'unité de couche photosensible à l'halogénure d'argent.

31. Procédé de formation d'une image en couleur selon la revendication 29, dans lequel l'exposition suivant une image du document au trait ou du document de caractères est effectuée par un système d'exposition par tube cathodique.

32. Procédé de formation d'une image en couleur selon la revendication 29, dans lequel ledit matériau photographique couleur est exposé suivant une image par une combinaison d'un système d'exposition en noir et blanc par tube cathodique et d'un système d'exposition d'une image photographique combinés par un dispositif à commutateur par commutation du trajet de la lumière.

33. Procédé de formation d'une image en couleur selon la revendication 29, dans lequel ladite couche photosensible est une couche colloïdale hydrophile contenant des grains d'halogénure d'argent formant une image latente principalement à la surface des grains.

34. Procédé de formation d'une image en couleur selon la revendication 29, dans lequel ladite couche photosensible est une couche colloïdale hydrophile contenant du chlorure d'argent ou du chlorobromure d'argent.

35. Procédé de formation d'une image en couleur selon la revendication 29, dans lequel ladite couche photosensible à l'halogénure d'argent contient un halogénure d'argent contenant 15 mol % ou plus de chlorure d'argent.

36. Procédé de formation d'une image en couleur selon la revendication 29, dans lequel ladite couche photosensible à l'halogénure d'argent contient un halogénure d'argent contenant 98 mol % ou plus de chlorure d'argent.

37. Procédé de formation d'une image en couleur selon la revendication 29, dans lequel ladite couche photosensible à l'halogénure d'argent contient un halogénure d'argent contenant pas plus de 1 mol % d'iodure d'argent.

38. Procédé de formation d'une image en couleur selon la revendication 30, dans lequel ladite couche colorée contient un colorant.

39. Procédé de formation d'une image en couleur selon la revendication 30, dans lequel ladite couche colorée contient une dispersion solide d'un colorant qui est insoluble dans une solution aqueuse à un degré capable de maintenir l'état dispersé dans un milicu colloïdal hydrophile ayant un pH de pas plus de 7,0 et soluble dans une solution aqueuse ayant un pH d'au moins 9,0.
